



US009523936B2

(12) **United States Patent**  
**Abe et al.**

(10) **Patent No.:** **US 9,523,936 B2**  
(45) **Date of Patent:** **\*Dec. 20, 2016**

(54) **TONER**(71) Applicant: **CANON KABUSHIKI KAISHA**,  
Tokyo (JP)(72) Inventors: **Koji Abe**, Numazu (JP); **Naoya Isono**,  
Suntou-gun (JP); **Taiji Katsura**,  
Suntou-gun (JP); **Yuhei Terui**, Numazu  
(JP); **Katsuyuki Nonaka**, Mishima (JP)(73) Assignee: **Canon Kabushiki Kaisha**, Tokyo (JP)(\* ) Notice: Subject to any disclaimer, the term of this  
patent is extended or adjusted under 35  
U.S.C. 154(b) by 0 days.This patent is subject to a terminal dis-  
claimer.(21) Appl. No.: **14/141,260**(22) Filed: **Dec. 26, 2013**(65) **Prior Publication Data**

US 2014/0186761 A1 Jul. 3, 2014

(30) **Foreign Application Priority Data**

Dec. 28, 2012 (JP) ..... 2012-288227

(51) **Int. Cl.**

**G03G 9/093** (2006.01)  
**G03G 9/08** (2006.01)  
**G03G 9/087** (2006.01)  
**G03G 9/097** (2006.01)

(52) **U.S. Cl.**

CPC ..... **G03G 9/09321** (2013.01); **G03G 9/0825**  
(2013.01); **G03G 9/08773** (2013.01); **G03G  
9/09328** (2013.01); **G03G 9/09392** (2013.01);  
**G03G 9/09775** (2013.01)

(58) **Field of Classification Search**CPC ..... G03G 9/09321; G03G 9/09328; G03G  
9/09392; G03G 9/09775; G03G 9/0825USPC ..... 430/110.2, 108.3  
See application file for complete search history.

(56)

**References Cited****U.S. PATENT DOCUMENTS**

|                 |         |                                     |
|-----------------|---------|-------------------------------------|
| 6,358,658 B1    | 3/2002  | Tazawa et al.                       |
| 7,829,254 B2 *  | 11/2010 | Kurose ..... G03G 9/0825<br>399/252 |
| 8,980,517 B2 *  | 3/2015  | Kawaguchi et al. ..... 430/110.2    |
| 2006/0292477 A1 | 12/2006 | Daimon                              |
| 2010/0075245 A1 | 3/2010  | Watanabe                            |
| 2010/0159375 A1 | 6/2010  | Zhou et al.                         |

(Continued)

**FOREIGN PATENT DOCUMENTS**

|    |              |        |
|----|--------------|--------|
| EP | 1003080 A1   | 5/2000 |
| JP | S57-124740 A | 8/1982 |

(Continued)

**OTHER PUBLICATIONS**

U.S. Appl. No. 14/141,241, filed Dec. 26, 2013, Kawaguchi.

*Primary Examiner* — Janis L Dote(74) *Attorney, Agent, or Firm* — Canon U.S.A., Inc., IP  
Division(57) **ABSTRACT**

A toner having good development durability, storage stability, environmental stability, and low-temperature fixability is provided. The toner contains toner particles each including a surface layer that contains an organic silicon polymer. The organic silicon polymer contains a specific unit. In a chart obtained by  $^{29}\text{Si-NMR}$  measurement of THF insoluble components of the toner particles, the ratio of a peak area attributable to a specific structure to the total peak area of the organic silicon polymer is 0.40 or more.

**7 Claims, 4 Drawing Sheets**

(56)

**References Cited**

U.S. PATENT DOCUMENTS

2010/0159376 A1 6/2010 Zhou et al.

FOREIGN PATENT DOCUMENTS

|    |             |   |         |
|----|-------------|---|---------|
| JP | 03-089361   | A | 4/1991  |
| JP | H08-095284  | A | 4/1996  |
| JP | 09-179341   | A | 7/1997  |
| JP | 2000-297106 | A | 10/2000 |
| JP | 2001-75304  | A | 3/2001  |
| JP | 2001-330996 | A | 11/2001 |
| JP | 2004-053916 | A | 2/2004  |
| JP | 2006-146056 | A | 6/2006  |
| JP | 2007-279712 | A | 10/2007 |

\* cited by examiner

FIG. 1



FIG. 2



FIG. 3



FIG. 4



**1**  
**TONER**

BACKGROUND OF THE INVENTION

1. Field of the Invention

The present invention relates to a toner for developing electrostatic latent images used in image forming methods such as electrophotographic methods and electrostatic printing methods.

2. Description of the Related Art

As computers and multimedia become more advanced, there arises an increasing need to develop ways to output high-definition full color images that satisfy various needs in homes and offices.

In offices where large quantities of copies and printouts are made, image forming apparatuses desirably have high durability whereby degradation of image quality is suppressed even when a large number of copies and printouts are made. In contrast, in small offices and homes, image forming apparatuses are desirably capable of producing high-quality images and are desirably small to save space and energy and reduce weight. To satisfy these needs, toners used therein desirably have improved properties, such as environmental stability, low-temperature fixability, development durability, and storage stability, and a lower tendency to soil parts of apparatuses (hereinafter this tendency is referred to as "non-soiling property").

In particular, a full color image is formed by superimposing color toners. Unless all of the color toners are developed equally, the color reproducibility is degraded and color nonuniformity is generated. If a pigment or a dye used as a colorant of a toner is precipitated on the surfaces of toner particles, the developing performance is affected and color nonuniformity may result.

In forming a full color image, fixability and color mixing property during fixing are important. For example, in order to achieve high-speed image formation, a binder resin suitable for low temperature fixing is selected. The influence of this binder resin on the developing performance and durability is also large.

Moreover, devices, mechanisms, etc., configured to output high-definition full color images and withstand long-term use in various environments that involve wide ranges of temperature and humidity are also in demand. In order to meet such a need, several challenges are desirably addressed, such as suppressing changes in the toner surface properties and changes in the charge amount of toners caused by changes in the operation environment and minimizing soiling of parts such as a developing roller, a charging roller, a regulating blade, and a photosensitive drum. In this respect, development of a toner that exhibits stable chargeability despite being stored in a wide variety of environments for a long time and has stable development durability that does not cause soiling of parts has been eagerly anticipated.

One of the causes of changes in charge amount and storage stability of the toner due to temperature and humidity is a phenomenon called bleeding in which a release agent and a resin component in the toner ooze out from the interior of the toner particle to the surface of the toner particle, thereby altering the surface properties of the toner.

One way to address this challenge is to cover the surface of a toner particle with a resin.

Japanese Patent Laid-Open No. 2006-146056 discloses a toner that has good high-temperature storage stability and exhibits good printing durability when printing is conducted in a normal temperature, normal humidity environment or a

**2**

high temperature, high humidity environment. This toner includes inorganic fine particles strongly fixed to toner particle surfaces. However, even if inorganic fine particles are strongly fixed to toner particles, bleeding of a release agent and a resin component occurs through gaps between the inorganic fine particles and the inorganic fine particles may detach due to deterioration of durability. Accordingly, the durability in a severe environment is desirably further improved and the problem of soiling of parts is desirably addressed.

Japanese Patent Laid-Open No. 03-089361 discloses a method for producing a polymerized toner, in which a silane coupling agent is added to the reaction system to try to prevent colorants and polar substances from becoming exposed in the toner particle surfaces and to obtain a toner that has a narrow charge amount distribution and very low dependence of charge amount on humidity. However, according to this method, the amount of precipitates of the silane compounds on the toner particle surfaces and hydrolytic polycondensation are insufficient. The environmental stability and the development durability are desirably further improved.

Japanese Patent Laid-Open No. 09-179341 discloses a polymerized toner that contains a silicon compound in a form of a continuous thin film on a surface portion. With this toner, the charge amount can be controlled and high quality images can be printed irrespective of the temperature and humidity in the environment. However, the polarity of organic functional groups is high, hydrolytic polycondensation and the amount of precipitates of the silane compound on the toner particle surfaces are insufficient, and the degree of crosslinking is low. Accordingly, further improvements are desired regarding the soiling of parts caused by deterioration of durability and changes in image density due to changes in chargeability in a high temperature, high humidity environment.

Japanese Patent Laid-Open No. 2001-75304 discloses a toner that improves fluidity, low temperature fixability, and blocking property and suppresses detachment of a fluidizer. This toner is a polymerized toner that includes a coating layer in which granular lumps containing a silicon compound are fixed to each other. However, bleeding of a release agent and a resin component occurs through gaps between the granular lumps containing a silicon compound. The image density changes due to changes in chargeability in a high temperature, high humidity environment due to insufficient hydrolytic polycondensation and an insufficient amount of silane compound precipitates on the toner particle surfaces. Moreover, parts become soiled by toner fusion. These problems are desirably addressed and the storage stability is desirably further improved.

SUMMARY OF THE INVENTION

The present invention provides a toner that addresses challenges described above. In particular, the present invention provides a toner having good development durability, storage stability, environmental stability, and low-temperature fixability.

The inventors of the present invention have conducted extensive studies and made the present invention based on the findings.

The present invention provides a toner that includes toner particles each including a surface layer that contains an organic silicon polymer, the organic silicon polymer including a unit represented by formula (1) or (2) below:



(In formula (2), L represents a methylene group, an ethylene group, or a phenylene group).

In a chart obtained by  $^{29}\text{Si}$ -NMR measurement of THF insoluble components of the toner particles, a ratio SQ3 of a peak area attributable to a structure represented by formula (Q3) below to a total peak area of the organic silicon polymer satisfies mathematical formula (3) below:



(Q3)

(In formula (Q3),  $\text{R}_F$  represents one of structures represented by formulae (i) to (iv) below:



(In formulae (i) to (iv), \* represents a bonding portion that bonds to the silicon atom. In formulae (ii) and (iv), L independently represents a methylene group, an ethylene group, or a phenylene group), and



(3)

Further features of the present invention will become apparent from the following description of exemplary embodiments with reference to the attached drawings.

#### BRIEF DESCRIPTION OF THE DRAWINGS

FIG. 1 is a diagram showing an example of a cross-sectional image of a toner particle observed with TEM.

FIG. 2 is a chart measured by  $^{29}\text{Si}$ -NMR of toner particles and includes part (a) that indicates a composite peak difference obtained by subtracting a composite peak (b) from a measurement result (d), part (b) that indicates a composite peak in which split peaks are combined, part (c) that indicates split peaks obtained by splitting the composite peak, and part (d) that indicates peaks of measurement results.

FIG. 3 is a diagram showing a reversing heat flow curve of a toner according to an embodiment of the present invention measured with a differential scanning calorimeter (DSC).

FIG. 4 is a schematic diagram of an image-forming apparatus used in examples.

#### DESCRIPTION OF THE EMBODIMENTS

The present invention will now be described in detail. A toner according to one embodiment of the invention includes toner particles each including a surface layer that contains an organic silicon polymer.

The organic silicon polymer includes a unit represented by formula (1) or (2) below:



(In formula (2), L represents a methylene group, an ethylene group, or a phenylene group.)

In a chart obtained by  $^{29}\text{Si}$ -NMR measurement of THF insoluble components of the toner particles, a ratio SQ3 of the peak area attributable to a structure represented by formula (Q3) below to a total peak area of the organic silicon polymer satisfies mathematical formula (3) below:



(Q3)

(In formula (Q3),  $\text{R}_F$  represents one of structures represented by formulae (i) to (iv) below:



(In formulae (i) to (iv), \* represents a bonding portion that bonds to the silicon atom. In formulae (ii) and (iv), L independently represents a methylene group, an ethylene group, or a phenylene group)



(3)

#### Organic Silicon Polymer

Since toner particles have surface layers that contain an organic silicon polymer having a unit represented by formula (1) or (2) above, the hydrophobicity of the surfaces of the toner particles can be improved and a toner with good environmental stability can be obtained.

The organic structure in the unit represented by formula (1) or (2) exhibits a high bonding energy to the silicon atom. Accordingly, toner particles having surface layers containing such an organic silicon polymer can exhibit good development durability.

When the ratio SQ3 of the peak area attributable to a structure represented by formula (Q3) below with respect to a total peak area of the organic silicon polymer in a chart

obtained by  $^{29}\text{Si-NMR}$  measurement of a THF insoluble components of the toner particles satisfies the formula (3) below, the surface free energy of the surfaces of the toner particles can be lowered and thus the environmental stability can be enhanced:



(In formula (Q3),  $\text{R}_F$  represents one of structures represented by formulae (i) to (iv) below (this structure may be referred to as "Q3 structure" hereinafter)



(In formulae (i) to (iv), \* represents a bonding portion that bonds to the silicon atom. In formulae (ii) and (iv), L independently represents a methylene group, an ethylene group, or a phenylene group)



Since the toner particles include surface layers containing the organic silicon polymer, bleeding of the release agent and resin components is suppressed and a toner having good storage stability, environmental stability, and development durability can be obtained. SQ3 can be controlled by adjusting the monomer type, reaction temperature, reaction time, reaction solvent, and pH.

The unit represented by formula (1) or (2) above may account for 50 mol % or more of the organic silicon polymer in order to enhance the environmental stability and low temperature fixability.

In a chart obtained by  $^{29}\text{Si-NMR}$  measurement of a THF insoluble components of the toner particles, SQ3 and a ratio SQ2 of the peak area attributable to a structure represented by formula (Q2) below (may be referred to as a "Q2 structure" hereinafter) with respect to a total peak area of the organic silicon polymer may satisfy the relationship (4) below:



(In formula (Q2),  $\text{R}_G$  and  $\text{R}_H$  each independently represent at least one selected from structures represented by formulae (i) to (iv) above)



When SQ3 is equal to or greater than SQ2, the balance between the chargeability and the durability of the toner attributable to the crosslinked siloxane structure is improved. Thus, the environmental stability and storage stability are improved. More preferably,  $(SQ3/SQ2) \geq 1.50$  and most preferably  $(SQ3/SQ2) \geq 2.00$ . SQ3/SQ2 can be

controlled by adjusting the monomer type, reaction temperature, reaction time, reaction solvent, and pH.

The organic silicon polymer having a unit represented by formula (1) or (2) above may be a polymer represented by formula (5) or (6) below.



(In formulae (5) and (6), L represents a methylene group, an ethylene group, or a phenylene group and  $\text{R}_A$  and  $\text{R}_B$  each independently represent a unit represented by formula (7) or (8) below:



(In formula (8),  $\text{R}_N$  represents a hydrogen atom or an alkyl group having 1 to 22 carbon atoms and  $\text{R}_M$  represents a hydrogen atom or a methyl group.)

When the organic silicon polymer is one represented by formula (5) or (6) above, the environmental stability and low temperature fixability are further enhanced.

$\text{R}_M$  in formula (8) represents a hydrogen atom or a methyl group that improve environmental stability.  $\text{R}_N$  in formula (8) represents a hydrogen atom or an alkyl group having 1 to 22 carbon atoms that improve the low temperature fixability and development durability.

#### Silicon Concentration at Surfaces of Toner Particles

A silicon concentration dSi of the toner at the surfaces of the toner particles is preferably 2.5 atomic % or higher, more preferably 5.0 atomic % or higher, and most preferably 10.0 atomic % or higher relative to the total of the silicon concentration dSi, the oxygen concentration dO, and the carbon concentration dC ( $d\text{Si}+d\text{O}+d\text{C}$ ) determined by electron spectroscopy for chemical analysis (ESCA) performed on the surfaces of the toner particles. ESCA is an element analysis technique of the outermost surface several nanometers in depth. When the silicon concentration in the outermost surface layers of the toner particles is 2.5 atomic % or higher, the surface free energy of the outermost surface layers can be lowered. The fluidity can be further improved and the soiling of parts and fogging can be further suppressed by adjusting the silicon concentration to 2.5 atomic % or higher.

The silicon concentration of the outermost surface layers of the toner particles determined by ESCA can be controlled by adjusting the ratio of the hydrophilic groups to the hydrophobic groups in the organic silicon polymer, reaction temperature, reaction time, reaction solvent, pH, and the content of the organic silicon polymer. For the purposes of the present invention, the "outermost surface layer" refers to a portion that extends from the surface of a toner particle (depth: 0.0 nm) to a depth of 10.0 nm toward the center of the toner particle (midpoint of the long axis).

In the toner particles, the ratio of the silicon concentration (atomic %) to the carbon concentration (atomic %) determined by ESCA is preferably 0.15 or more and 5.00 or less. At this ratio, the surface free energy can be further lowered, the storage stability can be improved, and the soiling of parts can be suppressed. The ratio of the silicon concentration to the carbon concentration is more preferably 0.20 or more and 4.00 or less and most preferably 0.30 or more in order to improve environmental stability. Average thickness  $D_{av}$  of surface layers of toner particles and percentage that surface layer thickness is 5.0 nm or less out of surface layer thicknesses  $FRA_n$ .

The average thickness  $D_{av}$  of the surface layers of the toner particles containing the organic silicon polymer and determined by observation of cross sections of the toner particles by using a transmission electron microscope (TEM) may be 5.0 nm or more and 150.0 nm or less. At this average thickness, bleeding of the release agent and the resin components can be suppressed and a toner having good storage stability, environmental stability, and development durability can be obtained. From the viewpoint of storage stability, the average thickness  $D_{av}$  of the surface layers of the toner particles is more preferably 10.0 nm or more and 150.0 nm or less and yet more preferably 10.0 nm or more and 125.0 nm or less, and most preferably 15.0 nm or more and 100.0 nm or less.

The average thickness  $D_{av}$  of the surface layers of the toner particles containing the organic silicon polymer can be controlled by adjusting the ratio of the hydrophilic groups to the hydrophobic groups in the organic silicon polymer, the reaction temperature, reaction time, reaction solvent, and pH for addition polymerization and condensation polymerization, and the content of the organic silicon polymer.

In order to increase the average thickness  $D_{av}$  (nm) of the surface layers of the toner particles, the proportion of the hydrophobic groups in the organic silicon polymer may be decreased.

In a cross section of a toner particle observed with a transmission electron microscope (TEM), sixteen straight lines that pass through the midpoint of a long axis L, which is a maximum diameter of the cross section, and extend across the cross section are drawn with reference to the long axis L such that the angles of the intersection between adjacent lines at the midpoint are equal to each other (namely, 11.25°) and that thirty-two line segments  $A_n$  ( $n=1$  to 32) that extend from the midpoint to the surface of the toner particle are formed. Assuming the length of each line segment to be  $RA_n$  ( $n=1$  to 32) and the thickness of the surface layer on a line segment  $A_n$  to be  $FRA_n$  ( $n=1$  to 32), the percentage of the surface layer thicknesses that are 5.0 nm or less out of surface layer thicknesses  $FRA_n$  may be 20.0% or less.

In the case where the percentage that the surface layer thicknesses that are 5.0 nm or less out of the surface layer thicknesses  $FRA_n$  is 20.0% or less, a toner having good image density stability and causes less fogging in a wide variety of environments can be obtained.

The average thickness  $D_{av}$  of the surface layers of the toner particles and the percentage that the surface layer thickness is 5.0 nm or less can be controlled by adjusting the ratio of the hydrophilic groups to the hydrophobic groups in the organic silicon polymer, reaction temperature, reaction time, reaction solvent, pH, and the content of the organic silicon polymer.

#### Method for Preparing Organic Silicon Polymer

A representative example of a method for preparing an organic silicon polymer according to an embodiment of the invention is a sol-gel method. In a sol-gel method, a metal alkoxide  $M(OR)_n$  ( $M$ : metal, O: oxygen, R: hydrocarbon, n: oxidation number of metal) is used as a starting material, is hydrolyzed and condensation polymerized in a solvent to form a sol, and is formed into a gel. A sol-gel method is used to synthesize glass, ceramics, organic-inorganic hybrid materials, and nano-composites. According to this method, functional materials of various forms, such as surface layers, fibers, bulks and fine particles, can be synthesized from a liquid phase at a low temperature.

In particular, surface layers of the toner particles are formed by hydrolytic polycondensation of a silicon compound such as alkoxy silane. When a surface layer is uniformly provided on the surface of each toner particle, the environmental stability is improved without fixing or adhering inorganic fine particles as in the toners of the related art. Moreover, the performance of the toner is rarely degraded in long-term use and a toner having good storage stability can be obtained.

In a sol-gel method, a solution is used in the initial stage and this solution is gelled to form a material. Thus, various fine structures and shapes can be fabricated. In particular, for toner particles formed in an aqueous medium, it is easy to provide an organic silicon compound on surfaces of toner particles due to the hydrophilicity exhibited by hydrophilic groups such as silanol groups in the organic silicon compound.

However, if the hydrophobicity of the organic silicon compound is high (for example, when the organic silicon compound contains functional groups that are highly hydrophobic), it becomes difficult to precipitate the organic silicon compound at the surface layers of the toner particles. Accordingly, it becomes difficult to form a toner particle that has a surface layer containing the organic silicon polymer.

In contrast, if the hydrophobicity of the organic silicon compound is low, the charge stability of the toner tends to be degraded. The fine structures and shapes of the toner particles can be controlled by adjusting the reaction temperature, reaction time, reaction solvent, pH, the type of the organic silicon compound, and the amount of the organic silicon compound added, for example.

The organic silicon polymer may be obtained by polymerizing a polymerizable monomer that contains a compound represented by formula (Z) below:



(In formula (Z),  $R^1$  represents a structure represented by formula (i) or (ii) and  $R^2$ ,  $R^3$ , and  $R^4$  each independently represent a halogen atom, a hydroxy group, or an alkoxy group.)

When toner particles contain, in their surface layers, an organic silicon polymer obtained by polymerizing a polymerizable monomer containing a compound represented by formula (Z) above, the hydrophobicity of the surfaces of the toner particles can be improved. As a result, the environmental stability of the toner can be further improved. To facilitate incorporation of the organic silicon polymer in the surface layers, the number of carbon atoms in R<sup>1</sup> is preferably 5 or less, more preferably 3 or less, and most preferably 2 or less. From the viewpoints of the coatability of the surface layers of the toner particles and the chargeability and durability of the toner, R<sup>1</sup> preferably represents a vinyl group or an allyl group and more preferably represents a vinyl group.

R<sup>2</sup>, R<sup>3</sup>, and R<sup>4</sup> each independently represent a halogen atom, a hydroxy group, or an alkoxy group (hereinafter may also be referred to as "reactive group"). These reactive groups undergo hydrolysis, addition polymerization, or condensation polymerization to form a crosslinked structure. Since such a crosslinked structure is formed on the surfaces of toner particles, a toner having good development durability can be obtained. In particular R<sup>2</sup>, R<sup>3</sup>, and R<sup>4</sup> preferably each independently represent an alkoxy group and more preferably each independently represent a methoxy group or an ethoxy group since hydrolysis proceeds slowly at room temperature, the organic silicon polymer can be smoothly precipitated at the surfaces of the toner particles, and the coatability on the surfaces of the toner particles is improved. Hydrolysis, addition polymerization, or condensation polymerization of R<sup>2</sup>, R<sup>3</sup>, and R<sup>4</sup> can be controlled by adjusting the reaction temperature, reaction time, reaction solvent, and pH.

Examples of the organic silicon compound represented by formula (Z) above (hereinafter may be referred to as "trifunctional silane") include trifunctional vinylsilanes such as vinyltrimethoxysilane, vinyltriethoxysilane, vinyldiethoxymethoxysilane, vinyllethoxydimethoxysilane, vinyl-trichlorosilane, vinylmethoxydichlorosilane, vinyllethoxydichlorosilane, vinyldimethoxychlorosilane, vinylmethoxyethoxychlorosilane, vinyldiethoxychlorosilane, vinyltriacetoxysilane, vinyldiacetoxymethoxysilane, vinyldiacetoxymethoxysilane, vinylacetoxymethoxysilane, vinylacetoxymethoxysilane, vinyltrihydroxysilane, vinylmethoxydihydroxysilane, vinyllethoxydihydroxysilane, vinyldimethoxyhydroxysilane, vinyllethoxymethoxyhydroxysilane, and vinyldiethoxyhydroxysilane; and trifunctional allylsilanes such as allyltrimethoxysilane, allyltriethoxysilane, allyldiethoxymethoxysilane, allylethoxydimethoxysilane, allyltrichlorosilane, allylmethoxydichlorosilane, allylethoxydichlorosilane, allyldimethoxychlorosilane, allylmethoxyethoxychlorosilane, allyldiethoxychlorosilane, allyltriacetoxysilane, allyldiacetoxymethoxysilane, allyldiacetoxymethoxysilane, allylacetoxydimethoxysilane, allylacetoxymethoxysilane, allylacetoxydiethoxysilane, allyltrihydroxysilane, allylmethoxydihydroxysilane, allylethoxydihydroxysilane, allyldimethoxyhydroxysilane, allylethoxymethoxyhydroxysilane, and allyldiethoxyhydroxysilane.

These organic silicon compounds may be used alone or in combination.

The content of the organic silicon compound represented by formula (Z) is preferably 50 mol % or more and more preferably 60 mol % or more in the organic silicon polymer. The environmental stability of the toner can be further improved when the content of the organic silicon compound represented by formula (Z) is 50 mol % or more.

An organic silicon polymer obtained by using an organic silicon compound having three functional group per molecule (trifunctional silane), an organic silicon compound having two functional groups per molecule (difunctional silane), or an organic silicon compound having one reactive group per molecule (monofunctional silane) in combination with the organic silicon compound represented by formula (Z) may also be used.

Examples of the organic silicon compound that can be used in combination with the organic silicon compound represented by formula (Z) include dimethyldiethoxysilane, tetraethoxysilane, hexamethyldisilazane, 3-glycidoxypropytrimethoxysilane, 3-glycidoxypropylmethyldiethoxysilane, 3-glycidoxypropyltriethoxysilane, p-styryltrimethoxysilane, 3-methacryloxypropylmethyldimethoxysilane, 3-methacryloxypropylmethyldiethoxysilane, 3-methacryloxypropyltriethoxysilane, 3-acryloxypropyltrimethoxysilane, 3-amino-propyltrimethoxysilane, 3-aminopropyltriethoxysilane, 3-(2-aminoethyl)aminopropyltrimethoxysilane, 3-(2-aminoethyl)aminopropyltriethoxysilane, 3-phenylaminopropyltrimethoxysilane, 3-anilinopropyltrimethoxysilane, 3-mercaptopropylmethyldimethoxysilane, 3-mercaptopropyltrimethoxysilane, 3-mercaptopropyltriethoxysilane, 3-glycidoxypropyltrimethoxysilane, 3-glycidoxypropylmethyldimethoxysilane, 3-glycidoxypropylmethyldiethoxysilane, hexamethyldisilane, tetraisocyanatesilane, methyl triisocyanatesilane, and vinyl triisocyanatesilane.

It is generally known that, in a sol-gel reaction, the bonding state of the siloxane bonds generated differs depending on the acidity of the reaction medium. To be more specific, when the reaction medium is acidic, a hydrogen ion is electrophilically added to an oxygen atom of one functional group (for example, an alkoxy group (—OR group)). Then oxygen atoms in the water molecules coordinate to a silicon atom, thereby forming a hydrosilyl group by substitution reaction. If there is enough water present, one H<sup>+</sup> attacks one oxygen atom of a reactive group (for example, an alkoxy group (—OR group)) and thus the speed of substitution reaction to hydroxy groups is low if the H<sup>+</sup> content in the reaction medium is low. As a result, polycondensation reaction occurs before all of the reactive groups attached to the silane are hydrolyzed and one-dimensional linear polymers and two-dimensional polymers are relatively easily generated.

In contrast, when the reaction medium is alkaline, hydroxide ions are added to the silicon atom and a 5-coordinated intermediate is produced during the course of the reaction. Accordingly, all of the reactive groups (for example, alkoxy groups (—OR groups)) can easily be eliminated and easily substituted into silanol groups. In particular, when a silicon compound having three or more reactive groups is used for the same silane, hydrolysis and polycondensation occurs three dimensionally and an organic silicon polymer having many three-dimensional crosslinks is formed. Moreover, the reaction ends in a short time.

In view of the above, an organic silicon polymer is preferably prepared by a sol-gel reaction in an alkaline reaction medium. In order to form the polymer in an aqueous medium, the pH may be 8.0 or more. In this manner, an organic silicon polymer that has a higher strength and higher durability can be formed. The sol-gel reaction may be performed for 5 hours or longer at a reaction temperature of 90° C. or higher. When a sol-gel reaction is performed at this reaction temperature for this reaction time, formation of coalesced particles in which silane compounds in a sol state

## 11

or a gel state on the surfaces of the toner particles are bonded to each other can be suppressed.

The organic silicon compound may be used in combination with an organic titanium compound or an organic aluminum compound.

Examples of the organic titanium compound include o-allyloxy(polyethylene oxide)triisopropoxytitanate, titanium allylacetoacetate triisopropoxide, titanium bis(triethanolamine)diisopropoxide, titanium tetra-n-butoxide, titanium tetra-n-propoxide, titanium chloride triisopropoxide, titanium chloride triisopropoxide, titanium di-n-butoxide (bis-2,4-pentanedionate), titanium chloride diethoxide, titanium diisopropoxide(bis-2,4-pentanedionate), titanium diisopropoxide bis(tetramethylheptanedionate), titanium diisopropoxide bis(ethyl acetoacetate), titanium tetraethoxide, titanium 2-ethylhexyloxide, titanium tetraisobutoxide, titanium tetraisopropoxide, titanium lactate, titanium methacrylate isopropoxide, titanium methacryloxyethyl acetoacetate triisopropoxide, (2-methacryloxyethoxy)triisopropoxy titanate, titanium tetramethoxide, titanium methoxypropoxide, titanium methylphenoxy, titanium n-nonyloxide, titanium oxide bis(pentanedionate), titanium n-propoxide, titanium stearyloxide, titanium tetrakis(bis-2,2-(allyloxyethyl)butoxide), titanium trisostearoylisopropoxide, titanium methacrylate methoxyethoxide, tetrakis(trimethylsiloxy)titanium, titanium tris(decylbenzenesulfonate) isopropoxide, and titanocene diphenoxide.

Examples of the organic aluminum compound include aluminum(III) n-butoxide, aluminum(III) s-butoxide, aluminum(III) s-butoxide bis(ethyl acetoacetate), aluminum(III) t-butoxide, aluminum(III) di-s-butoxide ethyl acetoacetate, aluminum(III) diisopropoxide ethyl acetoacetate, aluminum(III) ethoxide, aluminum(III) ethoxyethoxyethoxide, aluminum hexafluoropentanedioanate, aluminum(III) 3-hydroxy-2-methyl-4-pyronate, aluminum(III) isopropoxide, aluminum-9-octadecenyl acetoacetate diisopropoxide, aluminum(III) 2,4-pentanedionate, aluminum phenoxide, and aluminum(III) 2,2,6,6-tetramethyl-3,5-heptanedionate.

Two or more of these organic titanium compounds and two or more of the organic aluminum compounds may be used. The amount of charges can be controlled by appropriately selecting a combination of these compounds and adjusting the amount added.

The organic silicon polymer may be obtained by polymerizing the vinyl-based polymerizable monomer and the compound represented by formula (Z) above.

#### Method for Producing Toner Particles

A method for producing toner particles will now be described.

The description below provides specific embodiments of having an organic silicon polymer incorporated in surface layers of toner particles. However, the present invention is not limited to these embodiments.

A first production method includes forming particles in an aqueous medium from a polymerizable monomer composition containing a polymerizable monomer, a colorant, and an organic silicon compound and polymerizing the polymerizable monomer to obtain toner particles (hereinafter this method may also be referred to as a "suspension polymerization method").

A second production method includes preparing toner base bodies first, placing the toner base bodies in an aqueous medium, and forming surface layers of an organic silicon polymer on the toner base bodies in the aqueous medium. The toner base bodies may be obtained by melt kneading a binder resin and a colorant and pulverizing the resulting

## 12

product. Alternatively, the toner base bodies may be obtained by agglomerating and associating the binder resin particles and the colorant particles in an aqueous medium, or by suspending in an aqueous medium an organic phase dispersion, which is prepared by dissolving a binder resin, a silane compound, and a colorant in an organic solvent, so as to form particles and conduct polymerization and then removing the organic solvent.

A third production method includes suspending in an aqueous medium an organic phase dispersion, which is prepared by dissolving a binder resin, a silane compound, and a colorant in an organic solvent, so as to form particles and conduct polymerization, and then removing the organic solvent to obtain toner particles.

A fourth production method includes agglomerating and associating binder resin particles, colorant particles, and organic silicon compound-containing particles in a sol or gel state in an aqueous medium to form toner particles.

A fifth production method includes spraying a solvent containing an organic silicon compound onto surfaces of toner base bodies by a spray drying method and polymerizing or drying the surfaces by blowing hot air or by cooling so as to form surface layers containing the organic silicon compound. The toner base bodies may be obtained by melt kneading a binder resin and a colorant and pulverizing the resulting product, or by agglomerating and associating binder resin particles and colorant particles in an aqueous medium, or by suspending in an aqueous medium an organic phase dispersion, which is prepared by dissolving a binder resin, a silane compound, and a colorant in an organic solvent, so as to form particles and conduct polymerization and then removing the organic solvent.

Toner particles produced by these production methods include surface layers that contain an organic silicon polymer and thus exhibit good environmental stability (in particular, the chargeability in a severe environment). Moreover, changes in the surface state of the toner particles caused by bleeding of the release agent and the resin in the toner interior are suppressed even in a severe environment.

The toner particles obtained by these production methods may be surface-treated by applying hot air. When toner particles are surface-treated by applying hot air, condensation polymerization of the organic silicon polymer near the surfaces of the toner particles is accelerated and the environmental stability and the development durability can be improved.

A technique capable of treating surfaces of toner particles or a toner with hot air and cooling the treated toner particles by using cool air may be employed as the surface treatment that uses hot air described above. Examples of the machines used to conduct a surface treatment using hot air include Hybridization System (produced by Nara Machinery Co., Ltd.), Mechanofusion System (produced by Hosokawa Micron Corporation), Faculty (produced by Hosokawa Micron Corporation), and Meteorainbow MR type (produced by Nippon Pneumatic MFG., Co., Ltd.).

Examples of the aqueous medium used in the production methods described above include water, alcohols such as methanol, ethanol, and propanol, and mixed solvents of these.

Among the production methods described above, the first production method (suspension polymerization method) may be employed to produce toner particles. According to the suspension polymerization method, it is easy to have an organic silicon polymer uniformly precipitated in surfaces of the toner particles, good adhesion is achieved between the surface layers and the interiors of the toner particles, and the

storage stability, the environmental stability, and the development durability are enhanced. The suspension polymerization method is described in further detail below.

If needed, a release agent, a polar resin, and a low-molecular-weight resin may be added to the polymerizable monomer composition described above. Upon completion of the polymerization step, the particles generated may be washed and recovered by filtration, and dried to obtain toner particles. Heating may be conducted in the latter half of the polymerization step. In order to remove unreacted polymerizable monomer and by-products, part of the dispersion medium may be distilled away from the reaction system in the latter half of the polymerization step or after completion of the polymerization step.

#### Low-Molecular-Weight Resin

The following resins can be used as the low-molecular-weight resin as long as the effects of the invention are not impaired: homopolymers of styrene or its substitutes such as polystyrene and polyvinyl toluene; styrene-based copolymers such as a styrene-propylene copolymer, a styrene-vinyl toluene copolymer, a styrene-vinyl naphthalene copolymer, a styrene-methyl acrylate copolymer, a styrene-ethyl acrylate copolymer, a styrene-butyl acrylate copolymer, a styrene-octyl acrylate copolymer, a styrene-dimethylaminoethyl acrylate copolymer, a styrene-methyl methacrylate copolymer, a styrene-ethyl methacrylate copolymer, a styrene-butyl methacrylate copolymer, a styrene-dimethylaminoethyl methacrylate copolymer, a styrene-vinyl methyl ether copolymer, a styrene-vinyl ethyl ether copolymer, a styrene-vinyl methyl ketone copolymer, a styrene-butadiene copolymer, a styrene-isoprene copolymer, a styrene-maleic acid copolymer, and a styrene-maleic acid ester copolymer; and polymethyl methacrylate, polybutyl methacrylate, polyvinyl acetate, polyethylene polypropylene, polyvinyl butyral, silicone resin, polyester resin, polyamide resin, epoxy resin, polyacrylic resin, rosin, modified rosin, terpene resin, phenolic resin, aliphatic or alicyclic hydrocarbon resin, and aromatic petroleum resin.

These resins may be used alone or in combination.

In order to address changes in viscosity of the toner at high temperature, the resin may contain a polymerizable functional group. Examples of the polymerizable functional group include a vinyl group, an isocyanate group, an epoxy group, an amino group, a carboxylic acid group, and a hydroxy group.

The weight-average molecular weight (Mw) of the THF soluble of the low-molecular-weight resin determined by GPC may be 2000 to 6000.

#### Polar Resin

The polar resin may be a saturated or unsaturated poly-ester-based resin.

Examples of the polyester-based resin include those obtained by condensation polymerization of an acid component monomer and an alcohol component monomer. Examples of the acid component monomer include terephthalic acid, isophthalic acid, phthalic acid, cyclohexanedicarboxylic acid, and trimellitic acid.

Examples of the alcohol component monomer include bisphenol A, hydrogenated bisphenol, ethylene oxide adducts of bisphenol A, propylene oxide adducts of bisphenol A, glycerin, trimethylol propane, and pentaerythritol.

#### Release Agent

Examples of the release agent include petroleum-based wax and derivatives thereof such as paraffin wax, microcrystalline wax, and petrolatum, montan wax and derivatives thereof, Fisher-Tropsch hydrocarbon wax and derivatives thereof, polyolefin wax and derivatives thereof such as

polyethylene and polypropylene, natural wax and derivatives thereof such as carnauba wax and candelilla wax, higher aliphatic alcohols, fatty acids and compounds thereof such as stearic acid and palmitic acid, acid amide wax, ester wax, ketone, hydrogenated castor oil and derivatives thereof, vegetable wax, animal wax, and silicone resin.

The derivatives also refer to oxides, block copolymers with vinyl-based monomers, and graft modified products.

#### Polymerizable Monomer

10 The following vinyl-based polymerizable monomers can be used in addition to the compound represented by formula (Z) above as the polymerizable monomer used in the suspension polymerization method: styrene; styrene derivatives such as  $\alpha$ -methylstyrene,  $\beta$ -methylstyrene, o-methylstyrene, m-methylstyrene, p-methylstyrene, 2,4-dimethylstyrene, p-n-butylstyrene, p-tert-butylstyrene, p-n-hexylstyrene, p-n-octylstyrene, p-n-nonylstyrene, p-n-decylstyrene, p-n-dodecylstyrene, p-methoxystyrene, and p-phenylstyrene; acryl-based polymerizable monomers such as methyl acrylate, 15 ethyl acrylate, n-propyl acrylate, iso-propyl acrylate, n-butyl acrylate, iso-butyl acrylate, tert-butyl acrylate, n-amyl acrylate, n-hexyl acrylate, 2-ethylhexyl acrylate, n-octyl acrylate, n-nonyl acrylate, cyclohexyl acrylate, benzyl acrylate, 20 dimethyl phosphate ethyl acrylate, diethyl phosphate ethyl acrylate, dibutyl phosphate ethyl acrylate, and 2-benzyloxy ethyl acrylate; methacryl-based polymerizable monomers such as methyl methacrylate, ethyl methacrylate, n-propyl methacrylate, iso-propyl methacrylate, n-butyl methacrylate, 25 iso-butyl methacrylate, tert-butyl methacrylate, n-amyl methacrylate, n-hexyl methacrylate, 2-ethylhexyl methacrylate, n-octyl methacrylate, n-nonyl methacrylate, diethyl phosphate ethyl methacrylate, and dibutyl phosphate ethyl methacrylate; esters of methylene aliphatic monocarboxylic acids; vinyl esters such as vinyl acetate, vinyl propionate, 30 vinyl benzoate, vinyl butyrate, and vinyl formate; vinyl ethers such as vinyl methyl ether, vinyl ethyl ether, and vinyl isobutyl ether; and vinyl methyl ketone, vinyl hexyl ketone, and vinyl isopropyl ketone.

Among these vinyl-based polymers, styrene-based polymers, styrene-acryl-based copolymers, and styrene-methacryl-based copolymers are preferable. The adhesion with the organic silicon polymer is improved and the storage stability and the development durability are enhanced.

#### Other Additives

45 In polymerizing the polymerizable monomer, a polymerization initiator may be added.

Examples of the polymerization initiator include azo- or diazo-based polymerization initiators such as 2,2'-azobis-(2,4-divaleronitrile), 2,2'-azobisisobutyronitrile, 1,1'-azobis (cyclohexane-1-carbonitrile), 2,2'-azobis-4-methoxy-2,4-dimethylvaleronitrile, azobisisobutyronitrile; and peroxide-based polymerization initiators such as benzoyl peroxide, methyl ethyl ketone peroxide, diisopropyl peroxide, cumene hydroperoxide, 2,4-dichlorobenzoyl peroxide, and lauroyl peroxide.

The amount of the polymerization initiator added may be 0.5 to 30.0 mass % relative to the polymerizable monomer. Two or more polymerization initiators may be used in combination.

60 In order to control the molecular weight of the binder resin contained in the toner particles, a chain transfer agent may be added in polymerizing the polymerizable monomer. The amount of the chain transfer agent added may be 0.001 to 15.000 mass % of the polymerizable monomer.

65 In order to control the molecular weight of the binder resin contained in the toner particles, a crosslinking agent may be added in polymerizing the polymerizable monomer.

Examples of the crosslinking agent include divinylbenzene, bis(4-acryloxyethoxyphenyl)propane, ethylene glycol diacrylate, 1,3-butylene glycol diacrylate, 1,4-butanediol diacrylate, 1,5-pentanediol diacrylate, 1,6-hexanediol diacrylate, neopentyl glycol diacrylate, diethylene glycol diacrylate, triethylene glycol diacrylate, tetraethylene glycol diacrylate, #200, #400, and #600 diacrylates of polyethylene glycol, dipropylene glycol diacrylate, polypropylene glycol diacrylate, polyester-type diacrylate (MANDA produced by Nippon Kayaku Co., Ltd.), and methacrylates of the foregoing.

Examples of a polyfunctional crosslinking agent include pentaerythritol triacrylate, trimethylol ethane triacrylate, trimethylol propane triacrylate, tetramethylol methane tetraacrylate, oligo ester acrylate and methacrylate, 2,2-bis(4-methacryloxyethoxyphenyl)propane, diacryl phthalate, triallyl cyanurate, triallyl isocyanurate, triallyl trimellitate, and diallyl chlorendate.

The amount of the crosslinking agent added may be 0.001 to 15.000 mass % relative to the polymerizable monomer.

#### Binder Resin

The binder resin contained in the toner particles is preferably a vinyl-based resin and more preferably a styrene-based resin, a styrene-acryl-based resin, or a styrene-methacryl-based resin. A vinyl-based resin is synthesized as a result of polymerization of the vinyl-based polymerizable monomer described above. Vinyl-based resins have excellent environmental stability. Vinyl-based resins are also advantageous since they give highly uniform surfaces and cause an organic silicon polymer obtained by polymerization of a polymerizable monomer containing a compound represented by formula (Z) to precipitate in the surfaces of the toner particles.

#### Dispersion Stabilizer

In the case where the medium used in polymerizing the polymerizable monomer is an aqueous medium, the following can be used as the dispersion stabilizer for particles of the polymerizable monomer composition: hydroxyapatite, tricalcium phosphate, magnesium phosphate, zinc phosphate, aluminum phosphate, calcium carbonate, magnesium carbonate, calcium hydroxide, magnesium hydroxide, aluminum hydroxide, calcium metasilicate, calcium sulfate, barium sulfate, bentonite, silica, and alumina. Examples of the organic dispersion stabilizer include polyvinyl alcohol, gelatin, methyl cellulose, methyl hydroxypropyl cellulose, ethyl cellulose, carboxymethyl cellulose sodium salt, and starch.

Commercially available nonionic, anionic, and cationic surfactants can also be used.

Examples of the surfactant include sodium dodecyl sulfate, sodium tetradecyl sulfate, sodium pentadecyl sulfate, sodium octyl sulfate, sodium oleate, sodium laurate, and potassium stearate.

In the case where a slightly water-soluble inorganic dispersion stabilizer is used to prepare an aqueous medium, the amount of the dispersion stabilizer added may be 0.2 to 2.0 parts by mass per 100.0 parts by mass of the polymerizable monomer. The aqueous medium may be prepared by using 300 to 3,000 parts by mass of water per 100 parts by mass of the polymerizable monomer composition.

A commercially available dispersion stabilizer can be directly used in preparing an aqueous medium in which the slightly water-soluble inorganic dispersion stabilizer is dispersed. In order to obtain a dispersion stabilizer having fine and uniform particle size, a slightly water-soluble inorganic dispersion stabilizer may be generated in a liquid medium such as water under stirring at high speed. In particular, in

the case where tricalcium phosphate is used as the dispersion stabilizer, an aqueous solution of sodium phosphate and an aqueous solution of calcium chloride may be mixed under stirring at high speed so as to form fine particles of tricalcium phosphate and to obtain a desirable dispersion stabilizer.

#### Colorant

Examples of the colorant used in the toner are as follows.

Examples of the yellow pigment include iron oxide yellow, Naples Yellow, Naphthol Yellow S, Hansa yellow G, Hansa Yellow 10G, Benzidine Yellow G, Benzidine Yellow GR, Lake Quinoline Yellow, Permanent Yellow NCG, Lake Tartrazine, condensed azo compounds, isoindolinone compounds, anthraquinone compounds, azo metal complexes, methine compounds, and allylamide compounds.

Specific examples thereof include C.I. Pigment Yellow 12, C.I. Pigment Yellow 13, C.I. Pigment Yellow 14, C.I. Pigment Yellow 15, C.I. Pigment Yellow 17, C.I. Pigment Yellow 62, C.I. Pigment Yellow 74, C.I. Pigment Yellow 83, C.I. Pigment Yellow 93, C.I. Pigment Yellow 94, C.I. Pigment Yellow 95, C.I. Pigment Yellow 109, C.I. Pigment Yellow 110, C.I. Pigment Yellow 111, C.I. Pigment Yellow 128, C.I. Pigment Yellow 129, C.I. Pigment Yellow 147, C.I. Pigment Yellow 155, C.I. Pigment Yellow 168, and C.I. Pigment Yellow 180.

Examples of an orange pigment includes Permanent Orange GTR, Pyrazolone Orange, Vulcan Orange, Benzidine Orange G, Indanthrene Brilliant Orange RK, and Indanthrene Brilliant Orange GK.

Examples of a red pigment include red iron oxide, Permanent Red 4R, Lithol Red, Pyrazolone Red, Watching Red Calcium Salt, Lake Red C, Lake Red D, Brilliant Carmine 6B, Brilliant Carmine 3B, Eosine Lake, Rhodamine B Lake, Alizarin Lake, condensed azo compounds, diketopyrrolopyrrole compounds, anthraquinone, quinacridone compounds, basic dye lake compounds, naphthol compounds, benzimidazolone compounds, thioindigo compounds, and perylene compounds.

Specific examples thereof include C.I. Pigment Red 2, C.I. Pigment Red 3, C.I. Pigment Red 5, C.I. Pigment Red 6, C.I. Pigment Red 7, C.I. Pigment Red 23, C.I. Pigment Red 48:2, C.I. Pigment Red 48:3, C.I. Pigment Red 48:4, C.I. Pigment Red 57:1, C.I. Pigment Red 81:1, C.I. Pigment Red 122, C.I. Pigment Red 144, C.I. Pigment Red 146, C.I. Pigment Red 166, C.I. Pigment Red 169, C.I. Pigment Red 177, C.I. Pigment Red 184, C.I. Pigment Red 185, C.I. Pigment Red 202, C.I. Pigment Red 206, C.I. Pigment Red 220, C.I. Pigment Red 221, and C.I. Pigment Red 254.

Examples of a blue pigment include Alkali Blue Lake, Victoria Blue Lake, Phthalocyanine Blue, Metal-free Phthalocyanine Blue, Phthalocyanine Blue partial chlorides, Fast Sky Blue, Indanthrene Blue BG, and other copper phthalocyanine compounds and derivatives thereof, anthraquinone compounds, and basic dye lake compounds.

Specific examples thereof include C.I. Pigment Blue 1, C.I. Pigment Blue 7, C.I. Pigment Blue 15, C.I. Pigment Blue 15:1, C.I. Pigment Blue 15:2, C.I. Pigment Blue 15:3, C.I. Pigment Blue 15:4, C.I. Pigment Blue 60, C.I. Pigment Blue 62, and C.I. Pigment Blue 66.

Examples of a purple pigment include Fast Violet B and Methyl Violet Lake.

Examples of a green pigment include Pigment Green B, Malachite Green Lake, and Final Yellow Green G.

Examples of a white pigment include zinc oxide, titanium oxide, antimony white, and zinc sulfide.

Examples of a black pigment include carbon black, aniline black, nonmagnetic ferrite, magnetite, and those pig-

ments adjusted to have a black color by using the yellow colorants, the red colorants, and the blue colorants described above. These colorants can be used alone, in combination as a mixture, or in a solid solution form.

Care should be paid to the polymerization inhibiting effect of the colorant and the colorant's tendency to make transition into a dispersion medium depending on the toner production method. If needed, the colorant may be surface treated with a substance that does not inhibit polymerization so as to modify the surface. In particular, many dyes and carbon black exhibit polymerization inhibiting effects and care should be taken in using these.

An example of a method suitable for treating a dye include polymerizing a Polymerizable monomer in the presence of a dye in advance, and adding a polymerizable monomer composition to the resulting colored polymer. In the case where carbon black is used, the carbon black can be treated in the same way as the dye or can be treated with a substance (for example, organosiloxanes) that reacts with surface functional groups of the carbon black.

The colorant content may be 3.0 to 15.0 parts by mass per 100.0 parts by mass of the binder resin or the polymerizable monomer.

#### Charge Control Agent

The toner may contain a charge control agent. The charge control agent may be any available charge control agent. In particular, a charge control agent that exhibits a high charging speed and can stably maintain a particular amount of charges may be used. In the case where toner particles are produced by a direct polymerization method, a charge control agent that has a low polymerization inhibition effect and is substantially free of substances soluble in the aqueous medium may be used.

Examples of the charge control agent capable of forming negative charge toners include organic metal compounds and chelating compounds such as monoazo metal compounds, acetylacetone metal compounds, and metal compounds based on aromatic oxycarboxylic acids, aromatic dicarboxylic acids, oxycarboxylic acids, and dicarboxylic acids. Other examples include aromatic oxycarboxylic acids, aromatic mono- and poly-carboxylic acids and metal salts thereof, anhydrides, esters, and phenol derivatives such as bisphenol. Yet other examples include urea derivatives, metal-containing salicylic acid-based compounds, metal-containing naphthoic acid-based compounds, boron compounds, quaternary ammonium salts, and calixarene.

Examples of the charge control agent capable of forming positive charge toners include nigrosin and modified nigrosin such as fatty acid metal salts; guanidine compounds; imidazole compounds; quaternary ammonium salts, onium salts thereof such as phosphonium salts which are analogs of these, and lake pigments thereof such as tributylbenzyl ammonium-1-hydroxy-4-naphthosulfonic acid salt and tetrabutyl ammonium tetrafluoroborate; triphenyl methane dyes and lake pigments thereof (examples of the lake agent include phosphotungstic acid, phosphomolybodic acid, phosphotungstomolybodic acid, tannic acid, lauric acid, gallic acid, ferricyanide, and ferrocyanide); metal salts of higher aliphatic acids; and resin-based charge control agents.

These charge control agents may be used alone or in combination.

Among these charge control agents, metal-containing salicylic acid-based compounds are preferable and more preferably the metal is aluminum or zircon. Of these, 3,5-di-tert-butyl salicylic acid aluminum compound is most preferable.

The charge control resin may be a polymer having a sulfonic acid-based functional group. A polymer having a sulfonic acid-based functional group refers to a polymer or copolymer that has a sulfonic acid group, a sulfonic acid base, or a sulfonic acid ester group.

Examples of the polymer or copolymer that has a sulfonic acid group, a sulfonic acid base, or a sulfonic acid ester group include polymer-type compounds having sulfonic acid groups in the side chains. From the viewpoint of 10 improving the charge stability at high humidity, a polymer-type compound which is a styrene and/or styrene (meth) acrylic acid ester copolymer that has a glass transition temperature (Tg) of 40° C. to 90° C. and contains 2 mass % or more and preferably 5 mass % or more of a sulfonic acid group-containing (meth)acrylamide-based monomer in 15 terms of a copolymerization ratio may be used. With this compound, the charge stability at high humidity is improved.

The sulfonic acid group-containing (meth)acrylamide-based monomer may be one represented by general formula (X) below. Examples thereof include 2-acrylamide-2-methyl propanoic acid and 2-methacrylamide-2-methyl propanoic acid.



(In formula (X), R<sup>11</sup> represents a hydrogen atom or a methyl group, R<sup>12</sup> and R<sup>13</sup> each independently represents a hydrogen atom or an alkyl group, alkenyl group, aryl group, or alkoxy group having 1 to 10 carbon atoms, and n represents an integer in the range of 1 to 10.)

The polymer having a sulfonic acid group may be contained in an amount of 0.1 to 10.0 parts by mass per 100 parts by mass of the binder resin in the toner particles so that the charge state of the toner can be further improved when used in combination with a water-soluble initiator.

The amount of the charge control agent added may be 0.01 to 10.00 parts by mass per 100 parts by mass of the binder resin or the polymerizable monomer.

#### Organic Fine Particles and Inorganic Fine Particles

Various types of organic fine particles and inorganic fine particles may be externally added to the toner particles so as to impart various properties to the toner. The organic fine particles and the inorganic fine particles may have a particle size equal to or smaller than  $\frac{1}{10}$  of the weight-average particle size of the toner particles considering the durability of these particles added to the toner particles.

55 Examples of the organic fine particles and inorganic fine particles are as follows:

- (1) Fluidity imparting agent: silica, alumina, titanium oxide, carbon black, and fluorinated carbon;
- (2) Abrasives: metal oxides such as strontium titanate, cerium oxide, alumina, magnesium oxide, and chromium oxide; nitrides such as silicon nitride; carbide such as silicon carbide; and metal salts such as calcium sulfate, barium sulfate, and calcium carbonate;
- (3) Lubricant: fluorine-based resin powders such as vinylidene fluoride and polytetrafluoroethylene and aliphatic acid metal salts such as zinc stearate and calcium stearate; and

(4) Charge control particles: metal oxides such as tin oxide, titanium oxide, zinc oxide, silica, and alumina, and carbon black.

The organic fine particles or inorganic fine particles are used as the material for treating the surfaces of the toner particles in order to improve the fluidity of the toner and make the charges of the toner uniform. Since the chargeability of the toner can be controlled and the charge properties in a high humidity environment can be improved by hydrophobing the organic fine particles or the inorganic fine particles, hydrophobized organic or inorganic fine particles may be used. If organic fine particles or inorganic fine particles added to the toner absorb humidity, the chargeability of the toner is degraded and the developing performance and the transfer property tend to be lowered.

Examples of the treating agent used for hydrophobing the organic fine particles or inorganic fine particles include unmodified silicone varnishes, various modified silicone varnishes, unmodified silicone oils, various modified silicone oils, silane compounds, silane coupling agents, other silicon compounds, and organic titanium compounds. These treating agents may be used alone or in combination.

In particular, inorganic fine particles treated with a silicone oil are preferably used. More preferably, inorganic fine particles are hydrophobized with a coupling agent and, at the same time or after this treatment, treated with a silicone oil. Hydrophobized inorganic fine particles treated with a silicone oil help maintain the charge amount of the toner high even in a high humidity environment and reduce the selective developing performance.

The amount of the organic fine particles or the inorganic fine particles added is preferably 0.01 to 10.00 parts by mass, more preferably 0.02 to 1.00 parts by mass, and most preferably 0.03 to 1.00 parts by mass per 100.00 parts by mass of the toner particles. At this amount, penetration of organic fine particles or inorganic fine particles into interior of the toner particles is suppressed and non-soiling property is enhanced. The organic fine particles or the inorganic fine particles may be used alone or in combination.

The BET specific surface area of the organic fine particles or the inorganic fine particles may be 10 m<sup>2</sup>/g or more and 450 m<sup>2</sup>/g or less.

The BET specific surface area of the organic fine particles or the inorganic fine particles can be determined in accordance with a BET method (preferably a BET multipoint method) through a dynamic flow method and a low-temperature gas adsorption method. For example, a specific surface area meter "GEMINI 2375 Ver. 5.0" (product of Shimadzu Corporation) is used to allow nitrogen gas to adsorb onto surfaces of samples and conduct measurement by a BET multipoint method so as to calculate the BET specific surface area (m<sup>2</sup>/g).

The organic fine particles or the inorganic fine particles may be strongly fixed or attached to the surfaces of the toner particles. This can be achieved by using a HENSCHEL MIXER MECHANOFUSION, CYCLOMIX, TURBULIZER, FLEXOMIX, HYBRIDIZATION, MECHNOHYD-BRID, or NOBILTA, for example.

The organic fine particles or the inorganic fine particles can be strongly fixed or attached to the surfaces of the toner particles by increasing the rotation peripheral speed or extending the treatment time.

#### Physical Properties of Toner

The physical properties of the toner will now be described.

##### 80° C. Viscosity

The 80° C. viscosity of the toner measured with a constant-pressure extrusion system capillary rheometer may be 1,000 Pa·s or more and 40,000 Pa·s or less. When the 80° C. viscosity is within the range of 1,000 to 40,000 Pa·s, the toner exhibits good low-temperature fixability. The 80° C. viscosity is more preferably in the range of 2,000 Pa·s to 20,000 Pa·s. The 80° C. viscosity can be controlled by adjusting the amount of the low-molecular-weight resin added, the type of monomer used for producing the binder resin, the amount of the initiator, the reaction temperature, and the reaction time.

The 80° C. viscosity of the toner measured with the constant-pressure extrusion system capillary rheometer can be determined through the following procedure.

FLOW TESTER CFT-500D (produced by Shimadzu Corporation) is used as a measurement instrument, for example, and measurement is conducted under the following conditions.

Sample: About 1.0 g of the toner is weighed and pressure-compacted at a load of 100 kg/cm<sup>2</sup> for 1 minute to prepare a sample.

Die bore size: 1.0 mm

Die length: 1.0 mm

Cylinder pressure: 9.807×10<sup>5</sup> (Pa)

Measurement mode: ascending temperature method

Temperature ascending rate: 4.0° C./min

The viscosity (Pa·s) of the toner in the temperature range of 30° C. to 200° C. is measured by the above-described procedure and the 80° C. viscosity (Pa·s) is determined. The resulting value is assumed to be the 80° C. viscosity measured with a constant-pressure extrusion system capillary rheometer.

##### Weight-Average Particle Size (D4)

The weight-average particle size (D4) of the toner is preferably 4.0 to 9.0 µm, more preferably 5.0 to 8.0 µm, and most preferably 5.0 to 7.0 µm.

##### Glass Transition Temperature (T<sub>g</sub>)

The glass transition temperature (T<sub>g</sub>) of the toner is preferably 35° C. to 100° C., more preferably 40° C. to 80° C., and most preferably 45° C. to 70° C. When the glass transition temperature is within this range, blocking resistance, low-temperature offset resistance, and transparency of the projection images on the films for overhead projectors can be further improved.

##### THF Insoluble Content

The content of substances insoluble in tetrahydrofuran (THF) (hereinafter referred to as THF insoluble content) is preferably less than 50.0 mass %, more preferably 0.0 mass % or more and less than 45.0 mass %, and most preferably 5.0 mass % or more and less than 40.0 mass % relative to the toner components in the toner other than the colorant and the inorganic fine particles. When the THF insoluble content is less than 50.0 mass %, the low-temperature fixability can be improved.

The THF insoluble content of the toner refers to the mass ratio of the ultra high molecular weight polymer (substantially a crosslinked polymer) which became insoluble in the THF solvent. For the purposes of the present invention, the THF insoluble content is the value measured by the following procedure.

One gram of the toner is weighed (W1 g), placed in a cylindrical filter (for example, No. 86R produced by Toyo Roshi Kaisha, Ltd.), and loaded in a Soxhlet extractor.

21

Extraction is conducted for 20 hours by using 200 mL of THF as a solvent and the soluble components extracted with the solvent are condensed and vacuum dried for several hours at 40° C. Then the THF soluble resin components are weighed (W2 g). The weight of components, such as a pigment, other than the resin components in the toner is assumed to be W3 g. The THF insoluble content can be determined from the following equation:

$$\text{THF insoluble content (mass \%)} = \frac{(W1 - (W3 + W2))}{(W1 - W3)} \times 100$$

The THF insoluble content of the toner can be controlled by adjusting the degree of polymerization and degree of crosslinking of the binder resin.

Weight-Average Molecular Weight (Mw) and Weight-Average Molecular Weight (Mw)/Number-Average Molecular Weight (Mn)

The weight-average molecular weight (Mw) of the toner measured by gel permeation chromatography (GPC) performed on the tetrahydrofuran (THF) soluble components (hereinafter also referred to as "weight-average molecular weight of the toner") may be in the range of 5,000 to 50,000. When the weight-average molecular weight (Mw) of the toner is in this range, blocking resistance, development durability, and low-temperature fixability can be improved and high-gloss images can be produced. The weight-average molecular weight (Mw) of the toner can be controlled by adjusting the amount and the weight-average molecular weight (Mw) of the low-molecular-weight resin added, the reaction temperature and reaction time for toner production, and the amount of initiator, the amount of the chain transfer agent, and the amount of the crosslinking agent used for toner production.

The ratio (Mw/Mn) of the weight-average molecular weight (Mw) to the number-average molecular weight (Mn) of the toner determined by GPC performed on the tetrahydrofuran (THF) soluble components is preferably in the range of 5.0 to 100.0 and more preferably in the range of 5.0 to 30.0. When the Mw/Mn is within this range, the temperature range in which fixing is possible can be widened. Method for Measuring and Evaluating Physical Properties of Toner Particles or Toner

Methods for measuring and evaluating physical properties of the toner particles or toner will now be described.

Method for Determining Structure of Organic Silicon Polymer Method for Preparing THF Insoluble Components of Toner Particles

The THF insoluble components of the toner particles are prepared as follows.

Ten grams of a toner is weighed, placed in a cylindrical filter (for example, No. 86R produced by Toyo Roshi Kaisha, Ltd.), and loaded in a Soxhlet extractor. Extraction is conducted for 20 hours by using 200 mL of THF as a solvent and the residue in the cylindrical filter is vacuum dried for several hours at 40° C. The resulting product is assumed to be the THF insoluble components of the toner particles for NMR measurement.

Method for Confirming Presence of Unit Represented by Formula (1) or (2) Above

The presence of the unit represented by formula (1) or (2) above is confirmed by checking whether a methine group bonded to the silicon atom in formula (1) ( $>\text{CH—Si}$ ) is present or not or whether a methylene group bonded to the silicon atom in formula (2) ( $—\text{CH}_2\text{—Si}$ ) is present or not by  $^{13}\text{C}$ -NMR.

22

Measurement conditions for  $^{13}\text{C}$ -NMR (solid)

Instrument: AVANCE III 500 produced by Bruker Corporation

Probe: 4 mm MAS BB/1H

5 Measurement temperature: room temperature

Sample rotation speed: 6 kHz

Sample: 150 mg of a measurement sample (THF insoluble components of the toner particles for NMR measurement) is placed in a sample tube having a diameter of 4 mm.

10 Measurement nuclear frequency: 125.77 MHz

Reference substance: Glycine (external standard: 176.03 ppm)

Measurement width: 37.88 kHz

15 Measurement method: CP/MAS

Contact time: 1.75 ms

Repeating time: 4 s

Number of transients: 2048

LB value: 50 Hz

20 The presence of the unit represented by formula (1) above is confirmed by confirming whether a signal attributable to the methine group bonded to the silicon atom in formula (1) ( $>\text{CH—Si}$ ) is detected.

The presence of the unit represented by formula (2) above 25 is confirmed by confirming whether a signal attributable to the methylene group bonded to the silicon atom in formula (2) ( $—\text{CH}_2\text{—Si}$ ) is detected. Method for confirming the presence of the structures Q1 to Q4 and method for determining the quantities thereof

30 The presence of the structures Q1 to Q4 in the toner particles is confirmed through  $^{29}\text{Si}$ -NMR.

The structures Q1 to Q4 refer to those represented by formulae (Q1) to (Q4) below.

Structure Q1



(In formula (Q1),  $\text{R}_I$ ,  $\text{R}_J$ , and  $\text{R}_K$  each independently represent one of the structures represented by formulae (i) to (iv) below:



65 (In formulae (i) to (iv), \* represents a bonding portion that bonds to the silicon atom; and in formulae (ii) and (iv), L independently represents a methylene group, an ethylene group, or a phenylene group.)

Structure Q2



(Q2)

5

(In formula (Q2),  $R_G$  and  $R_H$  each independently represent one of the structures represented by formula (i) to (iv) above.)  
10

Structure Q3



(Q3)

(In the formula (Q3),  $R_F$  represents one of the structures represented by formula (i) to (iv) above.)  
15

Structure Q4



(Q4)

Measurement conditions for  $^{29}Si$ -NMR (solid)  
Instrument: AVANCE III 500 produced by Bruker Corporation  
Probe: 4 mm MAS BB/1H  
Measurement temperature: room temperature  
Sample rotation speed: 6 kHz  
Sample: 150 mg of a measurement sample (THF insoluble components of the toner particles for NMR measurement) is placed in a sample tube having a diameter of 4 mm.  
Measurement angular frequency: 99.36 MHz  
Reference substance: DSS (external standard: 1.534 ppm)  
Measurement width: 29.76 kHz  
Measurement method: DD/MAS, CP/MAS  
 $^{29}Si$  90°

Pulse width: 4.00  $\mu$ s

Contact time: 1.75 ms to 10 ms

Repeating time: 30 s (DD/MASS), 10 s (CP/MAS)

Number of transients: 2048

LB value: 50 Hz

After the measurement, peaks of silane components having different substituents and bonding groups in the toner particles are split into the structures Q1 to Q4 by curve fitting and the amount of each component in terms of mol % is calculated from the area ratio of the corresponding peak. In the structure Q1,  $R_P$ ,  $R_J$ , and  $R_K$  are bonded to the silicon atom. In the structure Q2,  $R_G$  and  $R_H$  are bonded to the silicon atom. In the structure Q3,  $R_F$  is bonded to the silicon atom. In the structure Q4, the center silicon atom is bonded to oxygen atoms. The curve fitting is performed by using software for JNM-EX400, namely, EXcalibur for Windows version 4.2 (EX series).  
40

Specifically, first, a menu icon 1D Pro is clicked to read measurement data. Then “Curve fitting function” is selected from “Command” in the menu bar to perform curve fitting. One example is shown in FIG. 2. Peak splitting is performed so that the composite peak difference (a), which is the difference between the composite peak (b) and the measurement result (d), is smallest.  
45

The areas of the structures Q1 to Q4 were determined as such.  
50

SQ1 to SQ4 were determined from the areas of the structures Q1 to Q4 by using the equations described below.  
55

For the purposes of the present invention, the silane monomer is identified through a chemical shift value and the unreacted monomer components were eliminated from the total peak area measured by  $^{29}Si$ -NMR of the toner particles. The resulting total area of the structures Q1 to Q4 is assumed to be the total peak area of the polymer.  
60

SQ1+SQ2+SQ3+SQ4=1.00

SQ1=area of structure Q1/(area of structure Q1+area of structure Q2+area of structure Q3+area of structure Q4)  
5

SQ2=area of structure Q2/(area of structure Q1+area of structure Q2+area of structure Q3+area of structure Q4)  
10

SQ3=area of structure Q3/(area of structure Q1+area of structure Q2+area of structure Q3+area of structure Q4)  
15

SQ4=area of structure Q4/(area of structure Q1+area of structure Q2+area of structure Q3+area of structure Q4)  
20

For the structures Q1 to Q4 above, examples of the chemical shift values of the silicon atom when the structures of  $R_P$ ,  $R_J$ ,  $R_K$ ,  $R_G$ ,  $R_H$ , and  $R_F$  are identified are as follows:  
Structure Q1 ( $R_P$ ,  $R_J$ =—OCH<sub>3</sub>,  $R_K$ =—CH—CH<sub>2</sub>): -43

20 ppm to -63 ppm, broad peak

Structure Q2 ( $R_G$ =—OCH<sub>3</sub>,  $R_H$ =—CH—CH<sub>2</sub>): -71 ppm

Structure Q3 ( $R_F$ =—CH—CH<sub>2</sub>): -81 ppm

The chemical shift value of silicon when the Q4 structure is present is as follows:  
25

Structure Q4: -108 ppm

In the case where the structure of the unit represented by formula (1) or (2) above needs to be confirmed in more detail, identification may be conducted based on the measurement results of  $^1H$ -NMR in addition to those of  $^{13}C$ -NMR and  $^{29}Si$ -NMR.  
30

Average thickness Dav. of surface layers of toner particles measured by observation of cross sections of toner particles with transmission electron microscope (TEM) and determining percentage of surface layer thicknesses that are 5.0 nm or less  
35

The cross sections of the toner particles can be observed by the following procedure.  
40

First, toner particles are dispersed in an epoxy resin curable at room temperature. The resulting dispersion is left in a 40° C. atmosphere for 2 days to cure the epoxy resin. Thin samples are cut out from the resulting cured product by using a microtome equipped with diamond knives. The cross section of each sample is observed with a transmission electron microscope (TEM) at a magnification of  $\times 10,000$  to  $\times 100,000$ . For the purposes of the present invention, observation is performed by utilizing the difference in atomic weight between the binder resin used and the organic silicon polymer since a portion with a higher atomic weight appears in light color. Moreover, in order to enhance the contrast between different materials, a ruthenium tetroxide staining method or an osmium tetroxide staining method may be employed.  
45

A TEM bright field image is acquired by using an electron microscope, TECNAI TF20XT produced by FEI Company at an acceleration voltage of 200 kV. Then an EF mapping image of a Si—K edge (99 eV) is acquired by a three window method by using an EELS detector, GIF TRIDIEM produced by Gatan Inc., so as to confirm presence of the organic silicon polymer at the surface layer.  
50

The toner particles used as the subject of the measurement for determining the average thickness Dav. of the surface layers of the toner particles and the percentage of the surface layer with a thickness of 5.0 nm or less by using a TEM are the particles which have an equivalent circle diameter  $D_{tem}$  within the range of  $\pm 10\%$  of the weight-average particle diameter of the toner determined with a Coulter counter by the procedure described below, where the equivalent circle  
55

diameter  $D_{tem}$  is determined from the cross sections of the toner particles in the TEM image.

A long axis L, which is a maximum diameter of a cross section of a toner particle, is drawn on each toner particle to be measured. Then sixteen straight lines that pass through the midpoint of the long axis L and extend across the cross section are drawn with reference to the long axis L such that the angles between adjacent lines at the intersection at the midpoint are equal (the angle of intersection is 11.25°) (refer to FIG. 1). As a result, thirty-two line segments that extend from the midpoint to the surface of the toner particle are drawn and assumed to be  $A_n$  (n=1 to 32), the length of each line segment is assumed to be  $RA_n$ , and the thickness of the surface layer of the toner particle containing the organic silicon polymer is assumed to be  $FRA_n$ . Then the thicknesses of the toner particle surface layer containing the organic silicon polymer observed on the thirty-two line segments are averaged to determine the average thickness  $Dav$ . Furthermore, the percentage of the surface layer thicknesses  $FRA_n$  that are 5.0 nm or less out of the thirty-two thicknesses is determined.

Equivalent Circle Diameter  $D_{tem}av$ . Determined from Cross Section of Toner in TEM Image

The equivalent circle diameter  $D_{tem}av$  is determined from a cross section of the toner in a TEM image through the following procedure.

First, the equivalent circle diameter  $D_{tem}$  of one toner particle is determined from the following formula from a toner cross section observed in a TEM image.

$$D_{tem} = \frac{(RA_1 + RA_2 + RA_3 + RA_4 + RA_5 + RA_6 + RA_7 + RA_8 + RA_9 + RA_{10} + RA_{11} + RA_{12} + RA_{13} + RA_{14} + RA_{15} + RA_{16} + RA_{17} + RA_{18} + RA_{19} + RA_{20} + RA_{21} + RA_{22} + RA_{23} + RA_{24} + RA_{25} + RA_{26} + RA_{27} + RA_{28} + RA_{29} + RA_{30} + RA_{31} + RA_{22})}{16}$$

This measurement and calculation are conducted on ten toner particles. The observed equivalent circle diameters are averaged and the result is assumed to be the equivalent circle diameter  $D_{tem}av$  determined from cross sections of the toner particles.

Average Thickness  $Dav$  of Surface Layer of Toner Particle

The average thickness  $Dav$  of the toner particle surface layer is determined by the following procedure.

First, the average thickness  $D_{(n)}$  of a surface layer of one toner particle is determined by the following equation:

$$D_{(n)} = \frac{\text{Total of surface layer thicknesses at thirty-two positions on the line segments}}{32}$$

This calculation is conducted on ten toner particles. The resulting average thicknesses  $D_{(n)}$  (n=1 to 10) of the toner particles are averaged in accordance with the equation below to determine the average thickness  $Dav$  of the surface layers of the toner particles.

$$Dav = \frac{(D_{(1)} + D_{(2)} + D_{(3)} + D_{(4)} + D_{(5)} + D_{(6)} + D_{(7)} + D_{(8)} + D_{(9)} + D_{(10)})}{10}$$

Percentage of surface layer thicknesses that are 5.0 nm or less out of thicknesses  $FRA_n$  of the surface layer of the toner particle

The percentage of the surface layer thicknesses that are 5.0 nm or less out of the thicknesses  $FRA_n$  of the surface layer is determined by the following procedure.

First, the percentage of the surface layer having a thickness of 5.0 nm or less is determined by using the equation below for one toner particle.

$$(\text{Percentage of surface layer having a thickness of 5.0 nm or less}) = \frac{(\text{Number of surface layer thicknesses } FRA_n \text{ that are 5.0 nm or less})}{32} \times 100$$

This calculation is conducted on ten toner particles. The obtained results are averaged and the result is assumed to be the percentage of the surface layer thicknesses that are 5.0 nm or less out of the thicknesses  $FRA_n$  of the surface layer of the toner particle.

Concentration (Atomic %) of Silicon Present at Surfaces of Toner Particles

Surface composition analysis is conducted by electron spectroscopy for chemical analysis (ESCA) to determine the carbon concentration dC (atomic %) and the ratio of the silicon concentration (atomic %) to the total (dC+dO+dSi) of the carbon concentration dC, the oxygen concentration dO, and the silicon concentration dSi at the surfaces of the toner particles.

The system used for ESCA and the measurement conditions are as follows.

System used: QUANTUM 2000 produced by ULVAC-PHI Incorporated ESCA measurement conditions: X-ray source: AlK $\alpha$

X-ray: 100  $\mu$ m, 25 W, 15 kV

Raster: 300  $\mu$ m  $\times$  200  $\mu$ m

Pass energy: 58.70 eV

Step size: 0.125 eV

Neutralizing electron gun: 20  $\mu$ A, 1 V

Ar ion gun: 7 mA, 10 V

Number of sweeps: 15 for Si, 10 for C

The observed peak intensities of the respective elements are used to calculate the surface atomic concentrations (atomic %) by using relative sensitivity factors provided by ULVAC-PHI Incorporated.

Method for Measuring Weight-Average Molecular Weight (Mw), Number-Average Molecular Weight (Mn), and Main Peak Molecular Weight (Mp) of Toner and Various Resins

The weight-average molecular weight (Mw), number-average molecular weight (Mn), and main peak molecular weight (Mp) of the toner and various resins are determined by gel permeation chromatography (GPC) under the following conditions.

Measurement Conditions

Columns (produced by Showa Denko K.K.): seven-column combination including Shodex GPC KF-801, KF-802, KF-803, KF-804, KF-805, KF-806, and KF-807 (diameter: 8.0 mm, length: 30 cm)

Eluent: tetrahydrofuran (THF)

Temperature: 40° C.

Flow rate: 0.6 mL/min

Detector: RI

Concentration and amount of sample: 10  $\mu$ l of a 0.1 mass % sample

Sample Preparation

In 20 mL of tetrahydrofuran, 0.04 g of a subject of measurement (toner or resin) is dispersed and dissolved. The resulting mixture is left standing still for 24 hours and filtered with a 0.2  $\mu$ m filter (Pretreatment Disk H-25-2 produced by Tosoh Corporation). The filtrate is used as a sample.

Molecular weight calibration curves prepared from monodisperse polystyrene standard samples are used as the calibration curves. The standard polystyrene samples used for plotting calibration curves are TSK standard polystyrene F-850, F-450, F-288, F-128, F-80, F-40, F-20, F-10, F-4, F-2, F-1, A-5000, A-2500, A-1000, and A-500 produced by Tosoh Corporation. At least ten standard polystyrene samples are to be used.

In determining the GPC molecular weight distribution, the measurement is started from the point where the chromatogram is rising from the baseline on the high-molecular-

weight side and conducted up to a molecular weight of about 400 on the low-molecular-weight side.

Method for Measuring Glass Transition Temperature (Tg) of Toner and Various Resins

The glass transition temperature (Tg) of the toner and various resins is measured with a differential scanning calorimeter (DSC) M-DSC (trade name: Q2000, produced by TA-Instruments) by the following procedure. First, 3 mg of a sample to be measured (toner or resin) is accurately weighed and placed in an aluminum pan. While using an empty aluminum pan as a reference, measurement is conducted in the measurement temperature range of 20° C. to 200° C. at a heating rate of 1° C./min at normal humidity. The measurement is conducted at a modulation amplitude of  $\pm 0.5^\circ$  C. and a frequency of 1/min. The glass transition temperature (Tg: ° C.) is calculated from the obtained reversing heat flow curve. The midpoint of a line connecting the intersections between the tangent line of the endothermic curve and the base lines before and after the endotherm is assumed to be the glass transition temperature Tg (° C.).

The integrated calorific value per gram of the toner (J/g) indicated by the peak area of the endothermic main peak in an endothermic chart during temperature elevation measured by DSC is measured. An example of a reversing flow curve obtained by DSC measurement on the toner is shown in FIG. 3.

The integrated calorific value (J/g) is determined by using the reversing flow curve obtained by the above-mentioned measurement. Analytic software, Universal Analysis 2000 for Windows 2000/XP Version 4.3A (produced by TA Instruments) is used in calculation. The integrated calorific value (J/g) is determined from the region defined by the endothermic curve and a straight line connecting the measurement points at 35° C. and 135° C. by using Integral Peak Linear function.

Method for Measuring Weight-Average Particle Size (D4) and Number-Average Particle Size (D1) of Toner

The weight-average particle size (D4) and the number-average particle size (D1) of the toner are measured by using a precision particle size distribution analyzer equipped with a 100  $\mu\text{m}$  aperture tube based on an aperture resistance method, namely, COULTER COUNTER MULTISIZER 3 (registered trade mark, product of Beckman Coulter Inc.) and bundled special software Beckman Coulter MULTISIZER 3 version 3.51 produced by Beckman Coulter Inc., for setting measurement conditions and analyzing the observed data. The number of effective measurement channels is 25,000. The observed data is analyzed to calculate D4 and D1.

The aqueous electrolytic solution used in the measurement is prepared by dissolving special grade sodium chloride in ion exchange water so that the concentration is about 1 mass %. An example of such a solution is ISOTON II produced by Beckman Coulter Inc.

Before conducting measurement and analysis, the setting of the special software is done as follows: Set the total count of the control mode appearing in a "Change standard operating method (SOM)" window of the bundled software to 50,000 particles. Set the number of runs to 1 and Kd value to a value obtained by using "Standard particles 10.0  $\mu\text{m}$ " produced by Beckman Coulter Inc. Press "Threshold/Noise level measurement button" to automatically set the threshold and the noise level. Set the current to 1600  $\mu\text{A}$ , gain to 2, and electrolyte to ISOTON II. Check the "Flush aperture tube after run" box. In the "Convert Pulse to Size Settings"

window of the bundled software, set the bin spacing to log diameter, size bin to 256 size bin, and size range to 2  $\mu\text{m}$  to 60  $\mu\text{m}$ .

A specific measurement method is as follows:

- 5 (1) Into a 250 mL round-bottomed glass beaker specially prepared for Multisizer 3, about 200 mL of the aqueous electrolytic solution is placed, the beaker is set in the sample stand, and anticlockwise stirring using a stirrer rod is conducted at 24 rotations/second. The contaminants and bubbles inside the aperture tube are preliminarily removed by "aperture flush" function of the software.
- 10 (2) Into a 100 mL flat-bottomed glass beaker, about 30 mL of the aqueous electrolytic solution is placed and about 0.3 mL of a diluted solution of a dispersing agent, "CONTAMINON N" (a 10 mass % aqueous solution of a neutral detergent for washing precision measurement instruments having pH of 7 and containing a nonionic surfactant, an anionic surfactant, and an organic builder, produced by Wako Pure Chemical Industries) diluted about 3 fold with ion exchange water on a mass basis is added thereto.
- 15 (3) A particular quantity of ion exchange water is placed in a water tank of an ultrasonic disperser, ULTRASONIC DISPERSION SYSTEM TETORA 150 produced by Nikkaki Bios Co., Ltd., equipped with two oscillators having an oscillation frequency of 50 kHz with a 180 degree phase shift and an electrical output of 120 W. To the water tank, about 2 mL of CONTAMINON N is added.
- 20 (4) The beaker prepared in (2) is set in a beaker securing hole of the ultrasonic disperser and the ultrasonic disperser is operated. The height position of the beaker is adjusted so that the resonant state of the liquid surface of the aqueous electrolytic solution in the beaker is maximum.
- 25 (5) While applying ultrasonic waves to the electrolyte aqueous solution in the beaker in (4), about 10 mg of the toner is added to the aqueous electrolytic solution in small divided portions to conduct dispersion. The ultrasonic dispersion treatment is continued further for 60 seconds. During the process of ultrasonic dispersion, the water temperature of the water tank is adjusted to be in a range of 10° C. or more and 40° C. or less.
- 30 (6) The ultrasonically dispersed aqueous electrolytic solution containing dispersed toner prepared in (5) is added dropwise using a pipette to the round-bottomed beaker prepared in (1) installed in the sample stand to adjust the measurement concentration to about 5%. Run is repeated until the count of particles reaches 50,000.
- 35 (7) The measurement data is analyzed with special software installed in the instrument to calculate the weight-average particle diameter (D4) and the number-average particle diameter (D1). The weight-average particle diameter (D4) is the number in "Average Diameter" of the "Analysis/volume statistic values (arithmetic mean)" window on Graph/Volume % setting, and the number-average particle diameter (D1) is the number in "Average Diameter" of the "Analysis/number statistic values (arithmetic mean)" window on Graph/Number % setting.
- 40
- 45
- 50
- 55

Method for Measuring Average Circularity and Mode Circularity of Toner

The average circularity of the toner is measured with a dynamic flow particle imaging instrument EPIA-3000 (produced by Sysmex Corporation) under the measurement and analytical conditions used in calibration operation.

To 20 mL of ion exchange water, an appropriate amount of a surfactant, which is preferably an alkyl benzene sulfonic acid salt, is added as a dispersant and then 0.02 g of the measurement sample is added thereto. The resulting mixture is dispersed for 2 minutes in a desktop-type ultrasonic

cleaner disperser (for example, VS-150 produced by Velvo-Clear) at an oscillation frequency of 50 kHz and a power output of 150 W to prepare a dispersion for measurement. During this process, cooling is appropriately conducted so that the temperature of the dispersion is within the range of 10° C. or more and 40° C. or less.

In measurement, the above-mentioned dynamic flow particle imaging instrument equipped with a standard object lens (magnification of 10) is used and particle sheath PSE-900A (produced by Sysmex Corporation) is used as the sheath solution. The dispersion prepared by the above-mentioned procedure is introduced into the dynamic flow particle imaging instrument and 3000 toner particles are measured at a total count mode and HPF measurement mode. The binarization threshold during the particle analysis is set to 85% and the analytic particle diameter is limited to an equivalent circle diameter of 1.98  $\mu\text{m}$  or more and 19.92  $\mu\text{m}$  or less so as to determine the average circularity of the toner.

Prior to measurement, automatic focus adjustment is conducted by using standard latex particles (for example, 5100A produced by Duke Scientific Corporation diluted with ion exchange water). After the start of the measurement, focus adjustment may be performed every two hours.

In the circularity distribution of the toner, a mode circularity of 0.98 to 1.00 means that most of toner particles have a shape close to spherical. At this circularity, the adhesion force of the toner to the photosensitive member attributable to image force and Van der Waals force is significantly decreased and the transfer efficiency is significantly increased.

The circularity is divided into sixty-one circularity classes ranging from a circularity of 0.40 to 1.00 at 0.01 intervals (for example, one class ranges from 0.40 to less than 0.41, the next class ranges from 0.41 to less than 0.42, and the last class ranges from 0.99 to less than 1.00). The observed circularities of the respective particles measured are assigned to corresponding classes and one of these classes where the highest number of particles are allotted in the circularity frequency distribution is assumed to be the mode circularity.

The present invention will be explained further through Examples below which do not limit the scope of the present invention. The number of parts in the description below indicate parts by mass unless otherwise noted.

Production Examples of the charge control resin used in embodiments of the present invention are described.

#### Production Example of Charge Control Resin 1

To a reactor equipped with a reflux duct, a stirrer, a thermometer, a nitrogen duct, a dropper, and a decompressor, 250 parts by mass of methanol, 150 parts by mass of 2-butanone, and 100 parts by mass of 2-propanol were added as solvents and 88 parts by mass of styrene, 6.0 parts by mass of 2-ethylhexyl acrylate, and 6.0 parts by mass of 2-acrylamide-2-methylpropane sulfonic acid were added as monomers. The resulting mixture was heated while being stirred at normal pressure under refluxing. Thereto, a solution prepared by diluting 1.0 part by mass of a polymerization initiator, 2,2'-azobisisobutyronitrile with 20 parts by mass of 2-butanone was added dropwise for 30 minutes and stirring was continued for 5 hours. A solution prepared by diluting 1.0 part by mass of 2,2'-azobisisobutyronitrile with 20 parts by mass of 2-butanone was added thereto dropwise for 30 minutes and stirring was conducted for 5 hours at normal pressure under refluxing to terminate the polymerization.

Next, the polymer obtained by distilling away the polymerization solvents at a reduced pressure was roughly pulverized to 100  $\mu\text{m}$  or less with a cutter mill equipped with a 150 mesh screen and then finely pulverized with a jet mill. The resulting fine particles were classified with a 250 mesh sieve, and particles having a size of 60  $\mu\text{m}$  or under were obtained by the classification. These particles were dissolved in methyl ethyl ketone to a concentration of 10% and the resulting solution was slowly added to methanol in an amount 20 times greater than that of methyl ethyl ketone so as to perform reprecipitation. The precipitates obtained were washed with methanol in an amount half that used for reprecipitation and the filtered particles were vacuum dried at 35° C. for 48 hours.

The particles after vacuum drying was re-dissolved in methyl ethyl ketone to a concentration of 10% and the resulting solution was slowly added to n-hexane in an amount 20 times greater than that of methyl ethyl ketone so as to perform reprecipitation. The precipitates obtained were washed with n-hexane in an amount half that used for reprecipitation and the filtered particles were vacuum dried at 35° C. for 48 hours. The resulting charge control resin had a Tg of about 82° C., a main peak molecular weight (Mp) of 21,500, a number-average molecular weight (Mn) of 13,700, and a weight-average molecular weight (Mw) of 22,800. The acid value was 18.4 mgKOH/g. The obtained resin was named "charge control resin 1".

#### Production Example of Polyester-Based Resin (1)

The following monomers were charged in an autoclave along with an esterification catalyst:

terephthalic acid: 11.0 mol  
bisphenol A-propylene oxide 2 mol adduct (PO-BPA): 10.9 mol

A decompressor, a water separator, a nitrogen gas introducing system, a temperature measurement system, and a stirrer were attached to the autoclave and the reaction was conducted in a nitrogen atmosphere at a reduced pressure according to a normal procedure at 210° C. until Tg was 68° C. As a result, a polyester-based resin (1) was obtained. The weight-average molecular weight (Mw) was 7,400 and the number-average molecular weight (Mn) was 3,020.

#### Production Example of Polyester-Based Resin (2)

##### Synthesis of Isocyanate Group-Containing Prepolymer

The following materials were reacted at 220° C. for 7 hours under stirring:

bisphenol A ethylene oxide 2 mol adduct: 725 parts by mass  
phthalic acid: 290 parts by mass  
dibutyl titanium oxide: 3.0 parts by mass

Then the reaction was continued at a reduced pressure for 5 hours. The resulting product was cooled to 80° C., reacted with 190 parts by mass of isophorone diisocyanate in ethyl acetate for 2 hours. As a result, an isocyanate group-containing polyester resin was obtained. The isocyanate group-containing polyester resin (25 parts by mass) and 1 part by mass of isophorone diamine were reacted at 50° C. for 2 hours. As a result, a polyester-based resin (2) containing a urea group-containing polyester as a main component was obtained. The resulting polyester-based resin (2) had a weight-average molecular weight (Mw) of 22300, a number-average molecular weight (Mn) of 2980, and a peak molecular weight of 7200.

#### Production Example of Toner Particles 1

To a four-necked container equipped with a reflux duct, a stirrer, a thermometer, and a nitrogen duct, 700 parts by mass of ion exchange water, 1000 parts by mass of a 0.1 mol/L  $\text{Na}_3\text{PO}_4$  aqueous solution, and 24.0 parts by mass of a 1.0 mol/L HCl aqueous solution were added. The resulting

mixture was held at 60° C. while being stirred at 12,000 rpm using a high-speed stirrer, TK-Homomixer. To the resulting mixture, 85 parts by mass of a 1.0 mol/L  $\text{CaCl}_2$  aqueous solution was slowly added to prepare an aqueous dispersion medium containing fine, slightly water-soluble dispersion stabilizer  $\text{Ca}_3(\text{PO}_4)_2$ .

The following materials were dispersed for three hours using an attritor to prepare a polymerizable monomer composition 1:

styrene: 70.0 parts by mass  
 n-butyl acrylate: 30.0 parts by mass  
 divinylbenzene: 0.1 parts by mass  
 vinyltriethoxysilane: 15.0 parts by mass  
 copper phthalocyanine pigment (Pigment Blue 15:3 (P.B. 15:3)): 6.5 parts by mass  
 polyester-based resin (1): 4.0 parts by mass  
 charge control agent 1 (aluminum compound of 3,5-di-tert-butyl salicylic acid): 0.5 parts by mass  
 charge control resin 1: 0.5 parts by mass  
 release agent (behenyl behenate, endothermic main peak temperature: 72.1° C.): 10.0 parts by mass

The polymerizable monomer composition 1 was held at 60° C. for 20 minutes. Subsequently, the polymerizable monomer composition 1 and 16.0 parts by mass (50% toluene solution) of t-butyl peroxypivalate serving as a polymerization initiator were placed in an aqueous medium. The resulting mixture was stirred with a high-speed stirrer at a rotation speed of 12,000 rpm for 10 minutes to form particles. The high-speed stirrer was changed to a propeller-type stirrer. The inner temperature was increased to 70° C. and the reaction was performed for 5 hours under slow stirring. The pH of the aqueous medium at this stage was 5.1. Next, 10.0 parts by mass of 1.0 N—NaOH was added to adjust the pH to 8.0. The temperature inside the reactor was increased to 90° C. and held thereat for 7.5 hours. Then 4.0 parts by mass of 10% hydrochloric acid was added to 50 parts by mass of ion exchange water to adjust the pH to 5.1. Then 300 parts by mass of ion exchange water was added, the reflux duct was removed, and a distillator was attached. Distillation was conducted for 5 hours while maintaining the temperature inside the reactor to 100° C., and a polymer slurry 1 was obtained as a result. The amount of the distillate fraction was 300 parts by mass. Diluted hydrochloric acid was added to a reactor containing the polymer slurry 1 after being cooled to 30° C. so as to remove the dispersion stabilizer. Filtration, washing, and drying were performed on the resulting product and toner particles having a weight-average particle size of 5.6  $\mu\text{m}$  were obtained as a result. These toner particles were assumed to be toner particles 1. The formulation and conditions of the toner particles 1 are shown in Table 1 and physical properties thereof are shown in Table 13. Silicon mapping was performed in TEM observation of the toner particles 1 and it was found that silicon atoms were uniformly present in the surface layer. In Examples and Comparative Examples below, silicon mapping was conducted on surface layers that contain the organic silicon polymer.

#### Production Example of Toner Particles 2

Toner particles 2 were obtained as in Production Example of toner particles 1 except that 15.0 parts by mass of allyltriethoxysilane was used instead of 15.0 parts by mass of vinyltriethoxysilane used in Production Example of toner particles 1. The formulation and conditions of the toner particles 2 are shown in Table 1 and the physical properties thereof are shown in Table 13. Silicon mapping was per-

formed in TEM observation of the toner particles 2 and it was found that silicon atoms were uniformly present in the surface layer.

#### Production Example of Toner Particles 3

5 Toner particles 3 were obtained as in Production Example of toner particles 1 except that 15.0 parts by mass of vinyltrimethoxysilane was used instead of 15.0 parts by mass of vinyltriethoxysilane used in Production Example of toner particles 1. The formulation and conditions of the toner particles 3 are shown in Table 1 and the physical properties thereof are shown in Table 13. Silicon mapping was performed in TEM observation of the toner particles 3 and it was found that silicon atoms were uniformly present in the surface layer.

#### 10 Production Example of Toner Particles 4

Toner particles 4 were obtained as in Production Example of toner particles 1 except that 15.0 parts by mass of vinyltrisopropoxysilane was used instead of 15.0 parts by mass of vinyltriethoxysilane used in Production Example of toner particles 1. The formulation and conditions of the toner particles 4 are shown in Table 1 and the physical properties thereof are shown in Table 13. Silicon mapping was performed in TEM observation of the toner particles 4 and it was found that silicon atoms were uniformly present in the surface layer.

#### 15 Production Example of Toner Particles 5

Toner particles 5 were obtained as in Production Example of toner particles 1 except that 15.0 parts by mass of vinyldiethoxylchlorosilane was used instead of 15.0 parts by mass of vinyltriethoxysilane used in Production Example of toner particles 1 and that the pH was adjusted to 5.1 by using 2.0 parts by mass of a 1.0 N—NaOH aqueous solution. The formulation and conditions of the toner particles 5 are shown in Table 1 and the physical properties thereof are shown in Table 13. Silicon mapping was performed in TEM observation of the toner particles 5 and it was found that silicon atoms were uniformly present in the surface layer.

#### 20 Production Example of Toner Particles 6

Toner particles 6 were obtained as in Production Example of toner particles 1 except that 30.0 parts by mass of vinyltriethoxysilane was used instead of 15.0 parts by mass of vinyltriethoxysilane used in Production Example of toner particles 1. The formulation and conditions of the toner particles 6 are shown in Table 1 and the physical properties thereof are shown in Table 13. Silicon mapping was performed in TEM observation of the toner particles 6 and it was found that silicon atoms were uniformly present in the surface layer.

#### 25 Production Example of Toner Particles 7

Toner particles 7 were obtained as in Production Example of toner particles 1 except that 10.5 parts by mass of vinyltriethoxysilane was used instead of 15.0 parts by mass of vinyltriethoxysilane used in Production Example of toner particles 1. The formulation and conditions of the toner particles 7 are shown in Table 1 and the physical properties thereof are shown in Table 13. Silicon mapping was performed in TEM observation of the toner particles 7 and it was found that silicon atoms were uniformly present in the surface layer.

#### 30 Production Example of Toner Particles 8

Toner particles 8 were obtained as in Production Example of toner particles 1 except that 9.5 parts by mass of vinyltriethoxysilane was used instead of 15.0 parts by mass of vinyltriethoxysilane used in Production Example of toner particles 1. The formulation and conditions of the toner particles 8 are shown in Table 2 and the physical properties thereof are shown in Table 14. Silicon mapping was per-

formed in TEM observation of the toner particles 8 and it was found that silicon atoms were uniformly present in the surface layer.

Production Example of Toner Particles 9

Toner particles 9 were obtained as in Production Example of toner particles 1 except that 5.0 parts by mass of vinyltriethoxysilane was used instead of 15.0 parts by mass of vinyltriethoxysilane used in Production Example of toner particles 1. The formulation and conditions of the toner particles 9 are shown in Table 2 and the physical properties thereof are shown in Table 14. Silicon mapping was performed in TEM observation of the toner particles 9 and it was found that silicon atoms were uniformly present in the surface layer.

Production Example of Toner Particles 10

Toner particles 10 were obtained as in Production Example of toner particles 1 except that 4.0 parts by mass of vinyltriethoxysilane was used instead of 15.0 parts by mass of vinyltriethoxysilane used in Production Example of toner particles 1. The formulation and conditions of the toner particles 10 are shown in Table 2 and the physical properties thereof are shown in Table 14. Silicon mapping was performed in TEM observation of the toner particles 10 and it was found that silicon atoms were uniformly present in the surface layer.

Production Example of Toner Particles 11

Toner particles 11 were obtained as in Production Example of toner particles 1 except that the pH was adjusted to 4.1 by adding a solution containing 1.0 part by mass of 10% hydrochloric acid and 50 parts by mass of ion exchange water and that no hydrochloric acid was added upon completion of the reaction 2. The formulation and conditions of the toner particles 11 are shown in Table 2 and the physical properties thereof are shown in Table 14. Silicon mapping was performed in TEM observation of the toner particles 11 and it was found that silicon atoms were uniformly present in the surface layer.

Production Example of Toner Particles 12

Toner particles 12 were obtained as in Production Example of toner particles 1 except that the amount of 1.0 N—NaOH used to adjust the pH to 8.0 in Production Example of toner particles 1 was changed from 10.0 parts by mass to 20.0 parts by mass so as to adjust the pH to 10.2 and hydrochloric acid was added upon completion of the reaction 2 so as to adjust the pH to 5.1. The formulation and conditions of the toner particles 12 are shown in Table 2 and the physical properties thereof are shown in Table 14. Silicon mapping was performed in TEM observation of the toner particles 12 and it was found that silicon atoms were uniformly present in the surface layer.

Production Example of Toner Particles 13

Toner particles 13 were obtained as in Production Example of toner particles 1 except that the amount of 1.0 N—NaOH used to adjust the pH to 8.0 in Production Example of toner particles 1 was changed from 10.0 parts by mass to 15.0 parts by mass so as to adjust the pH to 9.0 and hydrochloric acid was added upon completion of the reaction 2 so as to adjust the pH to 5.1. The formulation and conditions of the toner particles 13 are shown in Table 2 and the physical properties thereof are shown in Table 14. Silicon mapping was performed in TEM observation of the toner particles 13 and it was found that silicon atoms were uniformly present in the surface layer.

Production Example of Toner Particles 14

Toner particles 14 were obtained as in Production Example of toner particles 1 except that 7.5 parts by mass of vinyltriethoxysilane and 7.5 parts by mass of tetraethoxysi-

lane were used instead of 15.0 parts by mass of vinyltriethoxysilane used in Production Example of toner particles 1. The formulation and conditions of the toner particles 14 are shown in Table 2 and the physical properties thereof are shown in Table 14. Silicon mapping was performed in TEM observation of the toner particles 14 and it was found that silicon atoms were uniformly present in the surface layer.

Production Example of Toner Particles 15

Toner particles 15 were obtained as in Production Example of toner particles 1 except that 12.5 parts by mass of vinyltriethoxysilane and 2.5 parts by mass of dimethyl-diethoxysilane were used instead of 15.0 parts by mass of vinyltriethoxysilane used in Production Example of toner particles 1. The formulation and conditions of the toner particles 15 are shown in Table 3 and the physical properties thereof are shown in Table 14. Silicon mapping was performed in TEM observation of the toner particles 15 and it was found that silicon atoms were uniformly present in the surface layer.

Production Example of Toner Particles 16

Toner particles 16 were obtained as in Production Example of toner particles 1 except that the temperature was increased to 95° C. and held thereat for 10 hours instead of increasing the temperature to 90° C. and holding this temperature for 7.5 hours in Production Example of toner particles 1. The formulation and conditions of the toner particles 16 are shown in Table 3 and the physical properties thereof are shown in Table 15. Silicon mapping was performed in TEM observation of the toner particles 16 and it was found that silicon atoms were uniformly present in the surface layer.

Production Example of Toner Particles 17

Toner particles 17 were obtained as in Production Example of toner particles 1 except that the temperature was increased to 100° C. and held thereat for 10 hours instead of increasing the temperature to 90° C. and holding this temperature for 7.5 hours in Production Example of toner particles 1. The formulation and conditions of the toner particles 17 are shown in Table 3 and the physical properties thereof are shown in Table 15. Silicon mapping was performed in TEM observation of the toner particles 17 and it was found that silicon atoms were uniformly present in the surface layer.

Production Example of Toner Particles 18

Preparation of Toner Base Bodies 18

The following materials were mixed in a HENSCHEL MIXER:

- polyester-based resin (1): 60.0 parts by mass
- polyester-based resin (2): 40.0 parts by mass
- 50 copper phthalocyanine pigment (Pigment Blue 15:3): 6.5 parts by mass
- charge control agent 1 (aluminum compound of 3,5-di-tert-butyl salicylic acid): 0.5 parts by mass
- charge control resin 1: 0.5 parts by mass
- 55 release agent (behenyl behenate): 10.0 parts by mass

The resulting mixture was melt kneaded with a two-shaft mixing extruder at 135° C. and the kneaded product was cooled, roughly pulverized with a cutter mill, finely pulverized with a fine grinder that uses jet stream, and classified with an air classifier. As a result, toner base bodies 18 having a weight-average particle size of 5.5  $\mu\text{m}$  were obtained.

Preparation of Toner Particles 18

To a four-necked reactor equipped with a Liebig reflux condenser, 700 parts by mass of ion exchange water, 1000 parts by mass of a 0.1 mol/L  $\text{Na}_3\text{PO}_4$  aqueous solution, and 24.0 parts by mass of a 1.0 mol/L  $\text{HCl}$  aqueous solution were added. The resulting mixture was held at 60° C. while being

stirred at 12,000 rpm using a high-speed stirrer, TK-Homo-mixer. To the resulting mixture, 85 parts by mass of a 1.0 mol/L  $\text{CaCl}_2$  aqueous solution was slowly added to prepare an aqueous dispersion medium containing fine, slightly water-soluble dispersion stabilizer  $\text{Ca}_3(\text{PO}_4)_2$ .

Next, 100.0 parts by mass of the toner base bodies 18 and 15.0 parts by mass of vinyltriethoxysilane were mixed in a HENSCHEL MIXER. The resulting mixture was then stirred in a TK-HOMOMIXER at 5,000 rpm and toner materials were added thereto, followed by stirring for 5 minutes.

The resulting mixture was held at 70° C. for 5 hours. The pH was 5.1. Next, 10.0 parts by mass of 1.0 N— $\text{NaOH}$  was added to adjust the pH to 8.0 and the temperature was increased to 90° C. and held thereat for 7.5 hours. Then 4.0 parts by mass of 10% hydrochloric acid and 50 parts by mass of ion exchange water were added to the mixture to adjust the pH to 5.1. Then 300 parts by mass of ion exchange water was added, the reflux condenser was removed, and a distillator was attached. Distillation was conducted for 5 hours while maintaining the temperature inside the reactor to 100° C. and a polymer slurry 18 was obtained as a result. The amount of the distillation fraction was 320 parts by mass. Diluted hydrochloric acid was added to the reactor containing the polymer slurry 18 to remove the dispersion stabilizer. Then filtration, washing, and drying were conducted and toner particles 18 having a weight-average particle size of 5.6  $\mu\text{m}$  were obtained as a result. The physical properties of the toner particles are shown in Table 15. Silicon mapping was performed in TEM observation of the toner particles 18 and it was found that silicon atoms were uniformly present in the surface layer.

#### Production Example of Toner Particles 19

The following materials were dissolved in 400 parts by mass of toluene to obtain a solution:  
 polyester-based resin (1): 60.0 parts by mass  
 polyester-based resin (2): 40.0 parts by mass  
 copper phthalocyanine pigment (Pigment Blue 15:3): 6.5 parts by mass  
 charge control agent 1 (aluminum compound of 3,5-di-*tert*-butyl salicylic acid): 0.5 parts by mass  
 charge control resin 1: 0.5 parts by mass  
 vinyltriethoxysilane: 15.0 parts by mass  
 release agent (behenyl behenate): 10.0 parts by mass

To a four-necked reactor equipped with a Liebig reflux condenser, 700 parts by mass of ion exchange water, 1000 parts by mass of a 0.1 mol/L  $\text{Na}_3\text{PO}_4$  aqueous solution, and 24.0 parts by mass of a 1.0 mol/L  $\text{HCl}$  aqueous solution were added. The resulting mixture was held at 60° C. while being stirred at 12,000 rpm using a high-speed stirrer, TK-Homo-mixer. To the resulting mixture, 85 parts by mass of a 1.0 mol/L  $\text{CaCl}_2$  aqueous solution was slowly added to prepare an aqueous dispersion medium containing fine, slightly water-soluble dispersion stabilizer  $\text{Ca}_3(\text{PO}_4)_2$ .

Next, 100.0 parts by mass of the solution was added to the mixture by using a TK-Homomixer under stirring at 12,000 rpm. The stirring was conducted for 5 minutes after the addition. The resulting mixture was held at 70° C. for 5 hours. The pH was 5.1. Then 10.0 parts by mass of 1.0 N— $\text{NaOH}$  was added to adjust the pH to 8.0 and the temperature was increased to 90° C. and held thereat for 7.5 hours. Then 4.0 parts by mass of 10% hydrochloric acid and 50 parts by mass of ion exchange water were added to the mixture to adjust the pH to 5.1. Then 300 parts by mass of ion exchange water was added, the reflux condenser was removed, and a distillator was attached. Distillation was conducted for 5 hours while maintaining the temperature

inside the reactor to 100° C. and a polymer slurry 20 was obtained as a result. The amount of the distillation fraction was 320 parts by mass. Diluted hydrochloric acid was added to the reactor containing the polymer slurry 20 to remove the dispersion stabilizer. Then filtration, washing, and drying were conducted and toner particles 19 having a weight-average particle size of 5.6  $\mu\text{m}$  were obtained as a result. The physical properties of the toner particles 19 are shown in Table 15. Silicon mapping was performed in TEM observation of the toner particles 19 and it was found that silicon atoms were uniformly present in the surface layer.

#### Production Example of Toner Particles 20

##### Synthesis of Amorphous Polyester Resin (1)

The following monomers were charged in a flask equipped with a stirrer, a nitrogen duct, a temperature sensor, and a rectifier:

bisphenol A ethylene oxide 2 mol adduct: 10 mol %  
 bisphenol A propylene oxide 2 mol adduct: 94 mol %  
 terephthalic acid: 50 mol %  
 fumaric acid: 30 mol %  
 dodecenylsuccinic acid: 25 mol %

The resulting mixture was heated to 195° C. in one hour and it was confirmed that the reaction system was being stirred uniformly.

Next, 0.8 weight % of tin distearate relative to the total weight of the monomers was added to the resulting mixture. The temperature was increased from 195° C. to 250° C. in 5 hours while distilling away water produced and dehydration condensation reaction was performed at 250° C. for 2 hours. As a result, an amorphous polyester resin (1) having a glass transition temperature of 59.8° C., an acid value of 14.1 mgKOH/g, a hydroxy value of 26.2 mgKOH/g, a weight-average molecular weight of 15,700, a number-average molecular weight of 4,500, and a softening point of 114° C. was obtained.

##### Synthesis of Amorphous Polyester Resin (2)

The following monomers were placed in a flask equipped with a stirrer, a nitrogen duct, a temperature sensor, and a rectifier:

bisphenol A ethylene oxide 2 mol adduct: 50 mol % (2 mol adduct on a dual end basis)  
 bisphenol A propylene oxide 2 mol adduct: 50 mol % (2 mol adduct on a dual end basis)  
 terephthalic acid: 65 mol %  
 dodecenylsuccinic acid: 30 mol %

The resulting mixture was heated to 195° C. in one hour and it was confirmed that the reaction system was being uniformly stirred.

Next, 0.7 weight % of tin distearate relative to the total weight of the monomers was added to the resulting mixture. The temperature was increased from 195° C. to 240° C. in 5 hours while distilling away water produced and dehydration condensation reaction was performed at 240° C. for 2 hours. Then the temperature was decreased to 190° C., 6 mol % of trimellitic anhydride was slowly added to the mixture, and the reaction was continued at 190° C. for one hour. As a result, an amorphous polyester resin (2) having a glass transition temperature of 54.0° C., an acid value of 12.0 mgKOH/g, a hydroxy value of 25.1 mgKOH/g, a weight-average molecular weight of 51,200, a number-average molecular weight of 6,100, and a softening point of 110° C. was obtained.

##### Preparation of Resin Particle Dispersion (1)

In a reactor, 50 parts by mass of methyl ethyl ketone and 20 parts by mass of isopropyl alcohol were placed. Thereto, 100 parts by mass of the amorphous polyester resin (1) was

slowly added and completely dissolved under stirring. As a result, an amorphous polyester resin (1) solution was obtained.

The reactor containing the amorphous polyester resin (1) solution was set to 65° C. and a total of 5 parts by mass of a 10% ammonia aqueous solution was slowly added dropwise thereto under stirring. Then 230 parts by mass of ion exchange water was slowly added dropwise at a rate of 10 mL/min to perform phase-transfer emulsification. The pressure was reduced by using an evaporator to remove the solvent. As a result, a resin particle dispersion (1) of the amorphous polyester resin (1) was obtained. The volume-average particle size of the resin particles was 140 nm. The resin particle solid content was adjusted by ion exchange water to 20%.

#### Preparation of Resin Particle Dispersion (2)

In a reactor, 50 parts by mass of methyl ethyl ketone and 20 parts by mass of isopropyl alcohol were placed. Thereto, 100 parts by mass of the amorphous polyester resin (2) was slowly added and completely dissolved under stirring. As a result, an amorphous polyester resin (2) solution was obtained.

The reactor containing the amorphous polyester resin (2) solution was set to 40° C. and a total of 3.5 parts by mass of a 10% ammonia aqueous solution was slowly added dropwise thereto under stirring. Then 230 parts by mass of ion exchange water was slowly added dropwise at a rate of 10 mL/min to perform phase-transfer emulsification. The pressure was reduced to remove the solvent. As a result, a resin particle dispersion (2) of the amorphous polyester resin (2) was obtained. The volume-average particle size of the resin particles was 160 nm. The resin particle solid content was adjusted by ion exchange water to 20%.

#### Preparation of Sol-Gel Solution of Resin Particle Dispersion (1)

To 100 parts by mass (solid content: 20.0 parts by mass) of the resin particle dispersion (1), 20.0 parts by mass of vinyltriethoxysilane was added and the resulting mixture was stirred. The temperature was held at 70° C. for one hour, then increased to 80° C. at a heating rate of 20° C./hour, and held thereat for 3 hours. The mixture was cooled and a sol-gel solution of the resin particle dispersion (1) in which the resin fine particles were coated with sol/gel was obtained as a result. The volume-average particle size of the resin particles was 220 nm. The resin particle solid content was adjusted with ion exchange water to 20%. The sol-gel solution of the resin particle dispersion (1) was stored at a temperature of 10° C. or lower while being stirred and used within 48 hours after preparation. The surfaces of the particles may be in a highly viscous sol or gel state since the adhesion between the particles is improved.

#### Preparation of Colorant Particle Dispersion 1

The following components were mixed to prepare a mixture:

copper phthalocyanine (Pigment Blue 15:3): 45 parts by mass

ionic surfactant NEOGEN RK (produced by Dai-Ichi Kogyo Seiyaku Co., Ltd.): 5 parts by mass

ion exchange water: 190 parts by mass

The mixture was dispersed in a homogenizer (IKA ULTRA TURRAX) for 10 minutes and dispersed at 250 MPa with ULTIMIZER (collision-type wet atomizer produced by Sugino Machine Limited) for 20 minutes. As a result, a colorant particle dispersion 1 having a colorant particle volume-average particle size of 130 nm and a solid content of 20% was obtained.

#### Preparation of Release Agent Particle Dispersion

The following materials were mixed and heated to 100° C.:

olefin wax (melting point: 84° C.): 60 parts by mass  
ionic surfactant NEOGEN RK (produced by Dai-Ichi Kogyo Seiyaku Co., Ltd.): 2.0 parts by mass  
ion exchange water: 240 parts by mass

The mixture was then thoroughly dispersed in ULTRA TURRAX T50 produced by IKA, and heated to 115° C. and dispersed for 1 hour by using a pressure extrusion type Gaulin homogenizer. As a result, a release agent particle dispersion having a volume-average particle size of 160 nm and a solid content of 20% was obtained.

#### Preparation of Toner Particles 25

In a flask, 2.2 parts by mass of an ionic surfactant, NEOGEN RK was placed and then the following materials were added thereto:

resin particle dispersion (1): 100 parts by mass  
resin particle dispersion (2): 300 parts by mass  
sol-gel solution of resin particle dispersion (1): 300 parts by mass  
colorant particle dispersion 1: 50 parts by mass  
release agent particle dispersion: 50 parts by mass

The resulting mixture was stirred. Then a 1 N nitric acid aqueous solution was added to the mixture to adjust the pH to 3.7, 0.35 parts by mass of polyaluminum sulfate was added thereto, and the resulting mixture was dispersed by using ULTRA TURRAX. The flask was heated to 50° C. under stirring in a heating oil bath and held at 50° C. for 40 minutes. Then 300 parts by mass of the sol-gel solution of the resin particle dispersion (1) was slowly added thereto.

Next, a 1 N sodium hydroxide aqueous solution was added to adjust the pH in the system to 7.0. The stainless steel flask was hermetically sealed, slowly heated to 90° C. under stirring, and retained at 90° C. for 5 hours and then at 95° C. for 7.5 hours. Then 2.0 parts by mass of an ionic surfactant, NEOGEN RK was added and reaction was conducted at 100° C. for 5 hours. After completion of the reaction, distillation was conducted at a reduced pressure at 85° C. and 320 parts by mass of a fraction was recovered. The fraction was cooled, filtered, dried, and re-dispersed in 5 L of ion exchange water at 40° C. The resulting dispersion was stirred for 15 minutes with a stirring blade (300 rpm) and filtered.

The re-dispersion and filtration were repeated to conduct washing and washing was ended when the electrical conductivity reached 6.0  $\mu$ S/cm or lower. As a result, toner particles 20 were obtained. The physical properties of the toner particles 20 are shown in Table 15. Silicon mapping was performed in TEM observation of the toner particles 20 and it was found that silicon atoms were uniformly present in the surface layer.

#### Production Example of Toner Particles 21

In a HENSCHEL MIXER, while 100.0 parts by mass of toner base bodies 19 were being stirred at high speed, 3.5 parts by mass of an organic silicon polymer solution prepared by reacting 10.0 parts by mass of toluene, 5.0 parts by mass of ethanol, 5.0 parts by mass of water, and 15.0 parts by mass of vinyltriethoxysilane at 90° C. for 5 hours was sprayed toward the toner base bodies 19 to conduct uniform mixing.

Then the particles were circulated within a fluid-bed drier for 30 minutes at an inlet temperature of 90° C. and an outlet temperature of 45° C. to conduct drying and polymerization.

The obtained processed toner was placed in a HENSCHEL MIXER and 3.5 parts by mass of the organic silicon polymer solution described above per 100 parts by mass of the

processed toner was sprayed toward the processed toner. The processed toner was then circulated in a fluid-bed drier for 30 minutes at an inlet temperature of 90° C. and an outlet temperature of 45° C.

Spraying of the organic silicon polymer solution and drying were repeated a total of ten times to obtain toner particles 21. The physical properties of the toner particles 21 are shown in Table 15. Silicon mapping was performed in TEM observation of the toner particles 21 and it was found that silicon atoms were uniformly present in the surface layer.

#### Production Example of Toner Particle 22

Toner particles 22 were obtained as in Production Example of toner particles 1 except that 10.0 parts by mass of carbon black is used instead of 6.5 parts by mass of copper phthalocyanine in Production Example of toner particles 1. The formulation and conditions of the toner particles 22 are shown in Table 4 and the physical properties thereof are shown in Table 15. Silicon mapping was performed in TEM observation of the toner particles 3 and it was found that silicon atoms were uniformly present in the surface layer.

#### Production Example of Toner Particle 23

Toner particles 23 were obtained as in Production Example of toner particles 1 except that the amount of styrene used was changed from 70.0 parts by mass in Production Example of toner particles 1 to 60.0 parts by mass and the amount of n-butyl acrylate used was changed from 30.0 parts by mass in Production Example of toner particles 1 to 40.0 parts by mass, and that 1.0 part by mass of titanium tetra-n-butoxide was added. The formulation and conditions of the toner particles 23 are shown in Table 4 and the physical properties thereof are shown in Table 16. Silicon mapping was performed in TEM observation of the toner particles 23 and it was found that silicon atoms were uniformly present in the surface layer.

#### Production Example of Toner Particles 24

Toner particles 24 were obtained as in Production Example of toner particles 1 except that 8.0 parts by mass of Pigment Red 122 (P.R. 122) was used instead of 6.5 parts by mass of copper phthalocyanine (Pigment Blue 15:3) used in Production Example of toner particles 1. The formulation and conditions of the toner particles 24 are shown in Table 4 and the physical properties thereof are shown in Table 16. Silicon mapping was performed in TEM observation of the toner particles 24 and it was found that silicon atoms were uniformly present in the surface layer.

#### Production Example of Toner Particles 25

Toner particles 25 were obtained as in Production Example of toner particles 1 except that 6.0 parts by mass of Pigment Yellow 155 (P.Y. 155) was used instead of 6.5 parts by mass of copper phthalocyanine (Pigment Blue 15:3) used in Production Example of toner particles 1. The formulation and conditions of the toner particles 25 are shown in Table 4 and the physical properties thereof are shown in Table 16. Silicon mapping was performed in TEM observation of the toner particles 25 and it was found that silicon atoms were uniformly present in the surface layer.

#### Production Example of Toner Particles 26

Toner articles 26 were obtained as in Production Example of toner particles 1 except that 29.0 parts by mass of n-butyl methacrylate was used instead of 30.0 parts by mass of n-butyl acrylate used in Production Example 1, the amount of divinylbenzene was changed from 0.1 parts by mass to 0.0 parts by mass, and 1.0 part by mass of an acrylate was added. The formulation and conditions of the toner particles 26 are shown in Table 4 and the physical properties thereof are

shown in Table 16. Silicon mapping was performed in TEM observation of the toner particles 26 and it was found that silicon atoms were uniformly present in the surface layer. Production Example of Toner Particles 27

Toner particles 27 were obtained as in Production Example of toner particles 1 except that the amount of n-butyl acrylate used was changed from 30.0 parts by mass in Production Example of toner particles 1 to 20.0 parts by mass and that 10.0 parts by mass of behenyl acrylate was added. The formulation and conditions of the toner particles 27 are shown in Table 4 and the physical properties thereof are shown in Table 16. Silicon mapping was performed in TEM observation of the toner particles 27 and it was found that silicon atoms were uniformly present in the surface layer.

#### Production Example of Comparative Toner Particles 1

Comparative toner particles 1 were obtained as in Production Example of toner particles 1 except that 2.0 parts by mass of vinyltriethoxysilane was used instead of 15.0 parts by mass of vinyltriethoxysilane used in Production Example of toner particles 1. The formulation and conditions of the comparative toner particles 1 are shown in Table 5 and the physical properties thereof are shown in Table 17. Silicon mapping was performed in TEM observation of the comparative toner particles 1 and it was found that few silicon atoms are present in the surface layer.

#### Production Example of Comparative Toner Particles 2

Comparative toner particles 2 were obtained as in Production Example of comparative toner particles 1 except that 15.0 parts by mass of tetraethoxysilane was used instead of 2.0 parts by mass of vinyltriethoxysilane used in Production Example of comparative toner particles 1. The formulation and conditions of the comparative toner particles 2 are shown in Table 5 and the physical properties thereof are shown in Table 17. Silicon mapping was performed in TEM observation of the comparative toner particles 2 and it was found that silicon atoms are non-uniformly present in the surface layer.

#### Production Example of Comparative Toner Particles 3

Comparative toner particles 3 were obtained as in Production Example of comparative toner particles 1 except that 15.0 parts by mass of 3-methacryloxypropyltriethoxysilane was used instead of 2.0 parts by mass of vinyltriethoxysilane used in Production Example of comparative toner particles 1. The formulation and conditions of the comparative toner particles 3 are shown in Table 5 and the physical properties thereof are shown in Table 17. Silicon mapping was performed in TEM observation of the comparative toner particles 3 and it was found that few silicon atoms are present in the surface layer.

#### Production Example of Comparative Toner Particles 4

Comparative toner particles 4 were prepared as in Production Example of comparative toner particles 1 except that 15.0 parts by mass of 3-methacryloxypropyltriethoxysilane was used instead of 2.0 parts by mass of vinyltriethoxysilane used in Production Example of comparative toner particles 1, that the reactor was heated to 70° C. and held thereat for 10.0 hours instead of being heated to 90° C. and held thereat for 7.5 hours in Production Example of comparative toner particles 1, and the reaction 3 was not performed. The formulation and conditions of the comparative toner particles 4 are shown in Table 5 and the physical properties thereof are shown in Table 17. Silicon mapping was performed in TEM observation of the comparative toner particles 4 and it was found that few silicon atoms were present in the surface layers.

## Production Example of Comparative Toner Particles 5

Comparative toner particles 5 were prepared as in Production Example of comparative toner particle 1 except that 15.0 parts by mass of 3-methacryloxypropyltriethoxysilane was used instead of 2.0 parts by mass of vinyltriethoxysilane used in Production Example of comparative toner particles 1, the inner temperature was increased to 80° C. instead of 70° C., the reactor was heated to 80° C. and held thereof for 10 hours instead being heated to 90° C. and held thereof for 7.5 hours, and the reaction 3 was not performed. The formulation and conditions of the comparative toner particles 5 are shown in Table 5 and the physical properties thereof are shown in Table 17. Silicon mapping was performed in TEM observation of the comparative toner particles 5 and it was found that few silicon atoms were present in the surface layers.

## Production Example of Comparative Toner Particles 6

Comparative toner particles 6 were obtained as in Production Example of comparative toner particles 1 except that 3.1 parts by mass of 3-methacryloxypropyltriethoxysilane was used instead of 2.0 parts by mass of vinyltriethoxysilane used in Production Example of comparative toner particles 1. The formulation and conditions of the comparative toner particles 6 are shown in Table 6 and the physical properties thereof are shown in Table 18. Silicon mapping was performed in TEM observation of the comparative toner particles 6 and it was found that few silicon atoms were present in the surface layers.

## Production Example of Comparative Toner Particles 7

Comparative toner particles 7 were obtained as in Production Example of comparative toner particles 1 except that 3.0 parts by mass of vinyltriethoxysilane was used instead of 2.0 parts by mass of vinyltriethoxysilane used in Production Example of comparative toner particles 1. The formulation and conditions of the comparative toner particles 7 are shown in Table 6 and the physical properties thereof are shown in Table 18. Silicon mapping was performed in TEM observation of the comparative toner particles 7 and it was found that few silicon atoms were present in the surface layers.

## Production Example of Comparative Toner Particles 8

Comparative toner particles 8 were obtained as in Production Example of comparative toner 4 except that 3.0 parts by mass of vinyltriethoxysilane was used instead of 15.0 parts by mass of 3-methacryloxypropyltriethoxysilane used in Production Example of comparative toner particles 4. The formulation and conditions of the comparative toner particles 8 are shown in Table 6 and the physical properties thereof are shown in Table 18. Silicon mapping was performed in TEM observation of the comparative toner particles 8 and it was found that few silicon atoms were present in the surface layers.

## Production Example of Comparative Toner Particles 9

Comparative toner particles 9 were obtained as in Production Example of comparative toner 1 except that 11.0 parts by mass of aminopropyltrimethoxysilane was used instead of 2.0 parts by mass of vinyltriethoxysilane used in Production Example of comparative toner particles 1. The formulation and conditions of the comparative toner particles 9 are shown in Table 6 and the physical properties thereof are shown in Table 18. Silicon mapping was performed in TEM observation of the comparative toner particles 9 and it was found that few silicon atoms were present in the surface layers.

## Production Example of Comparative Toner Particles 10

Comparative toner particles 10 were obtained as in Production Example of comparative toner 1 except that the

amount of vinyltriethoxysilane used was changed from 2.0 parts by mass used in Production Example of comparative toner particle 1 to 0.0 parts by mass. The formulation and conditions of the comparative toner particles 10 are shown in Table 6 and the physical properties thereof are shown in Table 18. Silicon mapping was performed in TEM observation of the comparative toner particles 10 and it was found that no silicon atoms were present in the surface layers.

## Production Example of Comparative Toner Particles 11

10 To a four-necked flask equipped with a high-speed stirrer, TK-Homomixer, 900 parts by mass of ion exchange water and 95 parts by mass of polyvinyl alcohol were added. The resulting mixture was heated to 55° C. while being stirred at a rotation rate of 1300 rpm so as to prepare an aqueous dispersion medium.

## Composition of Monomer Dispersion

The following materials were dispersed in an attritor for three hours:

styrene: 70.0 parts by mass  
20 n-butyl acrylate: 30.0 parts by mass  
carbon black: 10.0 parts by mass  
salicylic acid silane compound: 1.0 part by mass  
release agent ( behenyl behenate): 10.0 parts by mass

25 To the resulting mixture, 14.0 parts by mass of a polymerization initiator, t-butyl peroxy pivalate was added to prepare a monomer dispersion.

The monomer dispersion was placed in the dispersion medium in the four-necked flask described above and particles were formed while maintaining the above-described 30 rotation rate for 10 minutes. Then polymerization was performed at 55° C. for 1 hour and then at 65° C. for 4 hours, and then at 80° C. for 5 hours under stirring at 50 rpm. After completion of the polymerization described above, the slurry was cooled and washed with purified water repeatedly 35 to remove the dispersant. Washing and drying were performed to obtain black toner particles that serve as base bodies. The weight-average particle size of the black toner particles was 5.70  $\mu\text{m}$ .

To a solution containing 2 parts by mass of isoamyl 40 acetate and silicon compounds, namely, 3.5 parts by mass of tetraethoxysilane and 0.5 parts by mass of methyltriethoxysilane, 3 parts by mass of a 0.3 mass % sodium dodecylbenzenesulfonate solution were added. The resulting mixture was stirred with an ultrasonic homogenizer to prepare a 45 mixed solution A containing isoamyl acetate, tetraethoxysilane, and methyltriethoxysilane.

To 30 parts by mass of a 0.3 mass % sodium dodecylbenzenesulfonate aqueous solution, 1.0 part by mass of the 50 black toner particles serving as base bodies and the mixed solution A were added. To the resulting solution, 5 parts by mass of a 29 mass %  $\text{NH}_4\text{OH}$  aqueous solution was added and stirring was performed at room temperature (25° C.) for 12 hours. The resulting product was washed with ethanol and then with purified water and particles were filtered and dried. As a result, comparative toner particles 11 were obtained. The weight-average particle size of the toner particles were 5.6  $\mu\text{m}$ . The physical properties of the comparative toner particles 11 are shown in Table 18. Silicon mapping was performed in TEM observation of the comparative toner particles 11 and it was found that few silicon atoms are present in the surface layers.

## Production Example of Toner 1

In a HENSCHEL MIXER (produced by Mitsui Mining Co., Ltd.), 100 parts by mass of the toner particles 1, 0.4 55 parts by mass of hydrophobic silica having a BET specific surface area of 200  $\text{m}^2/\text{g}$  and surfaces treated with 4.0 mass % of hexamethyldisilazane and 3 mass % of 100 cps silicone

oil, and 0.2 parts by mass of aluminum oxide having a BET specific surface area of 50 m<sup>2</sup>/g were mixed to prepare a toner. This toner was used as a toner 1. The physical properties of the toner 1 are shown in Table 7.

Production Examples of Toners 2 to 27

Toners 2 to 27 were obtained as in Production Example of toner 1 except that the toner particles 1 used in Production Example of toner 1 were changed to toner particles 2 to 27. The physical properties of the toners 2 to 27 are shown in Tables 7 to 10.

Production Examples of Comparative Toners 1 to 11

Comparative toners 1 to 11 were obtained as in Production Example of toner 1 except that the toner particles 1 used in Production Example of toner 1 were changed to the comparative toner particles 1 to 11. The physical properties of the comparative toners 1 to 11 are shown in Tables 11 and 12.

Evaluation of Physical Properties of Toners 1 to 27 and Comparative Toners 1 to 11 after Washing

A mixed solution of 1.0 part by mass of the toner 1, 100 parts by mass of ion exchange water, and 0.01 parts by mass of sodium dodecylbenzenesulfonate was ultrasonically dispersed for 5 minutes to conduct centrifugal separation. The upper 20% fraction of the filtrate was sampled. The filtrate was dried and the physical properties of the toner 1 after washing were measured. The physical properties of the toner 1 were the same as those before washing (Table 7).

The same operation was performed on the toners 2 to 27 and the comparative toners 1 to 11 and physical properties of the washed toners were measured. The same physical properties were exhibited as those before washing for all of the toners 2 to 27 and the comparative toners 1 to 11.

Example 1

The following evaluations were performed on the toner 1. The evaluation results are shown in Table 19.

Evaluation of Environmental Stability and Development Durability

Toner cartridges of a tandem-type laser beam printer LBP9600C produced by Canon Kabushiki Kaisha having a structure illustrated in FIG. 4 were each loaded with 240 g of the toner 1. As shown in FIG. 4, the printer included a photosensitive member 1 to which a laser beam 7 is applied, a developing roller 2, a toner supplying roller 3, a toner 4, a regulating blade 5, a developing device 6, a charging device 8, a cleaning device 9, a charging device 10 for cleaning, a stirring blade 11, a drive roller 12, a transfer roller 13, a bias power supply 14, a tension roller 15, a transfer conveying belt 16, a driven roller 17, a feed roller 19 that feeds a paper sheet 18, an attraction roller 20, and a fixing device 21.

The toner cartridges for the printer were respectively left in a low temperature, low humidity environment (10° C./15% RH) (hereinafter may be referred to as "LL"), a normal temperature, normal humidity (25° C./50% RH) environment (hereinafter may be referred to as "NN"), and a high temperature, high humidity environment (32.5° C./85% RH) (hereinafter may be referred to as "HH") for 24 hours. Each toner cartridge after being left in the corresponding environment for 24 hours was attached to LBP9600C and an initial solid image (toner coverage: 0.40 mg/cm<sup>2</sup>) was printed. Then an image with a 1.0% printing rate was printed on 15,000 sheets of A4-size paper in a sheet

transverse direction. After 15,000 sheets were printed out, a solid image was again output. The density of the solid image and extent of fogging before and after 15,000 sheets of printouts were made and soiling of parts after 15,000 sheets of printouts were made were evaluated.

Another toner cartridge was loaded with 240 g of the toner 1. The toner cartridge was left in a severe environment (40° C./90%) for 168 hours and then in a super high temperature, high humidity (35.0° C./85% RH) environment (hereinafter may be referred to as "SHH") for 24 hours. The toner cartridge after being left in the super high temperature, high humidity environment for 24 hours was attached to LBP9600C and an initial solid image was printed. Then an image with a 1.0% printing rate was printed on 15,000 sheets of paper. After 15,000 sheets were printed out, a solid image was again output. The density of the solid image and extent of fogging before and after 15,000 sheets of printouts were made and soiling of parts after 15,000 sheets of printouts were made were evaluated. A4-size paper having a weight of 70 g/m<sup>2</sup> was used as the transfer paper and printing was conducted in a transverse direction of A4-size paper.

Evaluation of Image Density

A Macbeth densitometer (RD-914 produced by Macbeth) equipped with an SPI auxiliary filter was used to measure the image density of a fixed image portion of the initial solid image and the solid image after 15,000 sheets of printouts. The evaluation standard of the image density was as follows:

- 35 A: 1.45 or more
- B: 1.40 or more and less than 1.45
- C: 1.35 or more and less than 1.40
- D: 1.30 or more and less than 1.35
- E: 1.20 or more and less than 1.30
- 40 F: less than 1.20

Evaluation of Fogging

The whiteness degree of background portions of an initial image with 0% printing rate and an image with 0% printing rate after 15,000 sheets of printouts were made was measured with a reflectometer (produced by Tokyo Denshoku Co., Ltd.). The observed values were compared with the whiteness degree of the transfer paper so as calculate the difference and the fogging density (%) was determined from the difference. Fogging was evaluated from the results of the fogging density based on the following standard:

- A: less than 1.0%
- B: 1.0% or more and less than 1.5%
- C: 1.5% or more and less than 2.0%
- D: 2.0% or more and less than 2.5%
- E: 2.5% or more and less than 3.0%
- F: 3.0% or more

Evaluation of Soiling of Parts

After 15,000 sheets of printouts were made, an image in which the upper half portion was a halftone image (toner coverage: 0.25 mg/cm<sup>2</sup>) and the lower half portion was a solid image (toner coverage: 0.40 mg/cm<sup>2</sup>) was printed out and evaluated according to the following standard.

- 60 A: Vertical streaks that extend in the sheet feeding direction are found on none of the developing roller, the halftone image portion, and the solid image portion.

45

B: One or two fine streaks extending in a circumferential direction are found on two ends of the developing roller, but vertical streaks that extend in the sheet feeding direction are found on none of the halftone image portion and the solid image portion.

C: Three to five fine streaks extending in a circumferential direction are found on two ends of the developing roller and few vertical streaks that extend in the sheet feeding direction are found on the halftone image portion and the solid image portion. However, these streaks can be erased by image processing.

D: Six to twenty fine streaks extending in a circumferential direction are found on two ends of the developing roller and several fine streaks are also found on the halftone image portion and the solid image portion. These streaks cannot be erased by image processing.

E: Twenty-one or more streaks are found on the developing roller and the halftone image portion and these streaks cannot be erased by image processing.

#### Measurement of Triboelectric Charge Amount of the Toner

The triboelectric charge amount of the toner was determined by the following method. First, a toner and a standard carrier for a negatively chargeable toner (trade name: N-01 produced by The Imaging Society of Japan) were left in the following environments for particular lengths of time.

(1) In a low temperature, low humidity environment (10° C./15% RH), a normal temperature, normal humidity environment (25° C./50% RH), or a high temperature, high humidity environment (32.5° C./85% RH), the toner and the standard carrier were left standing for 24 hours.

(2) In a severe environment (40° C./90% RH), the toner and the standard carrier were left there for 168 hours and then in a super high temperature, high humidity environment (35.0° C./85% RH) for 24 hours.

The toner and the standard carrier after being left in the above-described environment were mixed with each other by using a turbula mixer for 120 seconds in the same environment so that the toner content is 5 mass %. As a result, a two-component developer was obtained. Within one minute after completion of mixing of the two-component developer, the two-component developer was placed in a metal container having a bottom equipped with a conductive screen having an aperture of 20  $\mu\text{m}$  in a normal temperature, normal humidity (25° C./50% RH) environment. The container was suctioned with a suction machine. The difference in mass between before and after suction and the potential accumulated in a capacitor connected to the container was measured. The suction pressure was 4.0 kPa. The triboelectric charge amount of the toner was calculated by using the following equation based on the difference in mass between before and after suction, the potential accumulated, and the capacity of the capacitor.

The standard carrier for a negatively chargeable toner used for measurement (trade name: N-01 produced by The Imaging Society of Japan) was screened with a 250 mesh in advance and the undersize was used.

$$Q = (A \times B) / (W1 - W2)$$

46

Q (C/kg): triboelectric charge amount of charge control resin and toner

A ( $\mu\text{F}$ ): capacity of capacitor

B (V): potential difference accumulated in capacitor

W1-W2 (g): difference in mass between before and after suction

Evaluation of Low-Temperature Fixability (Low-Temperature Offset End Temperature)

The fixing unit of the laser beam printer LBP9600C produced by Canon Kabushiki Kaisha was modified so that the fixing temperature could be adjusted. The modified LBP9600C was used to heat-press an unfixed toner image having a toner coverage of 0.4 mg/cm<sup>2</sup> to an image-receiving sheet in an oil-less manner at a process speed of 230 mm/sec so as to form a fixed image on the image-receiving sheet.

The fixability was evaluated in terms of low-temperature offset end temperature at which the rate of decrease in density between before and after ten times of rubbing of a fixed image with Kimwipes (S-200 produced by NIPPON PAPER CRECIA Co., LTD.) under a 75 g/cm<sup>2</sup> load was less than 5%. Evaluation was conducted at normal temperature and normal humidity (25° C./50% RH).

#### Evaluation of Storage Stability

#### Evaluation of Storage Property

In a 100 ml glass jar, 10 g of a toner was placed and left at 55° C. and a humidity of 20% for 15 days. The toner was then observed with naked eye.

A: No changes were observed.

B: Some aggregates were observed but they were loose.

C: Aggregates that were not loose were observed.

D: No fluidity was observed.

E: Clear caking occurred.

#### Evaluation of Long-Term Storage Property

In a 100 ml glass jar, 10 g of a toner was placed and left at 45° C. and a humidity of 95% for three months. The toner was then observed with naked eye.

A: No changes were observed.

B: Some aggregates were observed but they were loose.

C: Aggregates that were not loose were found.

D: No fluidity was observed.

E: Clear caking occurred.

#### Examples 2 to 27

The same evaluation as that in Example 1 was conducted except that the toner 1 used in Example 1 was changed to toners 2 to 27. The results are shown in Tables 19 to 22.

#### Comparative Examples 1 to 11

The same evaluation as that in Example 1 was conducted except that the toner 1 used in Example 1 was changed to comparative toners 1 to 11. The results are shown in Tables 23 and 24.

#### Example 28

The same evaluation as that in Example 1 was conducted except that the toner 1 used in Example 1 was changed to toner particles 1. The results are shown in Table 22.

TABLE 1

| Toner particles               |                          | Ex. 1                 | Ex. 2                 | Ex. 3                 | Ex. 4                 | Ex. 5                   | Ex. 6                 | Ex. 7                 |
|-------------------------------|--------------------------|-----------------------|-----------------------|-----------------------|-----------------------|-------------------------|-----------------------|-----------------------|
|                               |                          | Toner particles 1     | Toner particles 2     | Toner particles 3     | Toner particles 4     | Toner particles 5       | Toner particles 6     | Toner particles 7     |
| Monomer                       | Styrene                  | pbm                   | 70.0                  | 70.0                  | 70.0                  | 70.0                    | 70.0                  | 70.0                  |
|                               | n-Butyl acrylate         | pbm                   | 30.0                  | 30.0                  | 30.0                  | 30.0                    | 30.0                  | 30.0                  |
|                               | n-Butyl methacrylate     | pbm                   | 0.0                   | 0.0                   | 0.0                   | 0.0                     | 0.0                   | 0.0                   |
|                               | Benzyll acrylate         | pbm                   | 0.0                   | 0.0                   | 0.0                   | 0.0                     | 0.0                   | 0.0                   |
|                               | Acrylate                 | pbm                   | 0.0                   | 0.0                   | 0.0                   | 0.0                     | 0.0                   | 0.0                   |
|                               | Divinylbenzene           | pbm                   | 0.1                   | 0.1                   | 0.1                   | 0.1                     | 0.1                   | 0.1                   |
|                               | Silane                   | Silane 1              | Vinyltriethoxysilane  | Allyltriethoxysilane  | Vinyltrimethoxysilane | Vinyltrisopropoxysilane | Vinyltriethoxysilane  | Vinyltriethoxysilane  |
|                               | Amount of silane 1 (pbm) | 15.0                  | 15.0                  | 15.0                  | 15.0                  | 15.0                    | 15.0                  | 15.0                  |
|                               | Silane 2                 | —                     | —                     | —                     | —                     | —                       | —                     | —                     |
|                               | Amount of silane 2 (pbm) | —                     | —                     | —                     | —                     | —                       | —                     | —                     |
| Polyester-based resin         | Silane 3                 | —                     | —                     | —                     | —                     | —                       | —                     | —                     |
|                               | Amount of silane 3 (pbm) | —                     | —                     | —                     | —                     | —                       | —                     | —                     |
|                               | Type                     | (1)                   | (1)                   | (1)                   | (1)                   | (1)                     | (1)                   | (1)                   |
|                               | pbm                      | 4.0                   | 4.0                   | 4.0                   | 4.0                   | 4.0                     | 4.0                   | 4.0                   |
|                               | Type                     | Behenyl behenate      | Behenyl behenate      | Behenyl behenate      | Behenyl behenate      | Behenyl behenate        | Behenyl behenate      | Behenyl behenate      |
|                               | pbm                      | 10.0                  | 10.0                  | 10.0                  | 10.0                  | 10.0                    | 10.0                  | 10.0                  |
|                               | Melting point (°C.)      | 72.1                  | 72.1                  | 72.1                  | 72.1                  | 72.1                    | 72.1                  | 72.1                  |
|                               | Heat absorption (1/g)    | 210.3                 | 210.3                 | 210.3                 | 210.3                 | 210.3                   | 210.3                 | 210.3                 |
|                               | Colorant                 | Copper phthalocyanine | Copper phthalocyanine | Copper phthalocyanine | Copper phthalocyanine | Copper phthalocyanine   | Copper phthalocyanine | Copper phthalocyanine |
|                               | Colorant type            | 6.5                   | 6.5                   | 6.5                   | 6.5                   | 6.5                     | 6.5                   | 6.5                   |
| Release agent                 | pbm                      | 0.5                   | 0.5                   | 0.5                   | 0.5                   | 0.5                     | 0.5                   | 0.5                   |
|                               | pbm                      | 0.5                   | 0.5                   | 0.5                   | 0.5                   | 0.5                     | 0.5                   | 0.5                   |
|                               | Amount added             | —                     | —                     | —                     | —                     | —                       | —                     | —                     |
|                               | Reaction 1               | Temperature           | 70                    | 70                    | 70                    | 70                      | 70                    | 70                    |
|                               |                          | Holding time (hour)   | 5 h                   | 5 h                   | 5 h                   | 5 h                     | 5 h                   | 5 h                   |
|                               | Reaction 2               | Temperature           | 90                    | 90                    | 90                    | 90                      | 90                    | 90                    |
|                               |                          | Holding time (hour)   | 7.5 h                 | 7.5 h                 | 7.5 h                 | 7.5 h                   | 7.5 h                 | 7.5 h                 |
|                               | Reaction 3               | pH                    | 8.0                   | 8.0                   | 8.0                   | 8.0                     | 8.0                   | 8.0                   |
|                               |                          | Temperature           | 100                   | 100                   | 100                   | 100                     | 100                   | 100                   |
|                               |                          | Holding time (hour)   | 5 h                   | 5 h                   | 5 h                   | 5 h                     | 5 h                   | 5 h                   |
| Negative charge control agent | Amount added             | —                     | —                     | —                     | —                     | —                       | —                     | —                     |
|                               | Reaction 1               | Temperature           | —                     | —                     | —                     | —                       | —                     | —                     |
|                               |                          | Holding time (hour)   | —                     | —                     | —                     | —                       | —                     | —                     |
|                               | Reaction 2               | pH                    | 5.1                   | 5.1                   | 5.1                   | 5.1                     | 5.1                   | 5.1                   |
|                               |                          | Temperature           | 90                    | 90                    | 90                    | 90                      | 90                    | 90                    |
|                               |                          | Holding time (hour)   | 7.5 h                 | 7.5 h                 | 7.5 h                 | 7.5 h                   | 7.5 h                 | 7.5 h                 |
|                               | Reaction 3               | pH                    | 5.1                   | 5.1                   | 5.1                   | 5.1                     | 5.1                   | 5.1                   |
|                               |                          | Temperature           | 100                   | 100                   | 100                   | 100                     | 100                   | 100                   |
|                               |                          | Holding time (hour)   | 5 h                   | 5 h                   | 5 h                   | 5 h                     | 5 h                   | 5 h                   |
|                               |                          | pH                    | 5.1                   | 5.1                   | 5.1                   | 5.1                     | 5.1                   | 5.1                   |

In Table 1 and all tables below, pbm denotes parts by mass, Ex. denotes Example, and C. Ex. denotes Comparative Example.

TABLE 2

TABLE 3

TABLE 4

TABLE 5

TABLE 6

TABLE 7

|                     | Toner                                                                                   | Example 1<br>Toner 1 | Example 2<br>Toner 2 | Example 3<br>Toner 3 | Example 4<br>Toner 4 | Example 5<br>Toner 5 | Example 6<br>Toner 6 | Example 7<br>Toner 7 |
|---------------------|-----------------------------------------------------------------------------------------|----------------------|----------------------|----------------------|----------------------|----------------------|----------------------|----------------------|
| Physical properties | THF insoluble content (%)                                                               | 27.1                 | 29.7                 | 27.3                 | 27.2                 | 27.5                 | 42.5                 | 22.5                 |
|                     | Average circularity                                                                     | 0.982                | 0.981                | 0.982                | 0.981                | 0.981                | 0.981                | 0.980                |
|                     | Mode circularity                                                                        | 1.00                 | 1.00                 | 1.00                 | 1.00                 | 1.00                 | 1.00                 | 1.00                 |
|                     | Weight-average molecular weight                                                         | 28200                | 27800                | 27900                | 29000                | 28100                | 26100                | 28800                |
|                     | Weight-average molecular weight/Number-average molecular weight                         | 12.1                 | 12.1                 | 12.3                 | 12.1                 | 12.1                 | 12.1                 | 12.3                 |
|                     | Equivalent circle diameter determined from cross section of toner particle Dtemav. (μm) | 5.7                  | 5.7                  | 5.7                  | 5.7                  | 5.7                  | 5.7                  | 5.6                  |
|                     | Weight-average particle size (μm)                                                       | 5.6                  | 5.7                  | 5.6                  | 5.6                  | 5.6                  | 5.7                  | 5.6                  |
|                     | Number-average particle size (μm)                                                       | 5.3                  | 5.3                  | 5.3                  | 5.4                  | 5.3                  | 5.3                  | 5.3                  |
|                     | Endothermic main peak temperature (° C.)                                                | 70.4                 | 70.3                 | 70.3                 | 70.4                 | 70.3                 | 70.4                 | 70.4                 |
|                     | Integrated calorific value (J/g)                                                        | 22.3                 | 22.3                 | 22.2                 | 22.1                 | 22.3                 | 22.2                 | 22.1                 |
|                     | Glass transition temperature (° C.)                                                     | 47.6                 | 48.6                 | 49.8                 | 47.6                 | 47.8                 | 46.1                 | 48.1                 |
|                     | 80° C. viscosity (Pa · S)                                                               | 16200                | 16400                | 16300                | 16300                | 16300                | 14200                | 16800                |

TABLE 8

|                     | Toner                                                                                   | Example 8<br>Toner 8 | Example 9<br>Toner 9 | Example 10<br>Toner 10 | Example 11<br>Toner 11 | Example 12<br>Toner 12 | Example 13<br>Toner 13 | Example 14<br>Toner 14 |
|---------------------|-----------------------------------------------------------------------------------------|----------------------|----------------------|------------------------|------------------------|------------------------|------------------------|------------------------|
| Physical properties | THF insoluble content (%)                                                               | 21.2                 | 17.0                 | 16.1                   | 27.2                   | 27.6                   | 26.8                   | 19.6                   |
|                     | Average circularity                                                                     | 0.980                | 0.980                | 0.980                  | 0.981                  | 0.981                  | 0.980                  | 0.981                  |
|                     | Mode circularity                                                                        | 1.00                 | 1.00                 | 1.00                   | 1.00                   | 1.00                   | 1.00                   | 1.00                   |
|                     | Weight-average molecular weight                                                         | 28900                | 27800                | 28200                  | 27200                  | 26900                  | 27000                  | 27300                  |
|                     | Weight-average molecular weight/Number-average molecular weight                         | 12.2                 | 12.2                 | 12.3                   | 12.1                   | 12.3                   | 12.1                   | 12.1                   |
|                     | Equivalent circle diameter determined from cross section of toner particle Dtemav. (μm) | 5.7                  | 5.7                  | 5.6                    | 5.7                    | 5.6                    | 5.7                    | 5.7                    |
|                     | Weight-average particle size (μm)                                                       | 5.7                  | 5.6                  | 5.6                    | 5.6                    | 5.6                    | 5.6                    | 5.7                    |
|                     | Number-average particle size (μm)                                                       | 5.3                  | 5.3                  | 5.3                    | 5.3                    | 5.3                    | 5.3                    | 5.3                    |
|                     | Endothermic main peak temperature (° C.)                                                | 70.4                 | 70.4                 | 70.4                   | 70.4                   | 70.4                   | 70.4                   | 70.4                   |
|                     | Integrated calorific value (J/g)                                                        | 22.3                 | 22.3                 | 22.4                   | 22.3                   | 22.1                   | 22.3                   | 22.1                   |
|                     | Glass transition temperature (° C.)                                                     | 48.2                 | 48.8                 | 49.2                   | 47.9                   | 47.8                   | 47.7                   | 47.8                   |
|                     | 80° C. viscosity (Pa · S)                                                               | 16900                | 17100                | 17300                  | 16000                  | 16400                  | 16300                  | 16700                  |

TABLE 9

|                     | Toner                                                                                   | Example 15<br>Toner 15 | Example 16<br>Toner 16 | Example 17<br>Toner 17 | Example 18<br>Toner 18 | Example 19<br>Toner 19 | Example 20<br>Toner 20 |
|---------------------|-----------------------------------------------------------------------------------------|------------------------|------------------------|------------------------|------------------------|------------------------|------------------------|
| Physical properties | THF insoluble content (%)                                                               | 24.6                   | 27.8                   | 28.9                   | 29.5                   | 26.7                   | 12.6                   |
|                     | Average circularity                                                                     | 0.980                  | 0.984                  | 0.981                  | 0.974                  | 0.972                  | 0.963                  |
|                     | Mode circularity                                                                        | 1.00                   | 1.00                   | 1.00                   | 0.99                   | 0.98                   | 0.97                   |
|                     | Weight-average molecular weight                                                         | 28100                  | 24000                  | 22800                  | 17200                  | 17400                  | 56200                  |
|                     | Weight-average molecular weight/Number-average molecular weight                         | 12.3                   | 12.1                   | 12.2                   | 23.1                   | 23.2                   | 23.1                   |
|                     | Equivalent circle diameter determined from cross section of toner particle Dtemav. (μm) | 5.7                    | 5.7                    | 5.6                    | 5.6                    | 5.6                    | 5.7                    |
|                     | Weight-average particle size (μm)                                                       | 5.7                    | 5.7                    | 5.6                    | 5.6                    | 5.6                    | 5.6                    |
|                     | Number-average particle size (μm)                                                       | 5.3                    | 5.3                    | 5.3                    | 5.3                    | 5.3                    | 5.3                    |
|                     | Endothermic main peak temperature (° C.)                                                | 70.4                   | 70.3                   | 70.3                   | 70.4                   | 70.4                   | 70.4                   |
|                     | Integrated calorific value (J/g)                                                        | 22.3                   | 22.1                   | 22.4                   | 22.5                   | 22.1                   | 22.4                   |
|                     | Glass transition temperature (° C.)                                                     | 48.8                   | 46.6                   | 46.8                   | 47.8                   | 47.4                   | 47.2                   |
|                     | 80° C. viscosity (Pa · S)                                                               | 16800                  | 14300                  | 13900                  | 13200                  | 24000                  | 16400                  |

TABLE 10

|                     | Toner                                                                                         | Example 21<br>Toner 21 | Example 22<br>Toner 22 | Example 23<br>Toner 23 | Example 24<br>Toner 24 | Example 25<br>Toner 25 | Example 26<br>Toner 26 | Example 27<br>Toner 27 |
|---------------------|-----------------------------------------------------------------------------------------------|------------------------|------------------------|------------------------|------------------------|------------------------|------------------------|------------------------|
| Physical properties | THF insoluble content (%)                                                                     | 29.2                   | 27.3                   | 27.9                   | 29.6                   | 26.7                   | 20.4                   | 24.2                   |
|                     | Average circularity                                                                           | 0.980                  | 0.980                  | 0.980                  | 0.978                  | 0.980                  | 0.978                  | 0.982                  |
|                     | Mode circularity                                                                              | 0.99                   | 1.00                   | 1.00                   | 1.00                   | 1.00                   | 1.00                   | 1.00                   |
|                     | Weight-average molecular weight                                                               | 17100                  | 23400                  | 33200                  | 32400                  | 26400                  | 26000                  | 25400                  |
|                     | Weight-average molecular weight/                                                              | 23.5                   | 12.4                   | 12.6                   | 13.4                   | 11.4                   | 11.2                   | 13.4                   |
|                     | Number-average molecular weight                                                               |                        |                        |                        |                        |                        |                        |                        |
|                     | Equivalent circle diameter<br>determined from cross section of<br>toner particle Dtemav. (μm) | 5.8                    | 5.6                    | 5.6                    | 5.8                    | 5.7                    | 5.8                    | 5.8                    |
|                     | Weight-average particle size (μm)                                                             | 5.6                    | 5.6                    | 5.6                    | 5.7                    | 5.6                    | 5.7                    | 5.6                    |
|                     | Number-average particle size (μm)                                                             | 5.4                    | 5.3                    | 5.4                    | 5.4                    | 5.3                    | 5.5                    | 5.3                    |
|                     | Endothermic main peak<br>temperature (° C.)                                                   | 70.3                   | 70.3                   | 70.4                   | 70.5                   | 70.6                   | 70.2                   | 70.1                   |
|                     | Integrated calorific value (J/g)                                                              | 21.4                   | 22.5                   | 22.2                   | 22.6                   | 22.1                   | 21.4                   | 26.4                   |
|                     | Glass transition temperature (° C.)                                                           | 46.2                   | 46.7                   | 47.4                   | 48.4                   | 47.2                   | 50.2                   | 46.1                   |
|                     | 80° C. viscosity (Pa · S)                                                                     | 12900                  | 16700                  | 16300                  | 18400                  | 16000                  | 15000                  | 16500                  |

TABLE 11

|                     | Toner                                                                                         | Comparative<br>Example 1<br>toner 1 | Comparative<br>Example 2<br>toner 2 | Comparative<br>Example 3<br>toner 3 | Comparative<br>Example 4<br>toner 4 | Comparative<br>Example 5<br>toner 5 |
|---------------------|-----------------------------------------------------------------------------------------------|-------------------------------------|-------------------------------------|-------------------------------------|-------------------------------------|-------------------------------------|
| Physical properties | THF insoluble content (%)                                                                     | 12.4                                | 12.5                                | 33.2                                | 33.6                                | 32.9                                |
|                     | Average circularity                                                                           | 0.923                               | 0.982                               | 0.982                               | 0.984                               | 0.983                               |
|                     | Mode circularity                                                                              | 1.00                                | 1.00                                | 1.00                                | 1.00                                | 1.00                                |
|                     | Weight-average molecular weight                                                               | 28300                               | 28400                               | 28600                               | 28100                               | 28000                               |
|                     | Weight-average molecular weight/                                                              | 12.3                                | 12.2                                | 12.1                                | 12.0                                | 12.2                                |
|                     | Number-average molecular weight                                                               |                                     |                                     |                                     |                                     |                                     |
|                     | Equivalent circle diameter<br>determined from cross section of<br>toner particle Dtemav. (μm) | 5.7                                 | 5.7                                 | 5.7                                 | 5.7                                 | 5.7                                 |
|                     | Weight-average particle size (μm)                                                             | 5.7                                 | 5.7                                 | 5.7                                 | 5.7                                 | 5.7                                 |
|                     | Number-average particle size (μm)                                                             | 5.3                                 | 5.3                                 | 5.3                                 | 5.3                                 | 5.3                                 |
|                     | Endothermic main peak<br>temperature (° C.)                                                   | 70.4                                | 70.4                                | 70.4                                | 70.4                                | 70.4                                |
|                     | Integrated calorific value (J/g)                                                              | 22.6                                | 22.6                                | 22.5                                | 22.6                                | 22.6                                |
|                     | Glass transition temperature (° C.)                                                           | 50.2                                | 50.3                                | 48.7                                | 48.6                                | 48.3                                |
|                     | 80° C. viscosity (Pa · S)                                                                     | 17200                               | 17600                               | 17400                               | 17400                               | 17300                               |

TABLE 12

|                     | Toner                                                                                         | Comparative<br>Example 6<br>toner 6 | Comparative<br>Example 7<br>toner 7 | Comparative<br>Example 8<br>toner 8 | Comparative<br>Example 9<br>toner 9 | Comparative<br>Example 10<br>toner 10 | Comparative<br>Example 11<br>toner 11 |
|---------------------|-----------------------------------------------------------------------------------------------|-------------------------------------|-------------------------------------|-------------------------------------|-------------------------------------|---------------------------------------|---------------------------------------|
| Physical properties | THF insoluble content (%)                                                                     | 17.4                                | 15.6                                | 15.7                                | 12.4                                | 12.2                                  | 12.2                                  |
|                     | Average circularity                                                                           | 0.982                               | 0.983                               | 0.983                               | 0.981                               | 0.981                                 | 0.981                                 |
|                     | Mode circularity                                                                              | 1.00                                | 1.00                                | 1.00                                | 1.00                                | 1.00                                  | 1.00                                  |
|                     | Weight-average molecular weight                                                               | 28100                               | 28100                               | 31000                               | 26200                               | 28200                                 | 28400                                 |
|                     | Weight-average molecular weight/                                                              | 12.3                                | 12.2                                | 13.2                                | 12.2                                | 12.1                                  | 12.4                                  |
|                     | Number-average molecular weight                                                               |                                     |                                     |                                     |                                     |                                       |                                       |
|                     | Equivalent circle diameter<br>determined from cross section of<br>toner particle Dtemav. (μm) | 5.7                                 | 5.7                                 | 5.7                                 | 5.7                                 | 5.7                                   | 5.7                                   |
|                     | Weight-average particle size (μm)                                                             | 5.7                                 | 5.7                                 | 5.7                                 | 5.7                                 | 5.7                                   | 5.6                                   |
|                     | Number-average particle size (μm)                                                             | 5.3                                 | 5.3                                 | 5.4                                 | 5.3                                 | 5.4                                   | 5.3                                   |
|                     | Endothermic main peak<br>temperature (° C.)                                                   | 70.3                                | 70.3                                | 70.4                                | 70.3                                | 70.4                                  | 70.3                                  |
|                     | Integrated calorific value (J/g)                                                              | 22.6                                | 22.5                                | 22.6                                | 22.6                                | 22.7                                  | 22.3                                  |
|                     | Glass transition temperature (° C.)                                                           | 48.6                                | 48.8                                | 47.6                                | 46.1                                | 50.2                                  | 47.9                                  |
|                     | 80° C. viscosity (Pa · S)                                                                     | 16800                               | 16700                               | 16300                               | 15300                               | 16700                                 | 16400                                 |

TABLE 13

|                                                                                                               | Toner particle No. |                   |                   |                   |                               |                   |                   |
|---------------------------------------------------------------------------------------------------------------|--------------------|-------------------|-------------------|-------------------|-------------------------------|-------------------|-------------------|
|                                                                                                               | Toner particles 1  | Toner particles 2 | Toner particles 3 | Toner particles 4 | Toner particles 5             | Toner particles 6 | Toner particles 7 |
| Absence or presence of methine group bonded to silicon atom in formula (1) ( $>\text{CH}-\text{Si}$ )         | Present            | Absent            | Present           | Present           | Present                       | Present           | Present           |
| Absence or presence of methylene group bonded to silicon atom in formula (2) ( $-\text{CH}_2-\text{Si}$ )     | Absent             | Present           | Absent            | Absent            | Absent                        | Absent            | Absent            |
| R1 in formula (Z)                                                                                             | Vinyl group 2      | Allyl group 3     | Vinyl group 2     | Vinyl group 2     | Vinyl group 2                 | Vinyl group 2     | Vinyl group 2     |
| Number of carbon atoms in R1 of formula (Z)                                                                   |                    |                   |                   |                   |                               |                   |                   |
| R2, R3, and R4 in formula (Z)                                                                                 | Ethoxy group       | Ethoxy group      | Methoxy group     | Isopropoxy group  | Chloro group and ethoxy group | Ethoxy group      | Ethoxy group      |
| SQ3                                                                                                           | 0.49               | 0.44              | 0.49              | 0.48              | 0.46                          | 0.51              | 0.45              |
| SQ3/SQ2                                                                                                       | 2.33               | 2.12              | 2.32              | 2.35              | 2.32                          | 2.34              | 2.21              |
| Si concentration at toner particle surface measured by ESCA (atomic %)                                        | 17.40              | 16.40             | 17.30             | 17.10             | 16.80                         | 20.80             | 15.40             |
| Ratio of Si concentration (atomic %) to C concentration (atomic %) at toner particle surface measured by ESCA | 0.25               | 0.22              | 0.45              | 0.46              | 0.47                          | 0.49              | 0.35              |
| Average thickness of surface layer Dav. (nm)                                                                  | 15.5               | 10.8              | 55.1              | 55.0              | 54.8                          | 85.4              | 40.2              |
| Percentage of surface layer thicknesses that are 5.0 nm or less                                               | 1.6                | 18.8              | 1.6               | 1.6               | 20.3                          | 0.0               | 6.3               |
| Production method                                                                                             | First method       | First method      | First method      | First method      | First method                  | First method      | First method      |

"First method" means the first production method described in the specification.

TABLE 14

|                                                                                                               | Toner particle No. |                   |                    |                    |                    |                               |                               |                    |
|---------------------------------------------------------------------------------------------------------------|--------------------|-------------------|--------------------|--------------------|--------------------|-------------------------------|-------------------------------|--------------------|
|                                                                                                               | Toner particles 8  | Toner particles 9 | Toner particles 10 | Toner particles 11 | Toner particles 12 | Toner particles 13            | Toner particles 14            | Toner particles 15 |
| Absence or presence of methine group bonded to silicon atom in formula (1) ( $>\text{CH}-\text{Si}$ )         | Present            | Present           | Present            | Present            | Present            | Present                       | Present                       | Present            |
| Absence or presence of methylene group bonded to silicon atom in formula (2) ( $-\text{CH}_2-\text{Si}$ )     | Absent             | Absent            | Absent             | Absent             | Absent             | Absent                        | Present                       | Absent             |
| R1 in formula (Z)                                                                                             | Vinyl group        | Vinyl group       | Vinyl group        | Vinyl group        | Vinyl group        | Vinyl group and allyl group   | Vinyl and TEOS                |                    |
| Number of carbon atoms in R1 of formula (Z)                                                                   | 2                  | 2                 | 2                  | 2                  | 2                  | 2                             | 2.3                           | 2.0                |
| R2, R3, and R4 in formula (Z)                                                                                 | Ethoxy group       | Ethoxy group      | Ethoxy group       | Ethoxy group       | Ethoxy group       | Ethoxy group and ethoxy group | Ethoxy group and ethoxy group |                    |
| SQ3                                                                                                           | 0.45               | 0.45              | 0.41               | 0.41               | 0.58               | 0.55                          | 0.43                          | 0.69               |
| SQ3/SQ2                                                                                                       | 2.20               | 2.10              | 2.10               | 0.97               | 2.67               | 2.46                          | 2.05                          | 3.20               |
| Si concentration at toner particle surface measured by ESCA (atomic %)                                        | 14.40              | 10.20             | 5.70               | 15.60              | 20.20              | 19.10                         | 13.70                         | 12.40              |
| Ratio of Si concentration (atomic %) to C concentration (atomic %) at toner particle surface measured by ESCA | 0.34               | 0.17              | 0.15               | 0.24               | 0.37               | 0.32                          | 0.32                          | 0.36               |

TABLE 14-continued

|                                                                 | Toner particle No. |                   |                    |                    |                    |                    |                    |                    |
|-----------------------------------------------------------------|--------------------|-------------------|--------------------|--------------------|--------------------|--------------------|--------------------|--------------------|
|                                                                 | Toner particles 8  | Toner particles 9 | Toner particles 10 | Toner particles 11 | Toner particles 12 | Toner particles 13 | Toner particles 14 | Toner particles 15 |
| Average thickness of surface layer Dav. (nm)                    | 39.8               | 10.4              | 5.4                | 34.2               | 58.2               | 38.4               | 36.2               | 52.2               |
| Percentage of surface layer thicknesses that are 5.0 nm or less | 7.9                | 18.6              | 20.5               | 19.7               | 0.0                | 0.0                | 23.2               | 4.6                |
| Production method                                               | First method       | First method      | First method       | First method       | First method       | First method       | First method       | First method       |

"First method" means the first production method described in the specification.

TABLE 15

|                                                                                                               | Toner particle No. |                    |                    |                    |                    |                    |                    |
|---------------------------------------------------------------------------------------------------------------|--------------------|--------------------|--------------------|--------------------|--------------------|--------------------|--------------------|
|                                                                                                               | Toner particles 16 | Toner particles 17 | Toner particles 18 | Toner particles 19 | Toner particles 20 | Toner particles 21 | Toner particles 22 |
| Absence or presence of methine group bonded to silicon atom in formula (1) ( $>\text{CH}-\text{Si}$ )         | Present            | Present            | Present            | Present            | Present            | Present            | Present            |
| Absence or presence of methylene group bonded to silicon atom in formula (2) ( $-\text{CH}_2-\text{Si}$ )     | Absent             | Absent             | Absent             | Absent             | Absent             | Absent             | Absent             |
| R1 in formula (Z)                                                                                             | Vinyl group        | Vinyl group        | Vinyl group        | Vinyl group        | Vinyl group        | Vinyl group        | Vinyl group        |
| Number of carbon atoms in R1 of formula (Z)                                                                   | 2                  | 2                  | 2                  | 2                  | 2                  | 2                  | 2                  |
| R2, R3, and R4 in formula (Z)                                                                                 | Ethoxy group       | Ethoxy group       | Ethoxy group       | Ethoxy group       | Ethoxy group       | Ethoxy group       | Ethoxy group       |
| SQ3                                                                                                           | 0.62               | 0.70               | 0.48               | 0.49               | 0.43               | 0.42               | 0.44               |
| SQ3/SQ2                                                                                                       | 3.41               | 3.72               | 2.30               | 2.35               | 2.14               | 2.21               | 2.25               |
| Si concentration at toner particle surface measured by ESCA (atomic %)                                        | 18.60              | 19.80              | 17.10              | 17.40              | 16.80              | 16.10              | 16.80              |
| Ratio of Si concentration (atomic %) to C concentration (atomic %) at toner particle surface measured by ESCA | 0.22               | 0.15               | 0.34               | 0.34               | 0.34               | 0.35               | 0.36               |
| Average thickness of surface layer Dav. (nm)                                                                  | 23.2               | 14.3               | 45.4               | 51.2               | 40.1               | 41.3               | 55.0               |
| Percentage of surface layer thicknesses that are 5.0 nm or less                                               | 0.0                | 0.0                | 21.9               | 0.0                | 0.0                | 28.1               | 0.0                |
| Production method                                                                                             | First method       | First method       | Second method      | Third method       | Fourth method      | Fifth method       | First method       |

"First method" means the first production method described in the specification.

"Second method" means the second production method described in the specification.

"Third method" means the third production method described in the specification.

"Fourth method" means the fourth production method described in the specification.

"Fifth method" means the fifth production method described in the specification.

TABLE 16

|                                                                                                           | Toner particle No. |                    |                    |                    |                    |
|-----------------------------------------------------------------------------------------------------------|--------------------|--------------------|--------------------|--------------------|--------------------|
|                                                                                                           | Toner particles 23 | Toner particles 24 | Toner particles 25 | Toner particles 26 | Toner particles 27 |
| Absence or presence of methine group bonded to silicon atom in formula (1) ( $>\text{CH}-\text{Si}$ )     | Present            | Present            | Present            | Present            | Present            |
| Absence or presence of methylene group bonded to silicon atom in formula (2) ( $-\text{CH}_2-\text{Si}$ ) | Absent             | Absent             | Absent             | Absent             | Absent             |

TABLE 16-continued

|                                                                                                               | Toner particle No. |                    |                    |                    |                    |
|---------------------------------------------------------------------------------------------------------------|--------------------|--------------------|--------------------|--------------------|--------------------|
|                                                                                                               | Toner particles 23 | Toner particles 24 | Toner particles 25 | Toner particles 26 | Toner particles 27 |
| R1 in formula (Z)                                                                                             | Vinyl group        | Vinyl group        | Vinyl group        | Vinyl group        | Vinyl group        |
| Number of carbon atoms in R1 of formula (Z)                                                                   | 2                  | 2                  | 2                  | 2                  | 2                  |
| R2, R3, and R4 in formula (Z)                                                                                 | Ethoxy group       | Ethoxy group       | Ethoxy group       | Ethoxy group       | Ethoxy group       |
| SQ3                                                                                                           | 0.49               | 0.48               | 0.48               | 0.48               | 0.48               |
| SQ3/SQ2                                                                                                       | 2.33               | 2.32               | 2.33               | 2.31               | 2.34               |
| Si concentration at toner particle surface measured by ESCA (atomic %)                                        | 16.40              | 17.20              | 17.50              | 17.20              | 17.10              |
| Ratio of Si concentration (atomic %) to C concentration (atomic %) at toner particle surface measured by ESCA | 0.16               | 0.24               | 0.26               | 0.26               | 0.24               |
| Average thickness of surface layer                                                                            | 15.5               | 15.4               | 15.6               | 15.2               | 15.3               |
| Dav. (nm)                                                                                                     |                    |                    |                    |                    |                    |
| Percentage of surface layer thicknesses that are 5.0 nm or less                                               | 4.6                | 1.6                | 1.7                | 1.5                | 1.7                |
| Production method                                                                                             | First method       | First method       | First method       | First method       | First method       |

"First method" means the first production method described in the specification.

TABLE 17

|                                                                                                               | Toner particle No.            |                               |                               |                               |                               |
|---------------------------------------------------------------------------------------------------------------|-------------------------------|-------------------------------|-------------------------------|-------------------------------|-------------------------------|
|                                                                                                               | Comparative toner particles 1 | Comparative toner particles 2 | Comparative toner particles 3 | Comparative toner particles 4 | Comparative toner particles 5 |
| Absence or presence of methine group bonded to silicon atom in formula (1) ( $>\text{CH}-\text{Si}$ )         | Present                       | Absent                        | Absent                        | Absent                        | Absent                        |
| Absence or presence of methylene group bonded to silicon atom in formula (1) ( $-\text{CH}_2-\text{Si}$ )     | Absent                        | Absent                        | Absent                        | Absent                        | Absent                        |
| R1 in formula (Z)                                                                                             | Vinyl group                   | None                          | 3-Methacryloxypropyl group    | 3-Methacryloxypropyl group    | 3-Methacryloxypropyl group    |
| Number of carbon atoms in R1 of formula (Z)                                                                   | 1                             | 0                             | 6                             | 6                             | 6                             |
| R2, R3, and R4 in formula (Z)                                                                                 | Ethoxy group                  | Ethoxy group                  | Methoxy group                 | Methoxy group                 | Methoxy group                 |
| SQ3                                                                                                           | 0.38                          | 0.00                          | 0.00                          | 0.00                          | 0.00                          |
| SQ3/SQ2                                                                                                       | 2.10                          | 0.00                          | 0.00                          | 0.00                          | 0.00                          |
| Si concentration at toner particle surface measured by ESCA (atomic %)                                        | 4.90                          | 4.70                          | 8.70                          | 4.20                          | 8.20                          |
| Ratio of Si concentration (atomic %) to C concentration (atomic %) at toner particle surface measured by ESCA | 0.13                          | 0.34                          | 0.03                          | 0.02                          | 0.02                          |
| Average thickness of surface layer                                                                            | 4.5                           | 4.7                           | 3.4                           | 2.3                           | 3.5                           |
| Dav. (nm)                                                                                                     |                               |                               |                               |                               |                               |
| Percentage of surface layer thicknesses that are 5.0 nm or less                                               | 74.2                          | 50.0                          | 94.4                          | 100.0                         | 96.7                          |
| Production method                                                                                             | First method                  | First method                  | First method                  | First method                  | First method                  |

"First method" means the first production method described in the specification.

TABLE 18

|                                                                                                               | Toner particle No.            |                               |                               |                               |                                |                                |
|---------------------------------------------------------------------------------------------------------------|-------------------------------|-------------------------------|-------------------------------|-------------------------------|--------------------------------|--------------------------------|
|                                                                                                               | Comparative toner particles 6 | Comparative toner particles 7 | Comparative toner particles 8 | Comparative toner particles 9 | Comparative toner particles 10 | Comparative toner particles 11 |
| Absence or presence of methine group bonded to silicon atom in formula (1) (>CH—Si)                           | Absent                        | Present                       | Present                       | Absent                        | Absent                         | Absent                         |
| Absence or presence of methylene group bonded to silicon atom in formula (2) (—CH <sub>2</sub> —Si)           | Absent                        | Absent                        | Absent                        | Absent                        | Absent                         | Absent                         |
| R1 in formula (Z)                                                                                             | 3-Methacryloxy-propyl group   | Vinyl group                   | Vinyl group                   | Aminopropyl-trimethoxysilane  | None                           | Methyl group                   |
| Number of carbon atoms in R1 of formula (Z)                                                                   | 6                             | 2                             | 2                             | 3                             | 0                              | 0, 1                           |
| R2, R3, and R4 in formula (Z)                                                                                 | Methoxy group                 | Ethoxy group                  | Ethoxy group                  | Methoxy group                 | None                           | Ethoxy group                   |
| SQ3                                                                                                           | 0.00                          | 0.37                          | 0.21                          | 0.00                          | 0.00                           | 0.00                           |
| SQ3/SQ2                                                                                                       | 0.00                          | 2.10                          | 2.10                          | 0.00                          | 0.00                           | 0.00                           |
| Si concentration at toner particle surface measured by ESCA (atomic %)                                        | 3.80                          | 2.30                          | 2.00                          | 22.40                         | 0.00                           | 2.60                           |
| Ratio of Si concentration (atomic %) to C concentration (atomic %) at toner particle surface measured by ESCA | 0.01                          | 0.09                          | 0.08                          | 0.01                          | 0.00                           | 0.09                           |
| Average thickness of surface layer Dav. (nm)                                                                  | 2.2                           | 4.7                           | 1.3                           | 24.0                          | 0.0                            | 2.4                            |
| Percentage of surface layer thicknesses that are 5.0 nm or less                                               | 100.0                         | 96.7                          | 81.4                          | 24.0                          | 0.0                            | 96.8                           |
| Production method                                                                                             | First method                  | First method                  | First method                  | First method                  | First method                   | First method                   |

"First method" means the first production method described in the specification.

TABLE 19

|                                                    |    |                      |                                                      | Ex. 1<br>Toner 1 | Ex. 2<br>Toner 2 | Ex. 3<br>Toner 3 | Ex. 4<br>Toner 4 | Ex. 5<br>Toner 5 | Ex. 6<br>Toner 6 | Ex. 7<br>Toner 7 |
|----------------------------------------------------|----|----------------------|------------------------------------------------------|------------------|------------------|------------------|------------------|------------------|------------------|------------------|
| Environmental stability and development durability | NN | Initial              | Storage property (50° C./15 days)                    | A                | A                | A                | A                | A                | A                | A                |
|                                                    |    |                      | Long-term storage property (45° C./95% three months) | A                | A                | A                | A                | A                | A                | A                |
|                                                    |    |                      | Triboelectric charge amount (μC/g)                   | -42.5            | -42.3            | -42.1            | -41.2            | -41.1            | -42.8            | -41.8            |
|                                                    |    | After 15,000 outputs | Fogging Density                                      | 0.1 A<br>1.55 A  | 0.2 A<br>1.54 A  | 0.1 A<br>1.55 A  | 0.1 A<br>1.54 A  | 0.1 A<br>1.54 A  | 0.1 A<br>1.55 A  | 0.2 A<br>1.52 A  |
|                                                    | LL | Initial              | Soiling of parts                                     | A                | A                | A                | A                | A                | A                | A                |
|                                                    |    |                      | Triboelectric charge amount (μC/g)                   | -44.6            | -44.2            | -44.3            | -43.7            | -43.4            | -44              | -45.6            |
|                                                    |    | After 15,000 outputs | Fogging Density                                      | 0.2 A<br>1.54 A  | 0.3 A<br>1.53 A  | 0.2 A<br>1.54 A  | 0.2 A<br>1.53 A  | 0.2 A<br>1.52 A  | 0.1 A<br>1.55 A  | 0.2 A<br>1.52 A  |
|                                                    | HH | Initial              | Soiling of parts                                     | A                | A                | A                | A                | B                | A                | A                |
|                                                    |    |                      | Triboelectric charge amount (μC/g)                   | -40.6            | -40.3            | -40.1            | -39.8            | -40.1            | -41.2            | -40.4            |
|                                                    |    | After 15,000 outputs | Fogging Density                                      | 0.3 A<br>1.52 A  | 0.3 A<br>1.51 A  | 0.3 A<br>1.53 A  | 0.4 A<br>1.51 A  | 0.4 A<br>1.52 A  | 0.2 A<br>1.54 A  | 0.3 A<br>1.52 A  |
|                                                    |    |                      | Soiling of parts                                     | A                | A                | A                | A                | B                | A                | A                |

TABLE 19-continued

|                            |                                                                |                      | Ex. 1<br>Toner 1                                | Ex. 2<br>Toner 2 | Ex. 3<br>Toner 3 | Ex. 4<br>Toner 4 | Ex. 5<br>Toner 5 | Ex. 6<br>Toner 6 | Ex. 7<br>Toner 7 |        |
|----------------------------|----------------------------------------------------------------|----------------------|-------------------------------------------------|------------------|------------------|------------------|------------------|------------------|------------------|--------|
| Low-temperature fixability | SHH after being left in severe environment for 168 hours       | Initial              | Triboelectric charge amount ( $\mu\text{C/g}$ ) | -37.4            | -37.1            | -37.2            | -36.8            | -36.0            | -40.1            | -35.2  |
|                            |                                                                |                      | Fogging                                         | 0.5 A            | 0.5 A            | 0.5 A            | 0.6 A            | 0.6 A            | 0.3 A            | 0.5 A  |
|                            |                                                                |                      | Density                                         | 1.50 A           | 1.50 A           | 1.50 A           | 1.49 A           | 1.48 A           | 1.54 A           | 1.48 A |
|                            |                                                                | After 15,000 outputs | Fogging                                         | 0.6 A            | 0.6 A            | 0.6 A            | 0.7 A            | 0.7 A            | 0.4 A            | 0.6 A  |
|                            |                                                                |                      | Density                                         | 1.49 A           | 1.48 A           | 1.48 A           | 1.47 A           | 1.46 A           | 1.52 A           | 1.45 A |
|                            | Low-temperature offset end temperature ( $^{\circ}\text{C}$ .) | Soiling of parts     | A                                               | A                | A                | B                | B                | A                | A                |        |
|                            |                                                                | Initial              |                                                 | 110              | 110              | 110              | 110              | 110              | 110              | 110    |
|                            |                                                                |                      |                                                 |                  |                  |                  |                  |                  |                  |        |
|                            |                                                                |                      |                                                 |                  |                  |                  |                  |                  |                  |        |
|                            |                                                                |                      |                                                 |                  |                  |                  |                  |                  |                  |        |

TABLE 20

|                                                    |                                                          |                                                                      | Ex. 8<br>Toner 8 | Ex. 9<br>Toner 9 | Ex. 10<br>Toner 10 | Ex. 11<br>Toner 11 | Ex. 12<br>Toner 12 | Ex. 13<br>Toner 13 | Ex. 14<br>Toner 14 | Ex. 15<br>Toner 15 |
|----------------------------------------------------|----------------------------------------------------------|----------------------------------------------------------------------|------------------|------------------|--------------------|--------------------|--------------------|--------------------|--------------------|--------------------|
| Environmental stability and development durability | Storage stability                                        | Storage property ( $50^{\circ}\text{C}/15$ days)                     | A                | B                | B                  | A                  | A                  | A                  | A                  | A                  |
|                                                    |                                                          | Long-term storage property ( $45^{\circ}\text{C}/95\%$ three months) | B                | B                | C                  | B                  | A                  | A                  | A                  | A                  |
|                                                    |                                                          | Initial                                                              | -41.2            | -40.4            | -39.4              | -41.2              | -42.8              | -42.6              | -40.2              | -43.2              |
|                                                    |                                                          | Triboelectric charge amount ( $\mu\text{C/g}$ )                      |                  |                  |                    |                    |                    |                    |                    |                    |
|                                                    |                                                          | Fogging                                                              | 0.2 A            | 0.3 A            | 0.4 A              | 0.2 A              | 0.1 A              | 0.1 A              | 0.4 A              | 0.1 A              |
|                                                    | After 15,000 outputs                                     | Density                                                              | 1.52 A           | 1.52 A           | 1.52 A             | 1.52 A             | 1.55 A             | 1.54 A             | 1.51 A             | 1.55 A             |
|                                                    |                                                          | Fogging                                                              | 0.1 A            | 0.4 A            | 0.7 A              | 0.4 A              | 0.1 A              | 0.2 A              | 0.7 A              | 0.1 A              |
|                                                    |                                                          | Density                                                              | 1.50 A           | 1.48 A           | 1.46 A             | 1.48 A             | 1.54 A             | 1.52 A             | 1.46 A             | 1.53 A             |
|                                                    |                                                          | Soiling of parts                                                     | A                | A                | A                  | A                  | A                  | A                  | A                  | A                  |
|                                                    |                                                          | Initial                                                              | -46.2            | -47.2            | -48.2              | -44.8              | -43.6              | -43.2              | -43.9              | -45.3              |
|                                                    | LL                                                       | Triboelectric charge amount ( $\mu\text{C/g}$ )                      |                  |                  |                    |                    |                    |                    |                    |                    |
|                                                    |                                                          | Fogging                                                              | 0.2 A            | 0.3 A            | 0.5 A              | 0.3 A              | 0.1 A              | 0.1 A              | 0.6 A              | 0.1 A              |
|                                                    |                                                          | Density                                                              | 1.51 A           | 1.50 A           | 1.51 A             | 1.50 A             | 1.55 A             | 1.54 A             | 1.50 A             | 1.53 A             |
|                                                    |                                                          | Fogging                                                              | 0.4 A            | 0.5 A            | 0.9 A              | 0.5 A              | 0.2 A              | 0.2 A              | 0.9 A              | 0.2 A              |
|                                                    |                                                          | Density                                                              | 1.46 A           | 1.47 A           | 1.44 A             | 1.47 A             | 1.54 A             | 1.52 A             | 1.44 B             | 1.51 A             |
|                                                    | HH                                                       | Soiling of parts                                                     | A                | A                | A                  | A                  | A                  | A                  | A                  | A                  |
|                                                    |                                                          | Initial                                                              | -39.6            | -38.2            | -36.8              | -39.2              | -41.2              | -41.0              | -36.2              | -42.1              |
|                                                    |                                                          | Triboelectric charge amount ( $\mu\text{C/g}$ )                      |                  |                  |                    |                    |                    |                    |                    |                    |
|                                                    |                                                          | Fogging                                                              | 0.4 A            | 0.5 A            | 1.0 B              | 0.5 A              | 0.2 A              | 0.2 A              | 0.7 A              | 0.2 A              |
|                                                    |                                                          | Density                                                              | 1.50 A           | 1.49 A           | 1.44 B             | 1.50 A             | 1.54 A             | 1.53 A             | 1.48 A             | 1.52 A             |
|                                                    | SHH after being left in severe environment for 168 hours | Fogging                                                              | 0.6 A            | 0.8 A            | 1.2 B              | 0.7 A              | 0.3 A              | 0.3 A              | 0.9 A              | 0.3 A              |
|                                                    |                                                          | Density                                                              | 1.46 A           | 1.45 A           | 1.39 C             | 1.47 A             | 1.52 A             | 1.51 A             | 1.45 A             | 1.50 A             |
|                                                    |                                                          | Soiling of parts                                                     | A                | A                | B                  | A                  | A                  | A                  | A                  | A                  |
|                                                    |                                                          | Initial                                                              | -34.4            | -33.2            | -32.1              | -37.4              | -40.1              | -39.7              | -34.1              | -39.0              |
|                                                    |                                                          | Triboelectric charge amount ( $\mu\text{C/g}$ )                      |                  |                  |                    |                    |                    |                    |                    |                    |
|                                                    | After 15,000 outputs                                     | Fogging                                                              | 0.5 A            | 0.7 A            | 1.5 C              | 0.7 A              | 0.2 A              | 0.3 A              | 0.8 A              | 0.4 A              |
|                                                    |                                                          | Density                                                              | 1.46 A           | 1.45 A           | 1.39 C             | 1.47 A             | 1.53 A             | 1.51 A             | 1.45 A             | 1.50 A             |
|                                                    |                                                          | Fogging                                                              | 0.7 A            | 0.9 A            | 1.8 C              | 1.0 B              | 0.3 A              | 0.4 A              | 1.1 B              | 0.5 A              |
|                                                    |                                                          | Density                                                              | 1.45 A           | 1.42 B           | 1.35 C             | 1.44 C             | 1.51 A             | 1.49 A             | 1.42 B             | 1.46 A             |
|                                                    |                                                          | Soiling of parts                                                     | A                | B                | C                  | A                  | A                  | A                  | A                  | A                  |
|                                                    | Low-temperature fixability                               | Low-temperature offset end temperature ( $^{\circ}\text{C}$ )        | 110              | 110              | 110                | 110                | 125                | 110                | 110                | 110                |
|                                                    |                                                          |                                                                      |                  |                  |                    |                    |                    |                    |                    |                    |

TABLE 21

|                                                                      |  |  | Ex. 16<br>Toner 16 | Ex. 17<br>Toner 17 | Ex. 18<br>Toner 18 | Ex. 19<br>Toner 19 | Ex. 20<br>Toner 20 | Ex. 21<br>Toner 21 | Ex. 22<br>Toner 22 |
|----------------------------------------------------------------------|--|--|--------------------|--------------------|--------------------|--------------------|--------------------|--------------------|--------------------|
| Storage stability                                                    |  |  | A                  | A                  | A                  | A                  | A                  | A                  | A                  |
| Storage property ( $50^{\circ}\text{C}/15$ days)                     |  |  | A                  | A                  | A                  | A                  | A                  | A                  | A                  |
| Long-term storage property ( $45^{\circ}\text{C}/95\%$ three months) |  |  |                    |                    |                    |                    |                    |                    |                    |

TABLE 21-continued

|                                                          |                                                                |                      | Ex. 16<br>Toner 16                              | Ex. 17<br>Toner 17 | Ex. 18<br>Toner 18 | Ex. 19<br>Toner 19 | Ex. 20<br>Toner 20 | Ex. 21<br>Toner 21 | Ex. 22<br>Toner 22 |        |
|----------------------------------------------------------|----------------------------------------------------------------|----------------------|-------------------------------------------------|--------------------|--------------------|--------------------|--------------------|--------------------|--------------------|--------|
| Environmental stability and development durability       | NN                                                             | Initial              | Triboelectric charge amount ( $\mu\text{C/g}$ ) | -42.4              | -43.6              | -41.0              | -42.4              | -42.3              | -42.6              | -42.1  |
|                                                          |                                                                |                      | Fogging                                         | 0.1 A              | 0.1 A              | 0.2 A              | 0.1 A              | 0.1 A              | 0.1 A              | 0.1 A  |
|                                                          |                                                                |                      | Density                                         | 1.56 A             | 1.57 A             | 1.54 A             | 1.55 A             | 1.55 A             | 1.56 A             | 1.54 A |
|                                                          |                                                                | After 15,000 outputs | Fogging                                         | 0.2 A              | 0.1 A              | 0.2 A              | 0.2 A              | 0.2 A              | 0.2 A              | 0.1 A  |
|                                                          |                                                                |                      | Density                                         | 1.55 A             | 1.55 A             | 1.52 A             | 1.53 A             | 1.52 A             | 1.54 A             | 1.53 A |
|                                                          | LL                                                             | Initial              | Soiling of parts                                | A                  | A                  | A                  | A                  | A                  | A                  | A      |
|                                                          |                                                                |                      | Triboelectric charge amount ( $\mu\text{C/g}$ ) | -44.8              | -45.4              | -42.4              | -44.8              | -44.5              | -44.8              | -43.8  |
|                                                          |                                                                |                      | Fogging                                         | 0.1 A              | 0.1 A              | 0.3 A              | 0.2 A              | 0.2 A              | 0.1 A              | 0.2 A  |
|                                                          |                                                                |                      | Density                                         | 1.55 A             | 1.56 A             | 1.52 A             | 1.54 A             | 1.53 A             | 1.55 A             | 1.53 A |
|                                                          |                                                                | After 15,000 outputs | Fogging                                         | 0.2 A              | 0.2 A              | 0.4 A              | 0.2 A              | 0.2 A              | 0.2 A              | 0.3 A  |
|                                                          | HH                                                             | Initial              | Soiling of parts                                | A                  | A                  | A                  | A                  | A                  | A                  | A      |
|                                                          |                                                                |                      | Triboelectric charge amount ( $\mu\text{C/g}$ ) | -41.5              | -42.1              | -39.8              | -40.1              | -40.4              | -40.9              | -41.2  |
|                                                          |                                                                |                      | Fogging                                         | 0.2 A              | 0.2 A              | 0.4 A              | 0.3 A              | 0.3 A              | 0.3 A              | 0.2 A  |
|                                                          |                                                                |                      | Density                                         | 1.54 A             | 1.55 A             | 1.50 A             | 1.52 A             | 1.53 A             | 1.54 A             | 1.53 A |
|                                                          |                                                                | After 15,000 outputs | Fogging                                         | 0.4 A              | 0.3 A              | 0.5 A              | 0.4 A              | 0.4 A              | 0.4 A              | 0.4 A  |
| SHH after being left in severe environment for 168 hours | SHH after being left in severe environment for 168 hours       | Initial              | Soiling of parts                                | A                  | A                  | A                  | A                  | A                  | A                  | A      |
|                                                          |                                                                |                      | Triboelectric charge amount ( $\mu\text{C/g}$ ) | -40.8              | -41.2              | -36.1              | -37.0              | -37.8              | -38.4              | -38.2  |
|                                                          |                                                                |                      | Fogging                                         | 0.2 A              | 0.2 A              | 0.6 A              | 0.5 A              | 0.4 A              | 0.4 A              | 0.4 A  |
|                                                          |                                                                |                      | Density                                         | 1.53 A             | 1.54 A             | 1.48 A             | 1.50 A             | 1.51 A             | 1.51 A             | 1.50 A |
|                                                          |                                                                | After 15,000 outputs | Fogging                                         | 0.3 A              | 0.3 A              | 0.8 A              | 0.6 A              | 0.5 A              | 0.5 A              | 0.6 A  |
| Low-temperature fixability                               | Low-temperature offset end temperature ( $^{\circ}\text{C}$ .) |                      |                                                 | 110                | 110                | 110                | 125                | 110                | 110                | 110    |

TABLE 22

|                                                    |                            |                      | Ex. 23<br>Toner 23                                                   | Ex. 24<br>Toner 24 | Ex. 25<br>Toner 25 | Ex. 26<br>Toner 26 | Ex. 27<br>Toner 27 | Ex. 28<br>Toner particles 1 |        |
|----------------------------------------------------|----------------------------|----------------------|----------------------------------------------------------------------|--------------------|--------------------|--------------------|--------------------|-----------------------------|--------|
| Environmental stability and development durability | NN                         | Initial              | Storage property ( $50^{\circ}\text{C}/15$ days)                     | A                  | A                  | A                  | A                  | A                           |        |
|                                                    |                            |                      | Long-term storage property ( $45^{\circ}\text{C}/95\%$ three months) | A                  | A                  | A                  | A                  | A                           |        |
|                                                    |                            |                      | Triboelectric charge amount ( $\mu\text{C/g}$ )                      | -40.4              | -40.2              | -43.4              | -42.5              | -42.3                       | -39.4  |
|                                                    |                            |                      | Fogging                                                              | 0.2 A              | 0.2 A              | 0.1 A              | 0.1 A              | 0.2 A                       | 0.2 A  |
|                                                    |                            | After 15,000 outputs | Density                                                              | 1.53 A             | 1.54 A             | 1.54 A             | 1.55 A             | 1.55 A                      | 1.52 A |
|                                                    | LL                         | Initial              | Fogging                                                              | 0.4 A              | 0.3 A              | 0.1 A              | 0.2 A              | 0.3 A                       | 0.4 A  |
|                                                    |                            |                      | Density                                                              | 1.50 A             | 1.52 A             | 1.53 A             | 1.53 A             | 1.51 A                      | 1.50 A |
|                                                    |                            |                      | Soiling of parts                                                     | A                  | A                  | A                  | A                  | A                           | A      |
|                                                    |                            |                      | Triboelectric charge amount ( $\mu\text{C/g}$ )                      | -42.4              | -42.3              | -44.6              | -44.2              | -44.2                       | -40.9  |
|                                                    |                            | After 15,000 outputs | Fogging                                                              | 0.3 A              | 0.3 A              | 0.1 A              | 0.2 A              | 0.3 A                       | 0.3 A  |
| HH                                                 | HH                         | Initial              | Density                                                              | 1.52 A             | 1.52 A             | 1.54 A             | 1.54 A             | 1.53 A                      | 1.53 A |
|                                                    |                            |                      | Fogging                                                              | 0.5 A              | 0.4 A              | 0.2 A              | 0.2 A              | 0.4 A                       | 0.4 A  |
|                                                    |                            |                      | Density                                                              | 1.49 A             | 1.51 A             | 1.53 A             | 1.52 A             | 1.50 A                      | 1.51 A |
|                                                    |                            |                      | Soiling of parts                                                     | A                  | A                  | A                  | A                  | A                           | A      |
|                                                    |                            | After 15,000 outputs | Triboelectric charge amount ( $\mu\text{C/g}$ )                      | -40.1              | -37.8              | -41.4              | -40.5              | -40.3                       | -38.7  |
| Low-temperature fixability                         | Low-temperature fixability |                      | Fogging                                                              | 0.3 A              | 0.3 A              | 0.2 A              | 0.3 A              | 0.3 A                       | 0.4 A  |
|                                                    |                            |                      | Density                                                              | 1.52 A             | 1.51 A             | 1.53 A             | 1.52 A             | 1.51 A                      | 1.51 A |
|                                                    |                            |                      | Fogging                                                              | 0.4 A              | 0.4 A              | 0.3 A              | 0.3 A              | 0.4 A                       | 0.6 A  |
|                                                    |                            | Soiling of parts     | A                                                                    | A                  | A                  | A                  | A                  | A                           |        |

TABLE 22-continued

|                                                                   |                                                                |                                                       | Ex. 23<br>Toner 23 | Ex. 24<br>Toner 24 | Ex. 25<br>Toner 25 | Ex. 26<br>Toner 26 | Ex. 27<br>Toner 27 | Ex. 28<br>Toner<br>particles 1 |
|-------------------------------------------------------------------|----------------------------------------------------------------|-------------------------------------------------------|--------------------|--------------------|--------------------|--------------------|--------------------|--------------------------------|
| SHH after being<br>left in severe<br>environment<br>for 168 hours | Initial                                                        | Triboelectric<br>charge<br>amount ( $\mu\text{C/g}$ ) | -36.7              | -36.4              | -37.4              | -38.6              | -37.1              | -36.4                          |
|                                                                   |                                                                | Fogging                                               | 0.5 A              | 0.5 A              | 0.3 A              | 0.5 A              | 0.5 A              | 0.5 A                          |
|                                                                   |                                                                | Density                                               | 1.49 A             | 1.48 A             | 1.52 A             | 1.50 A             | 1.50 A             | 1.48 A                         |
|                                                                   | After 15,000<br>outputs                                        | Fogging                                               | 0.6 A              | 0.6 A              | 0.4 A              | 0.6 A              | 0.7 A              | 0.7 A                          |
|                                                                   |                                                                | Density                                               | 1.48 A             | 1.47 A             | 1.50 A             | 1.49 A             | 1.59 A             | 1.47 A                         |
|                                                                   |                                                                | Soiling of parts                                      | A                  | A                  | A                  | A                  | A                  | A                              |
| Low-temperature<br>fixability                                     | Low-temperature offset end temperature ( $^{\circ}\text{C}$ .) |                                                       | 105                | 110                | 110                | 110                | 105                | 110                            |

TABLE 23

|                                                             |                                                                   |                                                               | C. Ex. 1<br>Comparative<br>toner 1 | C. Ex. 2<br>Comparative<br>toner 2 | C. Ex. 3<br>Comparative<br>toner 3 | C. Ex. 4<br>Comparative<br>toner 5 | C. Ex. 5<br>Comparative<br>toner 5 |
|-------------------------------------------------------------|-------------------------------------------------------------------|---------------------------------------------------------------|------------------------------------|------------------------------------|------------------------------------|------------------------------------|------------------------------------|
| Storage stability                                           |                                                                   | Storage property<br>(50° C./15 days)                          | C                                  | D                                  | C                                  | C                                  | B                                  |
|                                                             |                                                                   | Long-term<br>storage property<br>(45° C./95%<br>three months) | E                                  | E                                  | D                                  | D                                  | D                                  |
| Environmental<br>stability and<br>development<br>durability | NN                                                                | Initial                                                       | -34.0                              | -40.2                              | -34.9                              | -34.0                              | -36.7                              |
|                                                             |                                                                   | Triboelectric<br>charge amount<br>( $\mu\text{C/g}$ )         |                                    |                                    |                                    |                                    |                                    |
|                                                             |                                                                   | Fogging                                                       | 0.8 A                              | 1.3 B                              | 0.8 A                              | 1.3 B                              | 0.7 A                              |
|                                                             |                                                                   | Density                                                       | 1.41 B                             | 1.37 C                             | 1.39 C                             | 1.36 C                             | 1.41 B                             |
|                                                             | After 15,000<br>outputs                                           | Fogging                                                       | 1.0 B                              | 1.4 B                              | 1.2 B                              | 1.5 C                              | 1.1 B                              |
|                                                             |                                                                   | Density                                                       | 1.37 C                             | 1.31 C                             | 1.36 C                             | 1.32 C                             | 1.38 C                             |
|                                                             | LL                                                                | Initial                                                       | -45.4                              | -46.3                              | -37.1                              | -38.6                              | -37.7                              |
|                                                             |                                                                   | Triboelectric<br>charge amount<br>( $\mu\text{C/g}$ )         |                                    |                                    |                                    |                                    |                                    |
|                                                             |                                                                   | Fogging                                                       | 1.1 B                              | 1.4 B                              | 1.0 B                              | 1.7 C                              | 0.8 A                              |
|                                                             |                                                                   | Density                                                       | 1.38 C                             | 1.36 C                             | 1.36 C                             | 1.32 C                             | 1.38 C                             |
|                                                             | After 15,000<br>outputs                                           | Fogging                                                       | 1.3 B                              | 1.6 C                              | 1.2 B                              | 1.9 C                              | 1.0 C                              |
|                                                             |                                                                   | Density                                                       | 1.36 C                             | 1.30 C                             | 1.34 C                             | 1.30 C                             | 1.34 C                             |
|                                                             | HH                                                                | Initial                                                       | -27.8                              | -26.2                              | -28.1                              | -27.1                              | -32.2                              |
|                                                             |                                                                   | Triboelectric<br>charge<br>amount ( $\mu\text{C/g}$ )         |                                    |                                    |                                    |                                    |                                    |
|                                                             |                                                                   | Fogging                                                       | 1.5 C                              | 1.9 C                              | 1.7 C                              | 1.9 C                              | 0.9 A                              |
|                                                             |                                                                   | Density                                                       | 1.32 C                             | 1.34 C                             | 1.35 C                             | 1.30 C                             | 1.36 C                             |
|                                                             | After 15,000<br>outputs                                           | Fogging                                                       | 1.7 C                              | 2.2 D                              | 1.9 C                              | 2.1 D                              | 1.1 B                              |
|                                                             |                                                                   | Density                                                       | 1.31 C                             | 1.31 C                             | 1.30 C                             | 1.27 D                             | 1.32 C                             |
|                                                             | SHH after being<br>left in severe<br>environment<br>for 168 hours | Soiling of parts                                              | B                                  | B                                  | B                                  | B                                  | B                                  |
|                                                             |                                                                   | Triboelectric<br>charge<br>amount ( $\mu\text{C/g}$ )         |                                    |                                    |                                    |                                    |                                    |
|                                                             |                                                                   | Fogging                                                       | 2.5 E                              | 2.5 E                              | 2.3 D                              | 2.5 E                              | 2.1 D                              |
|                                                             |                                                                   | Density                                                       | 1.27 D                             | 1.26 D                             | 1.27 D                             | 1.22 E                             | 1.30 C                             |
|                                                             | After 15,000<br>outputs                                           | Fogging                                                       | 2.7 E                              | 2.8 E                              | 2.5 E                              | 2.4 D                              | 2.4 D                              |
|                                                             |                                                                   | Density                                                       | 1.24 E                             | 1.22 E                             | 1.25 D                             | 1.20 E                             | 1.26 D                             |
|                                                             | Low-temperature<br>fixability                                     | Soiling of parts                                              | D                                  | D                                  | D                                  | D                                  | D                                  |
|                                                             | Low-temperature offset end temperature ( $^{\circ}\text{C}$ .)    |                                                               | 115                                | 115                                | 115                                | 115                                | 115                                |

TABLE 24

|                   |                                                               | C. Ex. 6<br>Comparative<br>toner 6 | C. Ex. 7<br>Comparative<br>toner 7 | C. Ex. 8<br>Comparative<br>toner 8 | C. Ex. 9<br>Comparative<br>toner 9 | C. Ex. 10<br>Comparative<br>toner 10 | C. Ex. 11<br>Comparative<br>toner 11 |
|-------------------|---------------------------------------------------------------|------------------------------------|------------------------------------|------------------------------------|------------------------------------|--------------------------------------|--------------------------------------|
| Storage stability | Storage property<br>(50° C./15 days)                          | C                                  | B                                  | C                                  | C                                  | F                                    | B                                    |
|                   | Long-term<br>storage property<br>(45° C./95%<br>three months) | E                                  | D                                  | E                                  | C                                  | F                                    | E                                    |

TABLE 24-continued

|                                                                   |                                                                      |                            |                                                       | C. Ex. 6<br>Comparative<br>toner 6 | C. Ex. 7<br>Comparative<br>toner 7 | C. Ex. 8<br>Comparative<br>toner 8 | C. Ex. 9<br>Comparative<br>toner 9 | C. Ex. 10<br>Comparative<br>toner 10 | C. Ex. 11<br>Comparative<br>toner 11 |
|-------------------------------------------------------------------|----------------------------------------------------------------------|----------------------------|-------------------------------------------------------|------------------------------------|------------------------------------|------------------------------------|------------------------------------|--------------------------------------|--------------------------------------|
| Environmental<br>stability and<br>development<br>durability       | NN                                                                   | Initial                    | Triboelectric<br>charge amount<br>( $\mu\text{C/g}$ ) | -37.0                              | -36.7                              | -36.6                              | -7.3                               | -28.6                                | -36.8                                |
|                                                                   |                                                                      |                            | Fogging                                               | 1.6                                | C                                  | 0.9                                | A                                  | 7.6                                  | F                                    |
|                                                                   |                                                                      | After<br>15,000<br>outputs | Density                                               | 1.37                               | C                                  | 1.50                               | A                                  | 0.78                                 | F                                    |
|                                                                   |                                                                      |                            | Fogging                                               | 1.9                                | C                                  | 1.4                                | B                                  | 7.9                                  | F                                    |
|                                                                   |                                                                      |                            | Density                                               | 1.33                               | C                                  | 1.48                               | A                                  | 0.68                                 | F                                    |
|                                                                   | LL                                                                   | Initial                    | Soiling of parts                                      | A                                  | A                                  | A                                  | C                                  | F                                    | A                                    |
|                                                                   |                                                                      |                            | Triboelectric<br>charge amount<br>( $\mu\text{C/g}$ ) | -40.2                              | -39.3                              | -37.8                              | -9.3                               | -31.4                                | -42.2                                |
|                                                                   |                                                                      |                            | Fogging                                               | 1.8                                | C                                  | 1.0                                | B                                  | 7.8                                  | F                                    |
|                                                                   |                                                                      | After<br>15,000<br>outputs | Density                                               | 1.36                               | C                                  | 1.37                               | C                                  | 0.76                                 | F                                    |
|                                                                   |                                                                      |                            | Fogging                                               | 1.5                                | C                                  | 1.1                                | B                                  | 8.1                                  | F                                    |
| SHH after being<br>left in severe<br>environment<br>for 168 hours | HH                                                                   | Initial                    | Density                                               | 1.33                               | C                                  | 1.39                               | C                                  | 0.69                                 | F                                    |
|                                                                   |                                                                      |                            | Soiling of parts                                      | B                                  | B                                  | B                                  | C                                  | F                                    | B                                    |
|                                                                   |                                                                      |                            | Triboelectric<br>charge<br>amount ( $\mu\text{C/g}$ ) | -27.9                              | -27.7                              | -30.6                              | -5.2                               | -23.5                                | -27.2                                |
|                                                                   |                                                                      |                            | Fogging                                               | 2.2                                | D                                  | 1.5                                | C                                  | 8.1                                  | F                                    |
|                                                                   |                                                                      | After<br>15,000<br>outputs | Density                                               | 1.22                               | E                                  | 1.33                               | C                                  | 0.71                                 | F                                    |
|                                                                   | SHH after being<br>left in severe<br>environment<br>for 168 hours    | Initial                    | Fogging                                               | 2.5                                | E                                  | 1.7                                | C                                  | 8.4                                  | F                                    |
|                                                                   |                                                                      |                            | Density                                               | 1.20                               | E                                  | 1.31                               | C                                  | 0.66                                 | F                                    |
|                                                                   |                                                                      |                            | Soiling of parts                                      | C                                  | A                                  | B                                  | C                                  | F                                    | B                                    |
|                                                                   |                                                                      |                            | Triboelectric<br>charge<br>amount ( $\mu\text{C/g}$ ) | -11.0                              | -17.4                              | -14.8                              | -3.9                               | -11.5                                | -17.1                                |
|                                                                   |                                                                      |                            | Fogging                                               | 2.6                                | E                                  | 2.1                                | D                                  | 9.3                                  | F                                    |
| Low-temperature<br>fixability                                     | Low-temperature<br>offset end<br>temperature ( $^{\circ}\text{C.}$ ) | Initial                    | Density                                               | 1.20                               | E                                  | 1.30                               | C                                  | 0.47                                 | F                                    |
|                                                                   |                                                                      | After<br>15,000<br>outputs | Fogging                                               | 2.9                                | E                                  | 2.2                                | D                                  | 10.6                                 | F                                    |
|                                                                   |                                                                      |                            | Density                                               | 1.15                               | F                                  | 1.27                               | D                                  | 0.45                                 | F                                    |
|                                                                   |                                                                      |                            | Soiling of parts                                      | E                                  | D                                  | D                                  | F                                  | F                                    | D                                    |

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2012-288227 filed Dec. 28, 2012, which is hereby incorporated by reference herein in its entirety.

What is claimed is:

**1. A toner comprising:**

toner particles each including a surface layer that contains an organic silicon polymer, the organic silicon polymer including a unit represented by formula (1) or (2) below:



(in formula (2), L represents a methylene group, an ethylene group, or a phenylene group),

wherein, in a chart obtained by  $^{29}\text{Si-NMR}$  measurement performed on THF insoluble components of the toner

particles, a ratio  $\text{SQ3}$  of a peak area attributable to a structure represented by formula (Q3) below to a total peak area of the organic silicon polymer satisfies mathematical formula (3) below:



(in formula (Q3),  $\text{R}_F$  represents one of structures represented by formulae (i) to (iv) below:



(in formulae (i) to (iv), \* represents a bonding portion that bonds to the silicon atom, and in formulae (ii) and (iv), L independently represents a methylene group, an ethylene group, or a phenylene group)), and

$\text{SQ3} \geq 0.40$  (3), and

wherein a silicon concentration at surfaces of the toner particles determined by electron spectroscopy for

81

chemical analysis conducted on the surfaces of the toner particles is 2.5 atomic % or more.

2. The toner according to claim 1, wherein in the chart obtained by  $^{29}\text{Si}$ -NMR measurement performed on the THF insoluble components of the toner particles, the ratio SQ3 and a ratio SQ2 of a peak area attributable to a structure represented by formula (Q2) below to the total peak area of the organic silicon polymer satisfy mathematical formula (4) below:



(in formula (Q2),  $\text{R}_G$  and  $\text{R}_H$  each independently represent at least one selected from structures represented by formulae (i) to (iv) above), and

$$(SQ3/SQ2) \geq 1.00 \quad (4).$$

3. The toner according to claim 1, wherein the organic silicon polymer is obtained by polymerizing a polymerizable monomer that contains a compound represented by formula (Z) below:

82

(Z)



(in formula (Z),  $\text{R}^1$  represents a structure represented by formula (i) or (ii) and  $\text{R}^2$ ,  $\text{R}^3$ , and  $\text{R}^4$  each independently represent a halogen atom, a hydroxy group, or an alkoxy group).

10 4. The toner according to claim 3, wherein  $\text{R}^1$  in formula (Z) represents a vinyl group or an allyl group.

15 5. The toner according to claim 3, wherein  $\text{R}^2$ ,  $\text{R}^3$ , and  $\text{R}^4$  in formula (Z) each independently represent an alkoxy group.

20 6. The toner according to claim 1, wherein the silicon concentration at surfaces of the toner particles determined by electron spectroscopy for chemical analysis conducted on the surfaces of the toner particles is 5.0 atomic % or more.

25 7. The toner according to claim 1, wherein the silicon concentration at surfaces of the toner particles determined by electron spectroscopy for chemical analysis conducted on the surfaces of the toner particles is 10.0 atomic % or more.

\* \* \* \* \*